# EUROPEAN PATENT APPLICATION

(11) **EP 4 553 134 A1**
(43) Date of publication of application: **14.05.2025**
(21) Application number: 23209229.6
(22) Date of filing: 10.11.2023
(51) Int. Cl.: C10G 2/00, C10K 3/02

(54) **CATALYSTS FOR REVERSE WATER-GAS SHIFT AND INTEGRATED FISCHER-TROPSCH PROCESSES**

(71) Applicant: BP P.L.C., London SW1Y 4PD (GB)
(72) Inventor: PATERSON, Alexander James, London, SW1Y 4PD (GB); TAYLOR, Dave, London, SW1Y 4PD (GB)
(74) Representative: Mathys & Squire

(57) **Abstract**

The present disclosure relates generally to reverse water-gas shift processes, integrated Fischer-Tropsch processes, and a supported reverse water-gas shift catalyst for conducting these processes. The catalysts described herein include a support that is a cerium oxide support, a titanium oxide support, aluminum oxide support, zinc oxide support, a zirconium oxide support, or a mixed oxide support comprising a mixture of two or more of cerium oxide, titanium oxide, aluminum oxide, zinc oxide, and zirconium oxide; a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and optionally, at least one of platinum, palladium, gold, and nickel, present in an amount in the range of 0.05 to 10 wt% of the catalyst, based on the total weight of the catalyst.

## Description

### BACKGROUND OF THE DISCLOSURE

### 1. Field

The present disclosure relates generally to reverse water-gas shift catalysts, processes of making the same, and processes for performing reverse water-gas shift reactions. The present disclosure also relates to integrating processes for performing reverse water-gas shift reactions with processes for performing Fischer-Tropsch reactions.

### 2. Technical Background

The reverse water-gas shift reaction (rWGS) is an advantageous route to obtain carbon monoxide from carbon dioxide for further chemical processing. The rWGS converts carbon dioxide and hydrogen to carbon monoxide and water, as shown in Equation (1). $Δ {{H}^{0}}_{298} = 42.1 {kJmol}^{- 1}$ This can be used, for example, to modify the CO:H₂ ratio of a gas mixture for further processing. The carbon monoxide and hydrogen so formed is a valuable feedstock for a number of chemical processes, for example, the well-known Fischer-Tropsch (FT) process, shown in Equation (2). $Δ {{H}^{0}}_{298} = - 152 {kJmol}^{- 1}$

However, the rWGS reaction is not favored in all circumstances. For example, a competing reaction is the Sabatier reaction (Equation (3)), which decreases carbon monoxide yield in favor of methane production, which is not an active feedstock for FT. $Δ {{H}^{0}}_{298} = - 165 {kJmol}^{- 1}$ The strongly exothermic Sabatier reaction is thermodynamically favored over the endothermic rWGS reaction at lower reaction temperatures. As such, minimizing the methanation during rWGS, especially at low temperatures, can become a significant challenge.

Similarly, the carbon monoxide product from rWGS can be hydrogenated to methane, as shown in Equation (4). $Δ {{H}^{0}}_{298} = - 206.5 {kJmol}^{- 1}$ Hydrogenation of carbon monoxide to methane is also an exothermic reaction, so it too is favored at lower temperatures. The stoichiometry of the reaction requires at least a 3:1 ratio of hydrogen to carbon monoxide. This means that performing the rWGS reaction with a large excess of hydrogen to drive the equilibrium toward carbon monoxide (see Equation (1)) is not always ideal because it runs the risk of hydrogenating the carbon monoxide product to form methane.

Coupled with Equations (3) and (4), further undesirable side reactions can occur. These side reactions can form undesirable carbon deposits on the surface of catalysts used to promote rWGS. Examples of these carbon-producing side reactions are shown in Equations (5), (6), and (7). All three of these reactions are endothermic and are favored at higher temperatures, just like the rWGS reaction.

CO + H₂ ↔ C + H₂O

$Δ {{H}^{0}}_{298} = 131 {kJmol}^{- 1}$

CH₄ ↔ 2H₂ + C

$Δ {{H}^{0}}_{298} = 75 {kJmol}^{- 1}$

2CO ↔ CO₂ + C

$Δ {{H}^{0}}_{298} = 171 {kJmol}^{- 1}$ Accordingly, because the carbon-producing side reactions (Equations (5)-(7)) are also endothermic and are favored at higher temperatures, operation at higher temperatures to favor the desired carbon monoxide product can severely impact catalyst lifetime through the deposition of carbon.

Given the multiple reactions and competing thermodynamics at play, there remains a need in the art for new rWGS catalysts and processes, especially for integration with Fischer-Tropsch processes.

Additionally, CO₂ is a substantial input in these reactions. Carbon dioxide is a widely available gas (currently present in the atmosphere at about 400 ppm) that is inert to many transformations. Additionally, the tendency of carbon dioxide to absorb infrared radiation has led to its designation as a greenhouse gas. Thus, there is a need to develop economical processes that utilize carbon dioxide, especially waste carbon dioxide that would otherwise be added to the ever-rising concentration of carbon dioxide in the atmosphere.

### SUMMARY

In one aspect, the present disclosure provides for a supported reverse water-gas shift catalyst comprising:
a support that is a cerium oxide support, a titanium oxide support, an aluminum oxide support, zinc oxide support, a zirconium oxide support, or a mixed oxide support comprising a mixture of two or more of cerium oxide, titanium oxide, aluminum oxide, zinc oxide and zirconium oxide;
a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
optionally, at least one of platinum, palladium, gold, and nickel present in an amount in the range of 0.05 to 10 wt% of the catalyst, based on the total weight of the catalyst.

In one aspect, the present disclosure provides for a supported reverse water-gas shift catalyst comprising:
a support that is a cerium oxide support, a titanium oxide support, an aluminum oxide support, a zinc oxide support, a zirconium oxide support, or a mixed oxide support comprising a mixture of two or more of cerium oxide, titanium oxide, aluminum oxide, zinc oxide and zirconium oxide;
a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
at least one of platinum, palladium, gold, or nickel present in an amount in the range of 0.05 to 10 wt% of the catalyst, based on the total weight of the catalyst.

In another aspect, the present disclosure provides for a method of making the catalyst as described herein, the method comprising:
providing a support that is a cerium oxide support, a titanium oxide support, an aluminum oxide support, a zinc oxide support, a zirconium support, or a mixed oxide support comprising a mixture of two or more of cerium oxide, titanium oxide, aluminum oxide, zinc oxide and zirconium oxide;
contacting the support with one or more liquids each comprising one or more metal-containing compounds dispersed in a solvent(s), wherein the metal is selected from manganese, copper, gallium, indium, lanthanum, titanium, niobium, vanadium, and zirconium, and optionally one or more platinum-, palladium-, gold-, or nickel-containing compounds;
allowing the solvent to evaporate to provide a catalyst precursor; and calcining the catalyst precursor.

In another aspect, the present disclosure provides for a catalyst as described herein made by the method as described herein.

In another aspect, the present disclosure provides a method for performing a reverse water-gas shift reaction, the method comprising contacting at a temperature in the range of 200-1100 °C a catalyst as described herein with a feed stream comprising CO₂ and H₂, wherein at least part of the CO₂ of the first feed stream is from biogas, a CO₂ emission source, and/or direct air capture, to provide a product stream comprising CO and H₂, the product stream having a lower concentration of CO₂ and a higher concentration of CO than the feed stream. For example, in some embodiments, at least a part of CO₂ of the first feed stream is from biogas. In some embodiments, at least a part of the CO₂ of the first feed stream is from a CO₂ emission source. And in some embodiments, at least a part of the CO₂ of the first feed stream is from direct air capture.

In one aspect, the present disclosure provides for a process for performing an integrated Fischer-Tropsch process, the process comprising:
providing a first feed stream comprising H₂ and CO₂, wherein at least part of the CO₂ of the first feed stream is from biogas, a CO₂ emission source and/or direct air capture;
contacting at a first temperature in the range of 200-1100 °C and at a first pressure a reverse water-gas shift catalyst with the first feed stream to perform a reverse water-gas shift reaction to provide a first product stream comprising CO and H₂, the first product stream having a lower concentration of CO₂ and a higher concentration of CO than the first feed stream;
contacting at a second temperature and at a second pressure a Fischer-Tropsch catalyst with a second feed stream comprising H₂ and at least a portion of CO of the first product stream to provide a second product stream comprising C₅+ hydrocarbons,
wherein the reverse water-gas shift catalyst is a supported reverse water-gas shift catalyst comprising:
   a support that is a cerium oxide support, a titanium oxide support, an aluminum oxide support, zinc oxide support, zirconium oxide support, or a mixed oxide support comprising a mixture of two or more of cerium oxide, titanium oxide, aluminum oxide, zinc oxide and zirconium oxide;
   a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
   optionally, at least one of platinum, palladium, gold, and nickel, present in an amount in the range of 0.05 to 10 wt% of the catalyst, based on the total weight of the catalyst.
For example, in some embodiments, at least a part of CO₂ of the first feed stream is from biogas. In some embodiments, at least a part of the CO₂ of the first feed stream is from a COz emission source. And in some embodiments, at least a part of the CO₂ of the first feed stream is from direct air capture.

### BRIEF DESCRIPTION OF FIGURES

The accompanying drawings are included to provide a further understanding of the methods of the disclosure, and are incorporated in and constitute a part of this specification. The drawings are not necessarily to scale, and sizes of various elements may be distorted for clarity. The drawings illustrate one or more embodiment(s) of the disclosure and together with the description serve to explain the principles and operation of the disclosure.
FIG. 1 is a schematic of the reverse water-gas shift reaction as described herein.
FIG. 2 is a schematic of a process for performing an integrated Fischer-Tropsch process as described herein.
FIG. 3 is a schematic of a process for performing an integrated Fischer-Tropsch process as described herein.
FIG. 4 is a schematic of a process for performing an integrated Fischer-Tropsch process as described herein.
FIG. 5 is a schematic of a process for performing an integrated Fischer-Tropsch process as described herein.
FIG. 6 is a schematic of a process for performing an integrated Fischer-Tropsch process as described herein.
FIG. 7 is a schematic of a process for performing an integrated Fischer-Tropsch process as described herein.

### DETAILED DESCRIPTION

As discussed above, the reverse gas-water shift reaction reacts carbon dioxide with hydrogen to form carbon monoxide and water and can be useful in providing a feedstock containing carbon monoxide and hydrogen -- often called "synthesis gas" -- for use in processes such as the Fischer-Tropsch process. However, the Sabatier reaction, carbon monoxide methanation, and carbon-producing side reactions can interfere with the rWGS reaction. The Sabatier reaction and CO methanation are exothermic and favored at lower temperatures, while the rWGS and carbon-producing side reactions are endothermic and favored at higher temperatures. Additionally, these reactions rely on CO₂, a greenhouse gas. To prevent further waste of CO₂ that would otherwise be added to the atmosphere, here remains a need to develop process that use CO₂. Advantageously, hydrocarbon synthesis processes that use waste carbon dioxide as a feed have the potential to be low-carbon, carbon neutral, or even have a negative carbon footprint. One way to achieve this is to transform carbon dioxide into carbon monoxide through reverse water-gas shift reactions, as described herein. Accordingly, there remains a need for rWGS catalysts that can provide good performance in spite of these complicating factors. Here, the present inventors have provided supported reverse water-gas shift catalysts that include a metal oxide support, a metal selected from at least one of manganese, gallium, indium, lanthanum, titanium, niobium, vanadium, and zirconium, and optionally, at least one of platinum, palladium, gold, and nickel. Additionally, the present inventors have found rWGS processes that are particularly advantageous for integration with a Fischer-Tropsch process by using supported reverse water-gas shift catalysts as described herein and using renewable sources of CO₂.

### Reverse Water-Gas Shift Catalysts

In one aspect, the present disclosure provides a supported reverse water-gas shift catalyst comprising: a support that is a cerium oxide support, a titanium oxide support, aluminum oxide support, a zinc oxide support, a zirconium oxide support, or a mixed oxide support comprising a mixture of two or more of cerium oxide, titanium oxide, aluminum oxide, zinc oxide and zirconium oxide; a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and optionally, at least one of platinum, palladium, gold, and nickel, present in an amount in the range of 0.05 to 10 wt% of the catalyst, based on the total weight of the catalyst. Suitable catalysts have been described in International Application No. PCT/CN2022/102723, filed June 30, 2022, International Application No. PCT/CN2022/102660, filed June 30, 2022, International Application No. PCT/CN2022/102685, filed June 30, 2022, International Application No. PCT/CN2022/102763, filed June 30, 2022, International Application No. PCT/CN2022/102976, filed June 30, 2022, International Application No. PCT/CN2022/102812, filed June 30, 2022, International Application No. PCT/CN2022/102630, filed June 30, 2022, International Application No. PCT/CN2022/102630, filed June 30, 2022, International Application No. PCT/CN2022/102799, filed June 30, 2022, International Application No. PCT/IB2023/056800, filed June 29, 2023, International Application No. PCT/IB2023/056802, filed June 29, 2023, International Application No. PCT/IB2023/056803, filed June 29, 2023, International Application No. PCT/CN2023/104014, filed June 29, 2023, and International Application No. PCT/CN2023/103835, filed June 29, 2023, each of which is hereby incorporated by reference in its entirety.

In another aspect, the present disclosure provides a supported reverse water-gas shift catalyst comprising: a support that is a cerium oxide support, a titanium oxide support, aluminum oxide support, a zinc oxide support, a zirconium oxide support, or a mixed oxide support comprising a mixture of two or more of cerium oxide, titanium oxide, aluminum oxide, zinc oxide, and zirconium oxide; a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and at least one of platinum, palladium, gold, and nickel, present in an amount in the range of 0.05 to 10 wt% of the catalyst, based on the total weight of the catalyst.

As described above, the reverse water-gas shift catalysts of the present disclosure are supported catalysts. In various embodiments as otherwise described herein, the support makes up at least 70 wt%, e.g., at least 75 wt%, or 80 wt%, or 85 wt%, or 90 wt% of the catalyst on an oxide basis.

In various embodiments as otherwise described herein, the support is a cerium oxide support. As used herein, a "cerium oxide" support is a support that presents at least a surface layer (e.g., 50 microns in thickness) that is at least 50 wt% cerium oxide, on an oxide basis. In various embodiments of the disclosure as described herein, at least a surface layer of the cerium oxide support includes at least 60 wt% cerium oxide, e.g., at least 70 wt% cerium oxide, or at least 80 wt% cerium oxide. In some such embodiments, at least a surface layer of the cerium oxide support includes at least 90 wt% cerium oxide. For example, in some embodiments, at least a surface layer of the cerium oxide support includes at least 95 wt% cerium oxide or at least 98 wt% cerium oxide. In various examples, the cerium oxide support contains cerium oxide substantially throughout, e.g., at least 50 wt% of the cerium oxide support is cerium oxide, on an oxide basis. For example, in various embodiments, the cerium oxide support includes at least 60 wt% cerium oxide, e.g., at least 70 wt% cerium oxide, or at least 80 wt% cerium oxide. In various embodiments, the cerium oxide support includes at least 90 wt% cerium oxide, e.g., at least 95 wt% cerium oxide, or at least 98 wt% cerium oxide. In some embodiments, the cerium oxide support may further include additional metals or metal oxides.

In various embodiments as otherwise described herein, the support is a titanium oxide support. As used herein, a "titanium oxide" support is a support that presents at least a surface layer (e.g., 50 microns in thickness) that is at least 50 wt% titanium oxide, on an oxide basis. In various embodiments of the disclosure as described herein, at least a surface layer of the titanium oxide support includes at least 60 wt% titanium oxide, e.g., at least 70 wt% titanium oxide, or at least 80 wt% titanium oxide. In some such embodiments, at least a surface layer of the titanium oxide support includes at least 90 wt% titanium oxide. For example, in some embodiments, at least a surface layer of the titanium oxide support includes at least 95 wt% titanium oxide or at least 98 wt% titanium oxide. In various examples, the titanium oxide support contains titanium oxide substantially throughout, e.g., at least 50 wt% of the titanium oxide support is titanium oxide, on an oxide basis. For example, in various embodiments, the titanium oxide support includes at least 60 wt% titanium oxide, e.g., at least 70 wt% titanium oxide, or at least 80 wt% titanium oxide. In various embodiments, the titanium oxide support includes at least 90 wt% titanium oxide, e.g., at least 95 wt% titanium oxide, or at least 98 wt% titanium oxide. In some embodiments, the titanium oxide support may further include additional metals or metal oxides.

In various embodiments as otherwise described herein, the support is an aluminum oxide support. As used herein, an "aluminum oxide" support is a support that presents at least a surface layer (e.g., 50 microns in thickness) that is at least 50 wt% aluminum oxide, on an oxide basis. In various embodiments of the disclosure as described herein, at least a surface layer of the aluminum oxide support includes at least 60 wt% aluminum oxide, e.g., at least 70 wt% aluminum oxide, or at least 80 wt% aluminum oxide. In some such embodiments, at least a surface layer of the aluminum oxide support includes at least 90 wt% aluminum oxide. For example, in some embodiments, at least a surface layer of the aluminum oxide support includes at least 95 wt% aluminum oxide or at least 98 wt% aluminum oxide. In various examples, the aluminum oxide support contains aluminum oxide substantially throughout, e.g., at least 50 wt% of the aluminum oxide support is aluminum oxide, on an oxide basis. For example, in various embodiments, the aluminum oxide support includes at least 60 wt% aluminum oxide, e.g., at least 70 wt% aluminum oxide, or at least 80 wt% aluminum oxide. In various embodiments, the aluminum oxide support includes at least 90 wt% aluminum oxide, e.g., at least 95 wt% aluminum oxide, or at least 98 wt% aluminum oxide. In some embodiments, the aluminum oxide support may further include additional metals or metal oxides.

In various embodiments as otherwise described herein, the support is a zinc oxide support. As used herein, a " zinc oxide" support is a support that presents at least a surface layer (e.g., 50 microns in thickness) that is at least 50 wt% zinc oxide, on an oxide basis. In various embodiments of the disclosure as described herein, at least a surface layer of the zinc oxide support includes at least 60 wt% zinc oxide, e.g., at least 70 wt% zinc oxide, or at least 80 wt% zinc oxide. In some such embodiments, at least a surface layer of the zinc oxide support includes at least 90 wt% zinc oxide. For example, in some embodiments, at least a surface layer of the zinc oxide support includes at least 95 wt% zinc oxide or at least 98 wt% zinc oxide. In various examples, the zinc oxide support contains zinc oxide substantially throughout, e.g., at least 50 wt% of the zinc oxide support is zinc oxide, on an oxide basis. For example, in various embodiments, the zinc oxide support includes at least 60 wt% zinc oxide, e.g., at least 70 wt% zinc oxide, or at least 80 wt% zinc oxide. In various embodiments, the zinc oxide support includes at least 90 wt% zinc oxide, e.g., at least 95 wt% zinc oxide, or at least 98 wt% zinc oxide. In some embodiments, the zinc oxide support may further include additional metals or metal oxides.

In various embodiments as otherwise described herein, the support is a zirconium oxide support. As used herein, a "zirconium oxide" support is a support that presents at least a surface layer (e.g., 50 microns in thickness) that is at least 50 wt% zirconium oxide, on an oxide basis. In various embodiments of the disclosure as described herein, at least a surface layer of the zirconium oxide support includes at least 60 wt% zirconium oxide, e.g., at least 70 wt% zirconium oxide, or at least 80 wt% zirconium oxide. In some such embodiments, at least a surface layer of the zirconium oxide support includes at least 90 wt% zirconium oxide. For example, in some embodiments, at least a surface layer of the zirconium oxide support includes at least 95 wt% zirconium oxide or at least 98 wt% zirconium oxide. In various examples, the zirconium oxide support contains zirconium oxide substantially throughout, e.g., at least 50 wt% of the zirconium oxide support is zirconium oxide, on an oxide basis. For example, in various embodiments, the zirconium oxide support includes at least 60 wt% zirconium oxide, e.g., at least 70 wt% zirconium oxide, or at least 80 wt% zirconium oxide. In various embodiments, the zirconium oxide support includes at least 90 wt% zirconium oxide, e.g., at least 95 wt% zirconium oxide, or at least 98 wt% zirconium oxide. In some embodiments, the zirconium oxide support may further include additional metals or metal oxides.

In various embodiments as otherwise described herein, the support is a mixed oxide support. These can be provided, for example, by admixture of multiple of the oxides above and formation into a support that includes both. For example, in some embodiments, the mixed oxide support is a mixture of two or more metal oxides, such as cerium oxide, titanium oxide, aluminum oxide, zinc oxide, and zirconium oxide. In some embodiments, at least a surface layer of the support includes at least 50 wt% total of two or more of cerium oxide, titanium oxide, aluminum oxide, zinc oxide, and zirconium oxide, on an oxide basis. In some embodiments, at least a surface layer of the mixed oxide support includes at least 60 wt% total, e.g., at least 70 wt%, or at least 80 wt% of two or more of cerium oxide, titanium oxide, aluminum oxide, zinc oxide, and zirconium oxide. In some embodiments, at least a surface layer of the mixed oxide support includes at least 90 wt%, e.g., at least 95 wt%, or at least 98 wt% of two or more cerium oxide, titanium oxide, aluminum oxide, zinc oxide, and zirconium oxide. In various examples, the mixed oxide support contains the oxides substantially throughout, e.g., at least 50 wt% of the mixed oxide support is two or more of cerium oxide, titanium oxide, aluminum oxide, zinc oxide, and zirconium oxide. In various embodiments, the mixed oxide support includes at least 60 wt% total, e.g., at least 70 wt%, or at least 80 wt% of two or more of cerium oxide, titanium oxide, aluminum oxide, zinc oxide, and zirconium oxide. In various embodiments, the mixed oxide support includes at least 90 wt% total, e.g., at least 95 wt%, or at least 98 wt% of two or more of cerium oxide, titanium oxide, aluminum oxide, zinc oxide, and zirconium oxide. In some embodiments, the mixed oxide support may further include additional metals or metal oxides.

The present inventors have found that cerium oxide, titanium oxide, aluminum oxide, zinc oxide and zirconium oxide can provide good performance in the absence of substantial amounts of other metals in the support. For example, in various embodiments of the disclosure as otherwise described herein, the support does not include additional metals in a total amount of additional metals in excess of 2 wt%, e.g., in excess of 1 wt% or in excess of 0.5 wt%, on an oxide basis.

However, the inventors have noted that in many cases performance can be desirably effected by the inclusion of other metals in the support. Accordingly, in other embodiments as otherwise described herein, the support includes at least one additional metal. In various embodiments, the total amount of the at least one additional metal is in the range of 0.5-20 wt%, e.g., 1-20 wt%, or 2-20 wt%, or 0.5-15 wt%, or 1-15 wt%, or 2-15 wt%, or 0.5-10 wt%, or 1-10 wt%, or 2-10 wt%, or 0.5-5 wt%, or 1-5 wt%, on an oxide basis.

Supports suitable for use herein can be provided with a range of pore volumes. The person of ordinary skill in the art will select a pore volume appropriate for a desired catalytic process. For example, in various embodiments as otherwise described herein, the pore volume is at least 0.05 mL/g, e.g., at least 0.1 mL/g. In various embodiments as otherwise described herein, the pore volume is at most 1.5 mL/g, e.g., at most 1 mL/g. In various embodiments of the present disclosure as described herein, the pore volume is in the range of 0.05-1.5 mL/g, e.g., 0.1 mUg to 1 mL/g. Pore volumes are measured by mercury porosimetry, for example, as measured according to ASTM D4284-12.

As described above, the supported reverse water-gas shift catalysts of the disclosure include a metal selected from at least one of manganese, copper, gallium, indium, lanthanum, titanium, niobium, vanadium, and zirconium. In some embodiments, the metal is selected from one of manganese, copper, gallium, indium, lanthanum, titanium, niobium, vanadium, and zirconium. The present inventors have determined that inclusion of the metal(s) in the catalyst can provide improved CO selectivity for the rWGS reaction, as described in the Examples below. For the purposes of this disclosure, the amount of metal present is calculated as a weight percentage of metal atoms in the catalyst based on the total weight of the catalyst, despite the form in which that metal may be present. The metal may be present in the catalyst in a variety of forms; most commonly, metal is principally present as metal oxide, metal, or a combination thereof.

In various embodiments of the present disclosure as otherwise described herein, manganese is present in the catalyst in an amount in the range of 0.5 to 20 wt%, based on total weight of the catalyst. For example, in various embodiments, manganese is present in the catalyst in an amount in the range of 0.5 to 15 wt%, or 0.5 to 12 wt%, or 0.5 to 10 wt%, based on the total weight of the catalyst. In various embodiments of the present disclosure as described herein, manganese is present in the catalyst in an amount in the range of 1 to 20 wt%, e.g., in the range of 1 to 15 wt%, or 1 to 12 wt% or 1 to 10 wt%, based on the total weight of the catalyst. In various embodiments of the present disclosure as described herein, manganese is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, manganese is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, copper is present in the catalyst in an amount in the range of 0.5 to 20 wt%, based on total weight of the catalyst. For example, in various embodiments, copper is present in the catalyst in an amount in the range of 0.5 to 15 wt%, or 0.5 to 12 wt%, or 0.5 to 10 wt%, based on the total weight of the catalyst. In various embodiments of the present disclosure as described herein, copper is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, copper is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, copper is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, gallium is present in the catalyst in an amount in the range of 0.5 to 20 wt%, based on total weight of the catalyst. For example, in various embodiments, gallium is present in the catalyst in an amount in the range of 0.5 to 15 wt%, or 0.5 to 12 wt%, or 0.5 to 10 wt%, based on the total weight of the catalyst. In various embodiments of the present disclosure as described herein, gallium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, gallium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, gallium is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, indium is present in the catalyst in an amount in the range of 0.5 to 20 wt%, based on total weight of the catalyst. For example, in various embodiments, indium is present in the catalyst in an amount in the range of 0.5 to 15 wt%, or 0.5 to 12 wt%, or 0.5 to 10 wt%, based on the total weight of the catalyst. In various embodiments of the present disclosure as described herein, indium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, indium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, indium is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, lanthanum is present in the catalyst in an amount in the range of 0.5 to 20 wt%, based on total weight of the catalyst. For example, in various embodiments, lanthanum is present in the catalyst in an amount in the range of 0.5 to 15 wt%, or 0.5 to 12 wt%, or 0.5 to 10 wt%, based on the total weight of the catalyst. In various embodiments of the present disclosure as described herein, lanthanum is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, lanthanum is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, lanthanum is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, titanium is present in the catalyst in an amount in the range of 0.5 to 20 wt%, based on total weight of the catalyst. For example, in various embodiments, titanium is present in the catalyst in an amount in the range of 0.5 to 15 wt%, or 0.5 to 12 wt%, or 0.5 to 10 wt%, based on the total weight of the catalyst. In various embodiments of the present disclosure as described herein, titanium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, titanium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, titanium is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, niobium is present in the catalyst in an amount in the range of 0.5 to 20 wt%, based on total weight of the catalyst. For example, in various embodiments, niobium is present in the catalyst in an amount in the range of 0.5 to 15 wt%, or 0.5 to 12 wt%, or 0.5 to 10 wt%, based on the total weight of the catalyst. In various embodiments of the present disclosure as described herein, niobium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, niobium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, niobium is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, vanadium is present in the catalyst in an amount in the range of 0.5 to 20 wt%, based on total weight of the catalyst. For example, in various embodiments, vanadium is present in the catalyst in an amount in the range of 0.5 to 15 wt%, or 0.5 to 12 wt%, or 0.5 to 10 wt%, based on the total weight of the catalyst. In various embodiments of the present disclosure as described herein, vanadium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, vanadium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, vanadium is present in an amount in the range of 4 to 20 wt%, e.g., in the range of 4 to 15 wt%, or 4 to 12 wt%, or 4 to 10 wt%, based on the total weight of the catalyst.

In various embodiments of the present disclosure as otherwise described herein, zirconium is present in the catalyst in an amount in the range of 0.5 to 20 wt%, based on total weight of the catalyst. For example, in various embodiments, zirconium is present in the catalyst in an amount in the range of 0.5 to 15 wt%, or 0.5 to 12 wt%, or 0.5 to 10 wt%, based on the total weight of the catalyst. In various embodiments of the present disclosure as described herein, zirconium is present in the catalyst in an amount in the range of 1 to 20 wt%, e.g., in the range of 1 to 15 wt%, or 1 to 12 wt%, or 1 to 10 wt%, based on the total weight of the catalyst. In various embodiments of the present disclosure as described herein, zirconium is present in an amount in the range of 2 to 20 wt%, e.g., in the range of 2 to 15 wt%, or 2 to 12 wt%, or 2 to 10 wt%, based on the total weight of the catalyst. In various embodiments of the present disclosure as described herein, zirconium is present in an amount in the range of 4 to 20 wt%, e.g., in the range of 4 to 15 wt%, or 4 to 12 wt%, or 4 to 10 wt%, based on the total weight of the catalyst.

As described above, the supported reverse water-gas shift catalysts of the disclosure optionally include at least one of platinum, palladium, gold, and nickel. For example, in various embodiments as otherwise described herein, platinum is present in the catalyst. For the purposes of this disclosure, the amount of platinum present is calculated as a weight percentage of platinum atoms in the catalyst based on the total weight of the catalyst, despite the form in which that platinum may be present. The platinum may be present in the catalyst in a variety of forms; most commonly, platinum is principally present as metal, metal oxide, or a combination thereof. In some embodiments of the present disclosure as described herein, platinum is present in the catalyst in an amount in the range of 0.05 to 10 wt%, e.g., in the range of 0.1 to 10 wt%, or 0.5 to 10 wt%, 1 to 10 wt%, or 2 to 10 wt%, or 5 to 10 wt%, based on the total weight of the catalyst. For example, in some embodiments, platinum is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst. In some embodiments, platinum is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst. For example, in some embodiments of the present disclosure as described herein, platinum is present in the catalyst in an amount in the range of 0.05 to 2 wt%, e.g., in the range of 0.1 to 2 wt%, or 0.3 to 2 wt%, or 0.5 to 2 wt%, based on the total weight of the catalyst. In some embodiments, platinum is present in the catalyst in an amount in the range of 0.05 to 1.5 wt%, e.g., in the range of 0.1 to 1.5 wt%, or 0.3 to 1.5 wt%, or 0.5 to 1.5 wt%, based on the total weight of the catalyst. In some embodiments, platinum is present in an amount in the range of 0.05 to 1 wt%, e.g., in the range of 0.1 to 1 wt%, or 0.3 to 1 wt%, or 0.5 to 1 wt%, based on the total weight of the catalyst. In some embodiments, platinum is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.

In various embodiments as otherwise described herein, palladium is present in the catalyst. For the purposes of this disclosure, the amount of palladium present is calculated as a weight percentage of palladium atoms in the catalyst based on the total weight of the catalyst, despite the form in which that palladium may be present. The palladium may be present in the catalyst in a variety of forms; most commonly, palladium is principally present as metal, metal oxide, or a combination thereof. In some embodiments of the present disclosure as described herein, palladium is present in the catalyst in an amount in the range of 0.05 to 10 wt%, e.g., in the range of 0.1 to 10 wt%, or 0.5 to 10 wt%, 1 to 10 wt%, or 2 to 10 wt%, or 5 to 10 wt%, based on the total weight of the catalyst. For example, in some embodiments, palladium is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst. In some embodiments, palladium is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst. For example, in some embodiments of the present disclosure as described herein, palladium is present in the catalyst in an amount in the range of 0.05 to 2 wt%, e.g., in the range of 0.1 to 2 wt%, or 0.3 to 2 wt%, or 0.5 to 2 wt%, based on the total weight of the catalyst. In some embodiments, palladium is present in the catalyst in an amount in the range of 0.05 to 1.5 wt%, e.g., in the range of 0.1 to 1.5 wt%, or 0.3 to 1.5 wt%, or 0.5 to 1.5 wt%, based on the total weight of the catalyst. In some embodiments, palladium is present in an amount in the range of 0.05 to 1 wt%, e.g., in the range of 0.1 to 1 wt%, or 0.3 to 1 wt%, or 0.5 to 1 wt%, based on the total weight of the catalyst. In some embodiments, palladium is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.

In various embodiments as otherwise described herein, gold is present in the catalyst. For the purposes of this disclosure, the amount of gold present is calculated as a weight percentage of gold atoms in the catalyst based on the total weight of the catalyst, despite the form in which that palladium may be present. The gold may be present in the catalyst in a variety of forms; most commonly, gold is principally present as metal, metal oxide, or a combination thereof. In some embodiments of the present disclosure as described herein, gold is present in the catalyst in an amount in the range of 0.05 to 10 wt%, e.g., in the range of 0.1 to 10 wt%, or 0.5 to 10 wt%, 1 to 10 wt%, or 2 to 10 wt%, or 5 to 10 wt%, based on the total weight of the catalyst. For example, in some embodiments, gold is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst. In some embodiments, gold is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst. For example, in some embodiments of the present disclosure as described herein, gold is present in the catalyst in an amount in the range of 0.05 to 2 wt%, e.g., in the range of 0.1 to 2 wt%, or 0.3 to 2 wt%, or 0.5 to 2 wt%, based on the total weight of the catalyst. In some embodiments, gold is present in the catalyst in an amount in the range of 0.05 to 1.5 wt%, e.g., in the range of 0.1 to 1.5 wt%, or 0.3 to 1.5 wt%, or 0.5 to 1.5 wt%, based on the total weight of the catalyst. In some embodiments, gold is present in an amount in the range of 0.05 to 1 wt%, e.g., in the range of 0.1 to 1 wt%, or 0.3 to 1 wt%, or 0.5 to 1 wt%, based on the total weight of the catalyst. In some embodiments, gold is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.

In various embodiments as otherwise described herein, nickel is present in the catalyst. For the purposes of this disclosure, the amount of nickel present is calculated as a weight percentage of nickel atoms in the catalyst based on the total weight of the catalyst, despite the form in which that nickel may be present. The nickel may be present in the catalyst in a variety of forms; most commonly, nickel is principally present as metal, metal oxide, or a combination thereof. In some embodiments of the present disclosure as described herein, nickel is present in the catalyst in an amount in the range of 0.05 to 10 wt%, e.g., in the range of 0.1 to 10 wt%, or 0.5 to 10 wt%, 1 to 10 wt%, or 2 to 10 wt%, or 5 to 10 wt%, based on the total weight of the catalyst. For example, in some embodiments, nickel is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst. In some embodiments, nickel is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst. For example, in some embodiments of the present disclosure as described herein, nickel is present in the catalyst in an amount in the range of 0.05 to 2 wt%, e.g., in the range of 0.1 to 2 wt%, or 0.3 to 2 wt%, or 0.5 to 2 wt%, based on the total weight of the catalyst. In some embodiments, nickel is present in the catalyst in an amount in the range of 0.05 to 1.5 wt%, e.g., in the range of 0.1 to 1.5 wt%, or 0.3 to 1.5 wt%, or 0.5 to 1.5 wt%, based on the total weight of the catalyst. In some embodiments, nickel is present in an amount in the range of 0.05 to 1 wt%, e.g., in the range of 0.1 to 1 wt%, or 0.3 to 1 wt%, or 0.5 to 1 wt%, based on the total weight of the catalyst. In some embodiments, nickel is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.

The platinum, palladium, gold, and/or nickel and the metal can be provided in a variety of weight ratios. For example, in some embodiments of the present disclosure as described herein, the weight ratio of platinum, palladium, gold, and/or nickel to metal present in the catalyst is at least 0.05:1. For example, in various embodiments, the weight ratio of platinum, palladium, gold, and/or nickel to metal is at least 0.1:1. In various embodiments of the present disclosure as described herein, the weight ratio of platinum, palladium, gold, and/or nickel to metal present in the catalyst is at most 1:1. For example, the weight ratio of platinum, palladium, gold, and/or nickel to metal is at most 0.5:1. For example, in various embodiments, the weight ratio of platinum, palladium, gold, and/or nickel to metal present in the catalyst is in the range of 0.05:1 to 1:1. For example, the weight ratio of platinum, palladium, gold, and/or nickel to metal is in the range of 0.05:1 to 0.5:1, or 0.05:1 to 0.3:1, or 0.07:1 to 1:1, or 0.07:1 to 0.5:1, or 0.07:1 to 0.3:1, or 0.1:1 to 1:1, or 0.1:1 to 0.5:1, or 0.1:1 to 0.3:1.

The present inventors have determined that suitable reverse water-gas shift catalysts can be formed of one or more of cerium oxide, titanium oxide, aluminum oxide, zinc oxide, and zirconium oxide as a support, with a metal and optionally with platinum, palladium, gold, and/or nickel included in/on the catalyst. As would be understood by the person of ordinary skill in the art, the amount of cerium, titanium, aluminum, zinc, zirconium, metal, and platinum, palladium, gold, and nickel (if present) can be quantified on a metallic basis regardless of the form in which these metals may be present. For example, the amount of these metals can be calculated as a weight percentage based on the total weight of metals in the catalysts (i.e., on a metallic basis), without the inclusion of oxygen or non-metallic counterions in the calculation. Accordingly, in various embodiments of the present disclosure as described herein, the total amount of cerium, titanium, aluminum, zinc, zirconium, and metal in the catalyst is at least 90 wt%, e.g., at least 95 wt%, or at least 98 wt% of the catalyst, on a metallic basis. For example, in some particular embodiments, the total amount of cerium and metal in the catalyst is at least 90 wt%, e.g., at least 95 wt%, or at least 98 wt% of the catalyst, on a metallic basis. In other embodiments, the total amount of titanium and metal in the catalyst is at least 90 wt%, e.g., at least 95 wt%, or at least 98 wt% of the catalyst, on a metallic basis. In other embodiments, the total amount of aluminum and metal in the catalyst is at least 90 wt%, e.g., at least 95 wt%, or at least 98 wt% of the catalyst, on a metallic basis. In other embodiments, the total amount of zinc and metal in the catalyst is at least 90 wt%, e.g., at least 95 wt%, or at least 98 wt% of the catalyst, on a metallic basis. In other embodiments, the total amount of zirconium and metal in the catalyst is at least 90 wt%, e.g., at least 95 wt%, or at least 98 wt% of the catalyst, on a metallic basis. In various embodiments of the present disclosure as described herein, the total amount of cerium, titanium, aluminum, zinc, zirconium, metal, platinum, palladium, gold, and nickel in the catalyst is at least 90 wt%, e.g., at least 95 wt%, or at least 98 wt% of the catalyst, on a metallic basis. For example, in some particular embodiments, the total amount of cerium, metal, platinum, palladium, gold, and nickel in the catalyst is at least 90 wt%, e.g., at least 95 wt%, or at least 98 wt% of the catalyst, on a metallic basis. In other embodiments, the total amount of titanium, metal, platinum, palladium, gold, and nickel in the catalyst is at least 90 wt%, e.g., at least 95 wt%, or at least 98 wt% of the catalyst, on a metallic basis. In other embodiments, the total amount of aluminum, metal, platinum, palladium, gold, and nickel in the catalyst is at least 90 wt%, e.g., at least 95 wt%, or at least 98 wt% of the catalyst, on a metallic basis. In other embodiments, the total amount of zinc, metal, platinum, palladium, gold, and nickel in the catalyst is at least 90 wt%, e.g., at least 95 wt%, or at least 98 wt% of the catalyst, on a metallic basis. In other embodiments, the total amount of zirconium, metal, platinum, palladium, gold, and nickel in the catalyst is at least 90 wt%, e.g., at least 95 wt%, or at least 98 wt% of the catalyst, on a metallic basis.

As described above, the supported catalyst includes metals and optionally at least one of platinum, palladium, gold, and nickel. Depending on the process of synthesis, these species, which will typically be principally present in metallic form and/or oxide form, can be disposed at a variety of different places on the support. For example, they can be found in pores of the support and on the outer surface of the support. They may be found substantially throughout the support, e.g., as when a large volume of impregnation liquid is used, or only in a surface layer of the support, e.g., when impregnation liquid does not infiltrate into the entirety of the support, such as when using an incipient wetness technique.

Without intending to be bound by theory, it is believed that the active form of platinum and palladium is typically a substantially metallic form. As described below, as platinum and palladium may be present substantially in an oxide form after catalyst preparation and during shipment and storage, it is typically desirable to activate the catalyst by contacting it with a reductant, e.g., hydrogen gas, to convert a substantial fraction of such oxide to metallic form. However, the person of ordinary skill in the art will appreciate that the present disclosure contemplates the usefulness of a wide variety of palladium and platinum forms in its catalysts, as these can be active or can be conveniently transformed to active forms.

The metal will typically be provided in oxide form after catalyst preparation and during shipment and storage. Without intending to be bound by theory, the present inventors believe that the metal acts to improve the catalytic activity of the supported platinum, palladium, gold, and/or nickel catalysts by reducing CO methanation that can occur over the typical reverse water-gas shift reaction temperature range, which impacts CO selectivity. The present inventors believe that the improved activity can be attributed to the metal interfacing with the support (e.g., cerium oxide, titanium oxide, aluminum oxide, zinc oxide, zirconium oxide, or a mixed oxide). Additionally, when platinum, palladium, gold, and nickel are present in the catalyst, the present inventors believe that the improved activity can be attributed to the metal interfacing with both the noble metals and the support. The present inventors contemplate that it is possible that some metal oxide is converted to metallic form during the activation of the platinum, palladium, gold, and/or nickel species. However, the person of ordinary skill in the art will appreciate that the present disclosure contemplates the usefulness of a wide variety of metal forms in its catalysts, as these can provide a promoting effect or can be conveniently transformed to forms that will.

The person of ordinary skill in the art will appreciate that the catalysts of the disclosure can be provided in many forms, depending especially on the particular form of the reactor system in which they are to be used, e.g., in a fixed bed or as a fluid bed. The supports themselves can be provided as discrete bodies of material, e.g., as porous particles, pellets or shaped extrudates, with metal and optionally, palladium, platinum, gold, and/or nickel provided thereon to provide the catalyst. However, in other embodiments, a catalyst of the disclosure can itself be formed as a layer on an underlying substrate. The underlying substrate is not particularly limited. It can be formed of, e.g., a metal or metal oxide, and can itself be provided in a number of forms, such as particles, pellets, shaped extrudates, or monoliths. The person of ordinary skill in the art can, e.g., use coating or other forming techniques to provide a layer of support on the substrate, then add metal and optionally, platinum, palladium, gold, and/or nickel. Of course, as would be understood by the person of ordinary skill in the art, other embodiments may be possible.

Another aspect of the present disclosure provides for a method of making the catalyst as described herein. As described above, the method includes providing a support that is a cerium oxide support, a titanium oxide support, an aluminum oxide support, a zinc oxide support, a zirconium oxide support, or a mixed oxide support including a mixture of two or more of cerium oxide, titanium oxide, aluminum oxide, zinc oxide, and zirconium oxide; contacting the support with one or more liquids each comprising one or more metal-containing compounds dispersed in a solvent(s), wherein the metal is selected from manganese, copper, gallium, indium, lanthanum, titanium, niobium, vanadium, and zirconium, and optionally one or more platinum-, palladium-, gold-, or nickel-containing compounds; allowing the solvent(s) to evaporate to provide a catalyst precursor; and calcining the catalyst precursor. The person of ordinary skill in the art will appreciate, of course, that other methods can be used to make the catalysts described herein.

In some embodiments of the present disclosure as described herein, contacting the support with the liquid includes adding the liquid in an amount about equal to (i.e., within 25% of, or within 10% of) the pore volume of the support. In other embodiments, contacting the support with the liquid includes adding the liquid in an amount greater than the pore volume of the support. For example, in some embodiments, the ratio of the amount of liquid to the amount of support on a mass basis is in the range of 0.75:1 to 5:1, e.g., in the range of 0.9:1 to 3:1. In some embodiments, contacting the support with the liquid provides a slurry.

In various embodiments of the present disclosure as described herein, allowing the solvent to evaporate is conducted at ambient temperature. In various embodiments, allowing the solvent to evaporate is conducted at an elevated temperature for a drying time. The person of ordinary skill in the art would be able to select appropriate apparatuses or instruments to allow the solvent to evaporate, and such apparatuses or instruments are not particularly limited. Additionally, the person of ordinary skill in the art would understand that the elevated temperature that will allow the solvent to evaporate depends on the boiling point of the solvent. As such, the person of ordinary skill in the art would be able to select an appropriate elevated temperature. For example, in some embodiments, the elevated temperature is in the range of 50-150 °C, e.g., in the range of 50-120 °C, or 50-100 °C, or 100-150 °C, or 100-120 °C. In some embodiments, the drying time is in the range of 1 to 48 hours, e.g., in the range of 10 to 36 hours, or 12 to 24 hours. For example, in particular embodiments, the drying time is about 24 hours. In some embodiments, allowing the solvent to evaporate is conducted under vacuum and at an elevated temperature for a drying time, as described herein. In some embodiments, allowing the solvent to evaporate is conducted in a stirring drybath at an elevated temperature, for example, in the range of 30-100 °C.

In some embodiments of the present disclosure as described herein, calcining the catalyst precursor is conducted in a furnace for a calcining time and at a calcining temperature. For example, in some embodiments, the calcining time is in the range of 0.5 to 24 hours, or 0.5 to 15 hours, or 0.5 to 10 hours, or 0.5 to 5 hours. In some embodiments, the calcining temperature is in the range of 100-600 °C, e.g., in the range of 120-500 °C.

As described above, the method of making the catalyst as described herein includes contacting the support with one or more liquids each including one or more metal-containing compounds and optionally, one or more platinum-, palladium-, gold-, or nickel-containing compounds dispersed in a solvent. The platinum-, palladium-, gold-, and metal-containing compounds are not particularly limited and the person of ordinary skill in the art would be able to choose appropriate compounds that are soluble in the solvent. For example, in some embodiments of the disclosure as described herein, the platinum-, palladium-, gold-, and metal-containing compounds may be selected from metal salts (e.g., nitrates and acetates). The solvent is also not particularly limited and the person of ordinary skill in the art would be able to choose an appropriate solvent that can be absorbed by the support. For example, in some embodiments of the disclosure as described herein, the solvent is water. As the person of ordinary skill in the art will appreciate, these metal species are conveniently provided in the same liquid, so that only one step of contacting the support with liquid is required. However, other schemes are possible.

In another aspect, the present disclosure provides a catalyst as described herein made by the methods as described herein.

### Reverse Water-Gas Shift Reaction

Another aspect of the present disclosure provides a method for performing a reverse water-gas shift reaction. As described above, the method includes contacting at a temperature in the range of 250-1100 °C a catalyst as described herein with a feed stream that includes CO₂ and H₂, wherein at least part of the CO₂ of the first feed stream is from biogas, a CO₂ emission source, and/or direct air capture, to provide a product stream that includes CO and H₂, the product stream having a lower concentration of CO₂ and a higher concentration of CO than the feed stream. An example of such a method is shown schematically in FIG. 1. In FIG. 1, the method 100 includes performing a reverse water-gas shift reaction by providing a feed stream 111 comprising H₂ and CO₂, here, to a reaction zone, e.g., a reactor 110. A reverse water-gas shift catalyst 113, as described herein, is contacted at a temperature in the range of 250-1100 °C with the feed stream 111 to provide a product stream 112 comprising CO and H₂. The product stream has a lower concentration of CO₂ and a higher concentration of CO than the feed stream.

As used herein, a "feed stream" is used to mean the total material input to a process step, regardless of whether provided in a single physical stream or multiple physical streams, and whether through a single inlet or multiple inlets. For example, H₂ and CO of the feed stream can be provided to the reverse water-gas shift catalyst in a single physical stream (e.g., in a single pipe to reactor 110), or in multiple physical streams (e.g., separate inlets for CO and H₂, or one inlet for fresh CO and H2 and another for recycled CO and/or H2). Similarly, a "product stream" is used to mean the total material output from a process step, regardless of whether provided in a single physical stream or multiple physical streams, and whether through a single outlet or multiple outlets.

As described above, CO₂ is a substantial input to the claimed processes. Advantageously, the present inventors have recognized that at least part of the CO₂ of the first feed stream (e.g., at least 50%, at least 75%, at least 90% or at least 95%) can come from renewable or otherwise environmentally responsible sources. Accordingly, as described above, at least part of the CO₂ of the first feed stream is from biogas, a CO₂ emission source, and/or direct air capture.

In various embodiments, at least a portion of the CO₂ of the first feed stream is from biogas. Biogas is produced by anaerobic digestion of organic matter (e.g., animal water, food waste, plant matter) by microorganisms and includes substantial amounts of CO₂ and methane. In some embodiments as described herein, a majority (i.e., at least 50 mol%) the CO₂ of the first feed stream is from biogas. In some embodiments as described herein, substantially all (e.g., at least 90 mol%) of the CO₂ of the first feed stream is from biogas. For example, in some embodiments, the CO₂ of the first feed stream comprises at least 50 mol% (e.g., at least 75 mol%, at least 90 mol%, or at least 95 mol%) CO₂ from biogas. In various embodiments, such as when at least part of the CO₂ of the first feed stream is from biogas, the process as described herein may operate with significant amounts of unreacted methane. For example, in various embodiments wherein the first feed stream comprises methane, such as from biogas, the first feed stream comprises methane in an amount in the range of 10-70 mol%, or 10-50 mol%, or 20-70 mol%, or 20-50 mol%, or 30-70 mol%, or 30-50 mol%.. In other embodiments as described herein, when the first feed stream comprises biogas, the methane in the biogas may be separated out before being added to the first feed stream. Accordingly, in some embodiments, the process as described herein may operate with low amounts of unreacted methane. For example, in certain embodiments as otherwise described herein, the first feed stream comprises methane in an amount in the range of 0.1 to 10 mol%, or 0.1 to 5 mol%, or 0.1 to 1 mol%.

In various embodiments, at least a portion of the CO₂ of the first feed stream is from direct air capture. Carbon dioxide is a common waste material, and often desirable to be removed from waste streams rather than be vented to the atmosphere. Such capture of carbon dioxide is critical to the implementation of many renewable initiatives as it serves to lower the carbon footprint of the associated process. Advantageously, the carbon dioxide utilized in the processes described herein may be carbon dioxide collected from the atmosphere or that would otherwise have been released into the atmosphere, e.g., from a combustion or other industrial process. The carbon dioxide may be captured, where it is collected or absorbed after release from an industrial process, or harvested directly from the atmosphere. By using captured carbon dioxide, the eventual hydrocarbon product can be substantially carbon-neutral or of lower carbon intensity. Methods of carbon dioxide capture are known to those of skill in the art. In various embodiments, at least a portion of the CO₂ of the first feed stream is from direct air capture. In some embodiments as described herein, a majority (i.e., at least 50 mol%) the CO₂ of the first feed stream is from direct air capture. In some embodiments as described herein, substantially all (e.g., at least 90 mol%) of the CO₂ of the first feed stream is from direct air capture. For example, in some embodiments, the CO₂ of the first feed stream comprises at least 50 mol% (e.g., at least 75 mol%, at least 90 mol%, or at least 95 mol%) CO₂ from direct air capture.

In various embodiments as described herein, at least part of the CO₂ of the first feed stream is from a CO₂ emission source. Additionally or alternatively, carbon dioxide is often scrubbed from industrial effluent, especially processes that generate large amounts of carbon dioxide as a byproduct. As used herein, the source of this carbon dioxide byproduct from industrial processes is referred to as a CO₂ emission source. In some embodiments as described herein, a majority (i.e., at least50 mol%) the CO₂ of the first feed stream is from a CO₂ emission source. In some embodiments as described herein, substantially all (e.g., at least 90 mol%) of the CO₂ of the first feed stream is from a CO₂ emission source. For example, in some embodiments, the CO₂ of the first feed stream comprises at least 50 mol% (e.g., at least 75 mol%, at least 90 mol%, or at least 95 mol%) CO₂ from a CO₂ emission source. The CO₂ emission source is not particularly limited and may derived from any industrial production known in the art. For example, in some embodiments as described herein, the CO₂ emission source is a manufacturing plant, a bioethanol plant, a CO₂ producing fermentation plant, a steel plant, or a cement plant. Accordingly, in various embodiments as otherwise described herein, at least part of the CO₂ of the first feed stream (e.g., at least 50%, at least 75%, at least 90% or at least 95%) is captured from a manufacturing plant, e.g., a bioethanol plant (e.g., CO₂ produced fermentation), a steel plant or a cement plant. In some embodiments as described herein, the CO₂ emission source is a point source from a fermentation, manufacturing, or other industrial process. The point source may be in the form of a chimney or vent or other structure for containing and/or transporting CO₂ known in the art.

Accordingly, the rWGS-Fischer Tropsch integrated processes of the disclosure as described herein can be not only carbon neutral, but in some cases a net consumer of carbon dioxide. These benefits in particular make the integrated processes highly attractive for decarbonizing transportation fuels, for both automotive and aviation sectors, since the carbon monoxide produced in the rWGS reaction can be readily utilized by well-established technologies to synthesize liquid hydrocarbon fuels by Fischer-Tropsch processes.

For example, in various embodiments of the present disclosure as described herein, the reverse water-gas shift reaction has a CO selectivity of at least 50%, e.g., at least 50%. In various embodiments, the reverse water-gas shift reaction has a CO selectivity of at least 70%, e.g., of at least 80%. In various embodiments, the reverse water-gas shift reaction has a CO selectivity of at least 85%, e.g., or at least 90%. In various embodiments, the reverse water-gas shift reaction has a CO selectivity of at least 95%, e.g., or at least 96%. As used herein, a "selectivity" for a given reaction product is the molar fraction of the converted feed (here, the CO₂ that is converted to products other than CO₂) that is converted to the identified product (for "CO selectivity," CO). The present inventors have determined that the present catalysts, even when operating at lower temperatures (e.g., less than 900 °C) than many conventional reverse water-gas shift catalysts, can provide excellent selectivity for CO, despite the potential for competition by the Sabatier reaction and the methanation of CO. For example, in various embodiments of the present disclosure as described herein, the reverse water-gas shift reaction has a CO selectivity in the range of 50-99 wt%, e.g., 60-99%, or 70-99%, or 80-99%, or 90-99%, or 95-99%. In various embodiments, the reverse water-gas shift reaction has a CO selectivity in the range of 50-90%, e.g., 60-90%, or 70-90%, or 50-80%, or 60-80%, or 50-70%.

Notably, even over a broad range of temperatures in the range of 200-1100 °C, the catalysts described herein can be operated to provide carbon monoxide with only a very minor degree of methane formation. For example, in various embodiments of the present disclosure as described herein, the reverse water-gas shift reaction has a methane selectivity of no more than 40%, e.g., no more than 35%, or 30%, or 25%, or 20%. For example, in various embodiments of the present disclosure as described herein, the reverse water-gas shift reaction has a methane selectivity of no more than 15%, e.g., no more than 12%, or 10%, or 8%. For example, in various embodiments of the present disclosure as otherwise described herein, the reverse water-gas shift reaction has a methane selectivity of no more than 5%, e.g., no more than 4%. For example, in some embodiments, the reverse water-gas shift reaction has a methane selectivity of no more than 2%, e.g., no more than 1%. In some embodiments, the reverse water-gas shift reaction has a methane selectivity of no more than 0.5%, e.g., no more than 0.2%.

The present inventors have determined that the catalysts described here can provide desirably high CO selectivity and desirably low methane selectivity at commercially relevant conversion rates. As used herein, a "conversion" is a molar fraction of a feed that is reacted (be it to desirable products or undesirable species). In various embodiments of the present disclosure as described herein, the reverse water-gas shift reaction has a CO₂ conversion of at least 5%, e.g., at least 10%, or 20%. For example, in some embodiments, the reverse water-gas shift reaction has a CO₂ conversion of at least 30%, e.g., at least 40%, or 50%, or 60%. In various embodiments of the present disclosure as described herein, the reverse water-gas shift reaction has a CO₂ conversion of no more than 90%, e.g., no more than 80%, or no more than 70%. For example, in some embodiments, the reverse water-gas shift reaction has a CO₂ conversion of no more than 65%, e.g., no more than 60%. For example, in various embodiments as otherwise described herein, the CO₂ conversion is in the range of 10-90%, e.g., 10-80%, 10-70%, or 10-60%, or 10-65%, or 20-90%, or 20-80%, or 20-70%, or 20-60%, or 20-65%, or 30-90%, or 30-80%, or 30-70%, or 30-60%, or 30-65%, or 40-90%, or 40-80%, or 40-70%, or 40-60%, or 40-65%. The person of ordinary skill in the art will, based on the disclosure herein, operate at a degree of conversion that provides a desirable product. And of course, in other embodiments, e.g., when in a stacked-bed or mixed-bed system, the CO₂ conversion may be even higher than described here.

Advantageously, the processes described herein can be performed at temperatures that are lower than temperatures used in many conventional reverse water-gas shift processes. As described above, various processes of the disclosure can be performed in a temperature range of 200-1100°C, e.g., in the range of 200-1050 °C, or 200-1000 °C, or 200-950 °C, or 250-1050 °C, or 250-1000 °C, or 250-950 °C. For example, in some embodiments, the method for performing the reverse water-gas shift reaction is conducted at a temperature in the range of 250-900 °C, e.g., in the range of 250-850 °C, 250-800 °C, or 250-750 °C, or 250-700 °C, or 250-650 °C, or 250-600 °C. In some embodiments as described herein, the method for performing the reverse water-gas shift reaction is conducted at a temperature in the range of 300-1100 °C, e.g., in the range of 300-1050 °C, or 300-1000 °C, or 300-950 °C. In some embodiments of the present disclosure as described herein, the method for performing the reverse water-gas shift reaction is conducted at a temperature in the range of 300-900 °C, e.g., in the range of 300-850 °C, or 300-800 °C, or 300-750 °C, or 300-700 °C, or 300-650 °C, or 300-600 °C. In some embodiments as described herein, the method for performing the reverse water-gas shift reaction is conducted at a temperature in the range of 350-1100 °C, e.g., in the range of 350-1050 °C, or 350-1000 °C , or 350-950 °C. In some embodiments of the present disclosure as described herein, the method for performing the reverse water-gas shift reaction is conducted at a temperature in the range of 350-900 °C, e.g., in the range of 350-850 °C , or 350-800 °C , or 350-750 °C, or 350-700 °C, or 350-650 °C, or 350-600 °C. In some embodiments as described herein, the method for performing the reverse water-gas shift reaction is conducted at a temperature in the range of 400-1100 °C, e.g., in the range of 400-1050 °C, or 400-1000 °C , or 400-950 °C. In some embodiments, the method for performing the reverse water-gas shift reaction is conducted at a temperature in the range of 400-900 °C, e.g., in the range of 400-850 °C, or 400-800 °C , or 400-750 °C, or 400-700 °C, or 400-650 °C, or 400-600 °C. In some embodiments as described herein, the method for performing the reverse water-gas shift reaction is conducted at a temperature in the range of 450-1100 °C, e.g., in the range of 450-1050 °C, or 450-1000 °C, or 450-950 °C. In some embodiments, the method for performing the reverse water-gas shift reaction is conducted at a temperature in the range of 450-900 °C, e.g., in the range of 450-850 °C , or 450-800 °C, or 450-750 °C, or 450-700 °C, or 450-650 °C, or 450-600 °C. In some embodiments as described herein, the method for performing the reverse water-gas shift reaction is conducted at a temperature in the range of 500-1100 °C, e.g., in the range of 500-1050 °C, or 500-1000 °C, or 500-950 °C. In some embodiments, the method for performing the reverse water-gas shift reaction is conducted at a temperature in the range of 500-900 °C, e.g., in the range of 500-850 °C, or 500-800 °C, or 500-750 °C , or 500-700 °C, or 500-650 °C, or 500-600 °C. In some embodiments as described herein, the method for performing the reverse water-gas shift reaction is conducted at a temperature in the range of 550-1100 °C, e.g., in the range of 550-1050 °C, or 550-1000 °C, or 550-950 °C. In some embodiments, the method for performing the reverse water-gas shift reaction is conducted at a temperature in the range of 550-900 °C, e.g., in the range of 550-850 °C, or 550-800 °C, or 550-750°C, or 550-700 °C, or 550-650 °C, or 550-600 °C. In some embodiments as described herein, the method for performing the reverse water-gas shift reaction is conducted at a temperature in the range of 600-1100 °C, e.g., in the range of 600-1050 °C, or 600-1000 °C, or 600-950 °C. In some embodiments, the method for performing the reverse water-gas shift reaction is conducted at a temperature in the range of 600-900 °C, e.g., in the range of 600-850 °C, or 600-800 °C, or 600-750°C, or 600-700 °C, or 600-650 °C. In some embodiments as described herein, the method for performing the reverse water-gas shift reaction is conducted at a temperature in the range of 650-1100 °C, e.g., in the range of 650-1050 °C, or 650-1000 °C, or 650-950 °C. In some embodiments, the method for performing the reverse water-gas shift reaction is conducted at a temperature in the range of 650-900 °C, e.g., in the range of 650-850 °C, or 650-800 °C, or 650-750°C, or 650-700 °C. In some embodiments as described herein, the method for performing the reverse water-gas shift reaction is conducted at a temperature in the range of 700-1100 °C, e.g., in the range of 700-1050 °C, or 700-1000 °C, or 700-950 °C. In some embodiments, the method for performing the reverse water-gas shift reaction is conducted at a temperature in the range of 700-900 °C, e.g., in the range of 700-850 °C, or 700-800 °C, or 700-750°C.

In some embodiments, the reverse water-gas shift reaction is conducted at a temperature in the range of 200-500 °C, e.g., 200-450 °C, or 200-400 °C, or 200-350 °C, or 250-500 °C, or 250-450 °C, or 250-400 °C, or 250-350 °C. The present inventors have noted that operation at these temperatures can provide for lower energy demand, as well as for facile integration with a subsequent Fischer-Tropsch process step.

As described above, the feed stream includes CO₂ and H₂. Advantageously, the present inventors have recognized that both of these can come from renewable or otherwise environmentally responsible sources. For example, at least part of the H₂ can be so-called "green" hydrogen, e.g., produced from the electrolysis of water operated using renewable electricity (such as wind, solar, or hydroelectric power). In other embodiments, at least part of the H₂ may be from a so-called "blue" source, e.g., from a natural gas reforming process with carbon capture. Of course, other sources of hydrogen can be used in part or in full. For example, in some embodiments, at least a portion of the H₂ of the feed stream is grey hydrogen, black hydrogen, brown hydrogen, pink hydrogen, turquoise hydrogen, yellow hydrogen, and/or white hydrogen. CO₂ can be captured from the environment generally, or more directly from processes that form CO₂ (especially in difficult-to-abate sectors), making a product that is later made from the CO at least carbon-neutral. For example, in some embodiments, at least part of the CO₂ is from direct air capture, or from a manufacturing plant such as a bioethanol plant (e.g., CO₂ produced fermentation), a steel plant, or a cement plant. Accordingly, the rWGS reaction can be not only carbon neutral, but in some cases a net consumer of carbon dioxide. These benefits in particular makes the rWGS reaction highly attractive for decarbonizing transportation fuels, for both automotive and aviation sectors, since the carbon monoxide produced in the reaction can be readily utilized by well-established technologies to synthesize liquid hydrocarbon fuels.

The feed stream contains both H₂ and CO₂ (e.g., provided to a reaction zone in a single physical stream or multiple physical streams). As used herein, the feed stream includes all feeds to the process, regardless of whether provided as a mixture of gases or as gases provided individually to a reaction zone. In various embodiments as otherwise described herein, the molar ratio of H₂ to CO₂ in the feed stream is at least 0.1:1, e.g., at least 0.5:1. In some embodiments, the molar ratio of H₂ to CO₂ in the feed stream is at least 0.9:1, e.g., at 1:1 or least 1.5:1. In some embodiments, the molar ratio of H₂ to CO₂ in the feed stream is at least 2:1, e.g., at least 2.5:1. In some embodiments, the molar ratio of H₂ to CO₂ in the feed stream is no more than 100:1, e.g., no more than 75:1, or 50:1. In some embodiments, the molar ratio of H₂ to CO₂ in the feed stream is no more than 20:1, e.g., no more than 15:1, or 10:1. For example, in some embodiments, the molar ratio of H₂ to CO₂ in the feed stream is in the range of 0.5:1 to 10:1. The person of ordinary skill in the art will provide a desired ratio of H₂:CO₂ in the feed stream, based on the disclosure herein, that provides a desirable conversion and selectivity; excess H₂ can, if consistent with a desirable conversion and selectivity, be provided to flow through the system and provide a product stream with a desirable ratio of H₂ to CO for a downstream process.

Other gases may also be included in the feed stream. For example, in some embodiments, the feed stream further comprises CO. In various embodiments as described herein, the first feed stream comprises no more than 20 mol%, no more than 10 mol%, or no more than 5 mol%, or no more than 3 mol%, or no more than 1 mol%, of CO. In some embodiments of the disclosure as otherwise described herein, the feed stream further comprises one or more inert gases. For example, in some embodiments, the feed stream further comprises nitrogen and/or methane. In various embodiments as described herein, the first feed stream comprises no more than 10 mol%, no more than 6 mol%, or no more than 2 mol%, of nitrogen. In various embodiments as described herein, the gases of first feed steam may be separated out to provide the amounts of carbon dioxide, methane, and/or nitrogen as described herein. For example, in some embodiments as described herein, methane is separated from the first feed stream to provide a first feed stream comprising at least 50 mol% carbon dioxide, e.g., at least 60 mol% carbon dioxide, at least 70 mol% carbon dioxide, at least 80 mol% carbon dioxide, or at least 90 mol% carbon dioxide.

The processes described herein can be performed at a variety of pressures, as would be appreciated by the person of ordinary skill in the art. In various embodiments of the present disclosure, the method for performing the reverse water-gas shift reaction is conducted at a pressure in the range of 1 to 100 barg. For example, the method is conducted at a pressure in the range of 1 to 70 barg, or 1 to 50 barg, or 1 to 40 barg, or 1 to 35 barg, or 5 to 70 barg, or 5 to 50 barg, or 5 to 40 barg, or 5 to 35 barg, or 10 to 70 barg, 10 to 50 barg, or 10 to 40 barg, or 10 to 35 barg, or 20 to 70 barg, 20 to 50 barg, or 20 to 40 barg, or 20 to 35 barg, or 25 to 70 barg, 25 to 50 barg, or 25 to 40 barg, or 25 to 35 barg.

The processes described herein can be performed at a variety of GHSV (gas hourly space velocity), as would be appreciated by the person of ordinary skill in the art. As such, the GHSV for performing the reverse water-gas shift reaction is not particularly limited. For example, in some embodiments of the present disclosure, the method for performing the reverse water-gas shift reaction is conducted at a GHSV in the range of 1,000 to 2,000,000 h⁻¹. In various embodiments, the method for performing the reverse water-gas shift reaction is conducted at a GHSV in the range of 1,000 to 1,200,000 h⁻¹, or 1,000 to 500,000 h⁻¹, or 1,000 to 100,000 h⁻¹, or 5,000 to 1,200,000 h⁻¹, or 5,000 to 500,000 h⁻¹, or 5,000 to 100,000 h⁻¹, or 10,000 to 1,200,000 h⁻¹, or 10,000 to 500,000 h⁻¹, or 10,000 to 100,000 h⁻¹. In various embodiments of the present disclose, the method for performing the reverse water-gas shift reaction is conducted at a GHSV in the range of 1,000 to 50,000 h⁻¹, or 2,000 to 50,000 h⁻¹, or 5,000 to 50,000 h⁻¹, or 10,000 to 50,000, or 1,000 to 40,000 h⁻¹, or 2,000 to 40,000 h⁻¹, or 5,000 to 40,000 h⁻¹, or 10,000 to 40,000 h⁻¹, or 1,000 to 30,000 h⁻¹, or 2,000 to 30,000 h⁻¹, or 5,000 to 30,000 h⁻¹, or 10,000 to 30,000 h⁻¹.

The rWGS catalyst described herein is based in part on platinum, palladium, gold, and/or nickel. It will typically be desirable to activate the rWGS catalyst, e.g., before contacting with the feed stream. Thus in some embodiments of the present disclosure as described herein, the method comprises activating the rWGS catalyst prior to contacting the catalyst with the feed stream. For example, in some embodiments, activating the catalyst comprises contacting the catalyst with a reducing stream comprising a reductive gas, e.g., hydrogen. In various embodiments of the present disclose, the reducing stream comprises hydrogen in an amount of at least 25 mol%, e.g., at least 50 mol%, or 75 mol%, or 90 mol%. The person of ordinary skill in the art will determine suitable conditions for activation of the rWGS catalyst. As such, the person or ordinary skill in the art would be able to choose an appropriate temperature, pressure, and time for activating the rWGS catalyst. For example, in various embodiments activating the catalyst is conducted at a temperature in the range of 200 °C to 1000 °C. In some embodiment, activating the catalyst is conducted at a temperature in the range of 250 °C to 1000 °C, or 300 °C to 1000 °C, 200 °C to 900 °C, or 250 °C to 900 °C, or 300 °C to 900 °C, 200 °C to 800 °C, or 250 °C to 800 °C, or 300 °C to 800 °C, or 200 °C to 700 °C, or 250 °C to 800 °C, or 300 °C to 700 °C. In some embodiments of the present disclosure as described herein, activating the catalyst provides a catalyst that is at least 10% reduced (e.g., at least 25%, or at least 50% reduced).

The present inventors have found that contacting the rWGS catalysts as described herein with a feed stream can provide a product stream with advantageously high CO selectivity and low methane selectivity. The amount of CO in the product stream can be further controlled by the rWGS reaction conditions, as described above. But in general, the methods for performing the rWGS reaction as described herein, provide a product stream comprising H₂ and CO, with the product stream having a lower concentration of CO₂ and a higher concentration of CO than the feed stream, as is consistent with the degrees of conversion described herein. For example, in various embodiments, the product stream includes no more than 95 mol% CO₂, or no more than 90 mol% CO₂. In some embodiments, the product stream includes no more than 85 mol% CO₂, or no more than 80 mol% CO₂. In other examples, the product stream includes no more than 75 mol%, or no more than 70 mol% CO₂. However, as described above, the present inventors have determined that it can be desirable to perform the processes at intermediate degrees of conversion to provide desirably high CO selectivities and desirably low methane selectivities. Accordingly, in various embodiments as otherwise described herein, the product stream includes an amount of CO₂ together with the CO.

Other gases may also be included in the product stream. In some embodiments of the disclosure as otherwise described herein, the product stream further comprises one or more inert gases. These inert gases may be included from the feed stream or provided from a source other than the feed stream. For example, in some embodiments, the product stream further comprises nitrogen and/or methane.

Depending on, inter alia, the degree of conversion, the CO selectivity, the relative amounts of H₂ and CO₂ in the feed stream, and the reaction conditions, the product stream can include H₂ in combination with CO, in a variety of ratios. For example, in some embodiments, the ratio of H₂:CO in the product stream is in the range of 0.1:1 to 100:1 (e.g., in the range of 0.1:1 to 50:1, or 0.1:1 to 25:1, or 0.1:1 to 10:1, or 0.1:1 to 5:1, or 1:1 to 100:1, or 1:1 to 50:1, or 1:1 to 25:1, or 1:1 to 10:1, or 1:1 to 5:1).

The person of ordinary skill in the art would appreciate that, based on the methods as described herein, the product stream may include H₂, CO, and CO₂ and other components in various amounts. Components of the product stream may be separated and used for various purposes in the rWGS process.

For example, in various embodiments of the present disclosure as described herein, the method further comprises separating the product stream to recycle at least a portion (e.g., at least 5 mol%, at least 10 mol%, at least 25 mol%, at least 50 mol%, at least 75 mol%, or at least 90 mol%) of one or more components of the product stream to the feed stream. For example, when the product stream includes CO₂, the method can include recycling at least a portion (e.g., at least 5 mol%, at least 10 mol%, at least 25 mol%, at least 50 mol%. at least 75 mol%, or at least 90 mol%) of the CO₂ of the product stream to the feed stream. The product stream may also include H₂; in some embodiments, the method further includes recycling at least a portion of H₂ of the product stream (e.g., at least 5 mol%, at least 10 mol%, at least 25 mol%, at least 50 mol%, at least 75 mol%, or at least 90 mol%) to the feed stream.

Such recycling is shown in the process 100 of FIG. 1 (and of FIG. 2). Here, the process 100 includes separating from the product stream 112 at least a portion of CO₂ (stream 114) to recycle to the feed stream 111. Similarly, the process 100 includes separating from the product stream 112 at least a portion of H₂ (stream 115) to recycle to the product stream 111. While stream 115 is depicted as entering reactor 110 through a different inlet than the rest of the feed stream 111, it is considered to be part of the feed stream, as it is part of the material input to the process step.

As noted above, one competing reaction in the reverse water-gas shift reaction is the Sabatier reaction, which makes methane. While in various embodiments the reverse water-gas shift processes described herein can be performed without forming large amounts of methane, in some embodiments there can be some methane formed. Accordingly, in various embodiments of the method as described herein, the product stream comprises one or more light hydrocarbons. For example, in some embodiments, the product stream may include one or more of methane, ethane, propane, or combinations thereof. When the first product steam includes methane, a substantial fraction of such methane may be from biogas provided to the first feed stream (e.g., at least 50%, at least 75%, or at least 90%). As would be understood by the person of ordinary skill in the art, it may be desirable to operate the reverse water-gas shift reaction to provide higher amounts of light hydrocarbons in the product feed. For example, such light hydrocarbons may be inert in further processing of the product stream and so may be acceptable at higher amounts, especially when biogas is used in the first feed stream. The person of ordinary skill in the art would be able to select appropriate reaction conditions (e.g., temperature, pressure, feed stream composition) to provide a product stream that includes methane at a desired amount. For example, in various embodiments as otherwise described herein, the product stream includes no more than 20 mol% methane or no more than 15 mol%. As noted above, when lower amounts of methane are desired in the product stream, the catalysts of the disclosure can provide very low methane selectivity. Additionally, when biogas is present in the first feed stream, methane may be separated before contacting with the reverse water-gas shift catalyst to provide a first feed stream and a first product stream with low amounts of methane. Accordingly, in various embodiments as otherwise described herein, the product stream includes no more than 10 mol% methane. For example, in various embodiments, the product stream includes no more than 5 mol%, or 1 mol%, or 0.5 mol%, or no more than 0.1 mol% methane. In general, light hydrocarbons (e.g., C₁-C₅ hydrocarbons) may be present in the product stream. For example, in various embodiments as otherwise described herein, the product stream includes no more than 20 mol% light hydrocarbons (e.g., no more than 15 mol%, no more than 10 mol%, no more than 5 mol%, no more than 1 mol%, no more than 0.5 mol%, or no more than 0.1 no mol% light hydrocarbons).

These light hydrocarbons (e.g., C₁-C₅ hydrocarbons) of the product stream can be separated and used for other purposes. For example, in various embodiments, the method further includes separating at least a portion of one or more light hydrocarbons from the product stream to provide a light hydrocarbon stream. For example, in method 100 of FIG. 1, at least a portion of one or more light hydrocarbons are separated from the product stream 112 to provide a light hydrocarbon stream 116. The light hydrocarbon stream, for example, can be used to provide other products, can be partially oxidized to form CO, can be steam reformed to provide hydrogen, and/or can be burned to provide heat or other energy (e.g., electricity for electrolysis) for use in the rWGS method or otherwise. In some embodiments as described herein, the light hydrocarbon stream comprises methane from biogas which can be burned to provide energy (e.g., heat energy or electrical energy) for use in the integrated process (e.g., for heating the first feed stream).
Of course, as would be understood by the ordinary skill in the art, the light hydrocarbon stream may be used in other processes as well. For example, as would be understood by the person of ordinary skill in the art, some rWGS catalysts can have reforming capability. Without being bound by theory, the present inventors hypothesize that one explanation for the low methane production observed using the rWGS catalysts as described herein is that methane is formed but then immediately reformed into CO and H₂. Accordingly, in some embodiments as described herein, the light hydrocarbons of the process stream is recycled to the feed stream for the rWGS reaction. These light hydrocarbons can be separated and used for other purposes. For example, in various embodiments, the process further includes separating at least a portion of one or more light hydrocarbons from the first product stream to provide a light hydrocarbon stream. For example, in process 100 of FIG. 2, at least a portion of one or more light hydrocarbons are separated from the first product stream 112 to provide a light hydrocarbon stream 118. The light hydrocarbon stream, for example, can be used to provide other products, can be partially oxidized to form CO, can be steam reformed to provide hydrogen, and/or can be burned to provide heat or other energy (e.g., electricity for electrolysis) for use in the integrated process or otherwise. Of course, as would be understood by the person of ordinary skill in the art, the light hydrocarbon stream may be used in other processes as well.

### Integrated Fischer-Tropsch Processes

In some embodiments as described herein, the supported reverse water-gas can be used in a rWGS process integrated with an FT process. The embodiments related to the reverse water-gas shift portion of the integrated FT process are as described above in the previous section. For example, the feed stream of the rWGS process corresponds to the first feed stream in the integrated FT process and the product stream of the rWGS process corresponds to the first product stream in the integrated FT process.

Another aspect of the present disclosure provides a process for performing an integrated Fischer-Tropsch process (i.e., integrated with an rWGS process). The process includes providing a first feed stream comprising H₂ and CO₂, wherein at least part of the CO₂ of the first feed stream is from biogas, a CO₂ emission source, and/or direct air capture; contacting at a first temperature in the range of 200-1100 °C and at a first pressure a reverse water-gas shift catalyst, as described herein, with the first feed stream to perform a reverse water-gas shift reaction to provide a first product stream comprising CO and H₂, the first product stream having a lower concentration of CO₂ and a higher concentration of CO than the first stream feed stream. An example of such a process is shown schematically in FIG. 2. In FIG. 2, the process 100 includes performing a reverse water-gas shift reaction by providing a first feed stream 111 comprising H₂ and CO₂, here, to a first reaction zone, e.g., a reactor 110. A reverse water-gas shift catalyst 113, as described herein, is contacted at a first temperature in the range of 250-1100 °C and at a first pressure with the feed stream 111 to provide a first product stream 112 comprising CO and H₂. The first product stream has a lower concentration of CO₂ and a higher concentration of CO than the first feed stream. The process of this aspect of the disclosure also includes contacting at a second temperature and at a second pressure a Fischer-Tropsch catalyst with a second feed stream comprising H₂ and at least a portion of CO of the first product stream to provide a second product stream comprising C₅+ hydrocarbons, In the process 100 of FIG. 2, at least a portion of CO of the first product stream 112 is included in second feed stream 121, which is contacted with Fischer-Tropsch catalyst 123, here, in a second reaction zone (e.g., a reactor 120). This provides a second product stream 122, which includes C₅+ hydrocarbons.

The present inventors have found that contacting the rWGS catalysts as described herein with a first feed stream can provide a first product stream with advantageously high CO selectivity and low methane selectivity. The amount of CO in the first product stream can be further controlled by the rWGS reaction conditions, as described above. However, as described above, the present inventors have determined that it can be desirable to perform the processes at intermediate degrees of conversion to provide desirably high CO selectivities and desirably low methane selectivities. Moreover, the present inventors have noted that it can be advantageous to perform the downstream Fischer-Tropsch process with a relatively high level of inerts, and thus contemplate that passing a significant amount of CO₂ to the Fischer-Tropsch process step can be beneficial. Accordingly, in various embodiments as otherwise described herein, the first product stream includes an amount of CO₂ together with the CO. In various embodiments, the first product stream comprises in the range of 5-95 mol% CO₂, e.g., 5-90 mol%, or 5-85 mol%, or 5-80 mol%, or 5-75 mol%, or 5-70 mol%, or 10-95 mol%, or 10-90 mol%, or 10-85 mol%, or 10-80 mol%, or 10-75 mol%, or 10-70 mol%, or 20-95 mol%, or 20-90 mol%, or 20-85 mol%, or 20-80 mol%, or 20-75 mol%, or 20-70 mol%, or 30-95 mol%, or 30-90 mol%, or 30-85 mol%, or 30-80 mol%, or 30-75 mol%, or 30-70 mol% CO₂.

Moreover, as described below, Fischer-Tropsch catalysts typically require activation by a reducing gas. As would be understood by the person of skill in the art, different Fischer-Tropsch catalysts required different activation conditions (e.g., gas composition, temperature, pressure, time). For example, iron based Fischer-Tropsch catalysts require activation with both H₂ and CO, while cobalt based Fischer-Tropsch catalysts require activation with just H₂. As such, H₂ and CO or just H₂ from the first product stream can be used to perform this activation. Accordingly, in various embodiments as otherwise described herein, the process includes separating at least a portion of H₂ and CO (desirably in a ratio of at least 1:1 or at least 3:1) from the first product stream and contacting it with the Fischer-Tropsch catalyst to activate the Fischer-Tropsch catalyst. In various other embodiments as otherwise described herein, the process includes separating at least a portion of H₂ from the first product stream and contacting it with the Fischer-Tropsch catalyst to activate the Fischer-Tropsch catalyst. For example, in the process of FIG. 2, stream 125 separates H₂ or H₂ and CO and conducts it to reactor 120. This separation need not be continuous; rather, it need only be performed for a time desirable to provide reducing gas to the Fischer-Tropsch catalyst for activation. Of course, as would be understood by the person of skill in the art, other sources of H₂ or CO may be used to provide reducing gas to the Fischer-Tropsch catalyst for activation.

As shown above, water is a product of the reverse water-gas shift reaction. Accordingly, the first product stream will generally contain water. In many cases it can be desirable to reduce the amount of water that is provided to the Fischer-Tropsch process step. Accordingly, in various embodiments as otherwise described herein, the process further includes removing at least a portion (e.g., at least 25%, at least 50%, or at least 75%) of water from the first product stream. In the embodiment of FIG. 2, a water removal zone 116 is used to remove water and provide a water-containing stream 117. The person of ordinary skill in the art will appreciate that a variety of processes can be used to remove water from the first product stream. For example, the first product stream can be contacted with a water scavenger to remove water therefrom. For example, a molecular sieve guard bed can be used to remove water from the first product stream; water can be recovered from the molecular sieves of the guard bed, e.g., by heating and vacuum. In other embodiments, a knockout vessel can be used. However, use of a knockout vessel can in some cases cool the first product stream enough so that it is desirably reheated for introduction to the Fischer-Tropsch process step. Water removed from the first product stream can be used, e.g., as feed water for electrolysis processes described herein.

As noted above, the reverse water-gas shift process can be provided at a wide variety of temperatures. In some cases, those temperatures can be relatively close to the temperature of the subsequent Fischer-Tropsch process step (often 150-400 °C, e.g., 200-350 °C, or other temperatures as described below). In other cases, the reverse water-gas shift process can be performed at temperatures significantly higher than the temperature of the Fischer-Tropsch step. The present inventors have noted that it can be desirable to provide for heat exchange with a relatively hot first product stream to cool the first product stream to a temperature more appropriate for the Fischer Tropsch step and to provide heat elsewhere to the integrated process. For example, in various embodiments of the processes as otherwise described herein, the process further comprises exchanging heat between at least a portion of the first product stream and at least a portion of the first feed stream, thereby cooling at least a portion of the first product stream and heating at least a portion of the first feed stream. An example of such a process is shown schematically in FIG. 3. In FIG. 3, the process 200, first reactor 210, first feed stream 211, first product stream 212, reverse water-gas shift catalyst 213, second reactor 220, second feed stream 221, second product stream 222 and Fischer-Tropsch catalyst 223 are generally as described above. Here, the process 200 includes exchanging heat between at least a portion of the first product stream 212 and a least a portion of the first feed stream 211 in a first heat exchange zone 230, thereby cooling at least a portion of the first product stream 212 and heating at least a portion of the first feed stream 211. The person of ordinary skill in the art will appreciate that a wide variety of heat exchangers can be used for this purpose.

Of course, any excess heat in the first product stream can be additionally or alternatively used for other purposes. For example, in various embodiments the process further comprises exchanging heat between at least a portion of the first product stream and a steam generation zone, thereby cooling at least a portion of the first product stream and providing heat to the steam generation zone. This is shown in FIG. 3. Here, after heat exchange with the first feed stream 211, the first product stream 212 is conducted to steam generation zone 232, to cool the first product stream 212 and provide heat to the steam generation zone 232. Steam can be generated from the heat provided, and electricity can be generated from the steam. For example, in the embodiment of FIG. 3, electricity stream 264 is provided by the generation of electricity using steam generated in the steam generation zone 232. Of course, as would be understood to the person of ordinary skill in the art, the steam generated in the steam generation zone may be used in other processes. In various embodiments, the steam may be used to heat the first feed stream. For example, in the embodiment of FIG. 3, the steam stream 266 generated in the steam generation zone 232 is conducted to the heat exchange zone 290 to heat the first feed stream 211.

As noted above, at least a portion of the CO of the first product stream is included in the second feed stream, for reaction in a Fischer-Tropsch process. For example, in various embodiments as otherwise described herein, at least 25% of the CO of the first product stream, e.g., at least 50% of the CO, at least 75% of the CO, or at least 90% of the CO of the first product stream is included in the second feed stream. Of course, as noted above, some of the CO of the first product stream can be used for other purposes, e.g., catalyst activation as described herein.

In some embodiments, substantially all of the CO of the second feed stream comes from the first product stream. However, in other embodiments, CO can be provided to the second feed stream from other sources, fossil-derived or otherwise. For example, in various embodiments, CO is provided to the second feed stream from a CO source other than the first product stream. In FIG. 3, a stream of CO 226a from some other source is included in the second feed stream 221. The person of ordinary skill in the art will appreciate that CO can be provided from a variety of sources, e.g., gasification, reforming, or electrochemical CO₂ reduction. Moreover, as described in more detail below, CO can be recycled to the second feed stream from the second product stream; and/or can be provided by reaction of a light hydrocarbon stream, e.g., by partial oxidation or reforming (e.g., steam reforming and/or autothermal reforming)..

As noted above, the second feed stream includes H₂. Notably, the first product stream will often include H₂, e.g., unreacted from the first feed stream. In various embodiments, the first product stream includes H₂ wherein the second feed stream includes at least a portion of the H₂ of the first product stream. For example, in various embodiments as otherwise described herein, at least 25% of the H₂ of the first product stream, e.g., at least 50% of the H₂, at least 75% of the H₂, or at least 90% of the H₂ of the first product stream is included in the second feed stream. Of course, as noted above, some of the H₂ of the first product stream can be used for other purposes, e.g., catalyst activation as described herein.

In some embodiments, substantially all of the H₂ of the second feed stream comes from the first product stream. In fact, the person of ordinary skill in the art can provide more H₂ than necessary for the reverse water-gas shift reaction in the first feed stream, to provide excess H₂ in the first product stream that can then provide a desired amount of H₂ to the second feed stream for the Fischer-Tropsch process step. However, in other embodiments, H₂ can be provided to the second feed stream from other sources. For example, in various embodiments, H₂ is provided to the second feed stream from a H₂ source other than the first product stream. In FIG. 3, a stream of H₂ 226b from some other source is included in the second feed stream 221. The person of ordinary skill in the art will appreciate that H₂ can be provided from a variety of sources, e.g., gasification, reforming, or H₂O electrolysis (including the electrolysis described herein). Moreover, as described in more detail below, H₂ can be recycled to the second feed stream from the second product stream.

The person of ordinary skill in the art can, based on the disclosure herein, adjust the relative amounts of H₂ and CO in the second feed stream to provide a desired ratio. For example, more or less H₂ of the first feed stream and/or more or less H₂ from electrolysis can be included in the second feed stream. Similarly, more or less CO of the first feed stream and more or less CO from other sources (e.g., partial oxidation and reforming as described below) can be included in the second feed stream.

As noted above, it can be desirable to perform the Fischer-Tropsch process step in the presence of a significant level of inerts. One such inert, CO₂, can come from the reverse water-gas shift, e.g., via the first product stream. Accordingly, in various embodiments as otherwise described herein, the second feed stream includes at least a portion of CO₂ of the first product stream. For example, in various embodiments, at least 10% of the CO₂ of the first product stream, e.g., at least 25% of the CO₂, at least 50% of the CO₂, at least 75% of the CO₂, or at least 90% of the CO₂ of the first product stream is included in the second feed stream. Of course, in other embodiments, the second feed stream may not include any substantial amount of CO₂ of the first product stream. Accordingly, in various embodiments, the second feed stream does not include a substantial amount of CO₂ of the first product stream. While it can be desirable generally to recycle CO₂ to the first feed stream for use in the reverse water-gas shift reaction, as described in more detail below, unreacted CO₂ can be recycled from the second product stream to the first feed stream.

But it can additionally or alternatively be desirable to include additional inert content to the second feed stream, be it CO₂ or other inerts such as nitrogen and methane. For example, in various embodiments, one or more inerts (e.g., CO₂, nitrogen and/or methane) are provided to the second feed stream from a source other than the first product stream. In FIG. 3, a stream of inert(s) 226c from some other source is included in the second feed stream 221. The person of ordinary skill in the art will appreciate that inerts can be provided from a variety of sources. Moreover, as described in more detail below, inerts can be recycled to the second feed stream from the second product stream.

As noted above, it can be desirable to perform the Fischer-Tropsch process step in the presence of inerts. Accordingly, in various embodiments as otherwise described herein, the portion of the first product stream that is included in the second feed stream has a CO₂ content in the range of 10-95 mol% CO₂, e.g., 10-90 mol%, or 10-85 mol%, or 10-80 mol%, or 10-75 mol%, or 10-70 mol%, or 20-95 mol%, or 20-90 mol%, or 20-85 mol%, or 20-80 mol%, or 20-75 mol%, or 20-70 mol%, or 30-95 mol%, or 30-90 mol%, or 30-85 mol%, or 30-80 mol%, or 30-75 mol%, or 30-70 mol% CO₂.

Other gases may also be included in the second feed stream, as described above. For example, as noted above, it can be desirable to perform the Fischer-Tropsch process step in the presence of a significant amount of inerts (i.e., components that are not H₂ or CO). For example, in various embodiments, the second feed stream includes up to 80 mol% of one or more inerts, e.g., in the range of 3-80 mol%, or 5-80 mol%, or 10-80 mol%, or 15-80 mol%, or 30-80 mol% of one or more inerts. In various embodiments, the second feed stream includes up to 70 mol% inerts, up to 60 mol% inerts, or up to 50 mol% inerts, e.g., 3-70 mol%, or 5-70 mol%, or 10-70 mol%, or 15-70 mol%, or 30-70 mol%, or 3-60 mol%, or 5-60 mol%, or 10-60 mol%, or 15-60 mol%, or 30-60 mol%, or 3-50 mol%, or 5-50 mol%, or 10-50 mol%, or 15-50 mol%, or 30-50 mol% inerts. In various embodiments, the second feed stream includes up to 80% of one or more inerts selected from CO₂, methane and nitrogen, e.g., up to 70 mol%, up to 60 mol%, or up to 50 mol%, or 15-70 mol%, or 30-70 mol%, or 15-60 mol%, or 30-60 mol%, or 15-50 mol%, or 30-50 mol%. In various embodiments, the second feed stream includes up to 80 mol% of CO₂, e.g., up to 70 mol%, up to 60 mol%, or up to 50 mol%, or 15-70 mol%, or 30-70 mol%, or 15-60 mol%, or 30-60 mol%, or 15-50 mol%, or 30-50 mol%.

The person of ordinary skill in the art can tune the portion of the first product stream that is included in the second feed stream to provide a desirable H₂:CO ratio. For example in various embodiments, the portion of the first product stream that is included in the second feed stream has a H₂:CO ratio in the range of 0.5:1 to 10:1, e.g., in the range of 1:1 to 2.5:1. Of course, whatever the H₂:CO ratio of the portion of the first product stream that is included in the second feed stream, the person of ordinary skill in the art can add H₂ or CO as described above as necessary to provide the desired ratio overall in the second feed stream.

As described above, the second feed stream contains both H₂ and CO and the second feed stream includes all feeds to the Fischer Tropsch reactor, regardless of whether the second feed stream is provided as a mixture of feeds or as feeds provided individually to a reaction zone. In various embodiments of the present disclosure as described herein, the second feed stream has a H₂:CO ratio in the range of 0.5:1 to 6:1. In some embodiments, the second feed stream has a H₂:CO ratio in the range of 1:1 to 3:1, or 1:1 to 2.5:1. In some embodiments, the second feed stream has a H₂:CO ratio of at least 1.4:1. For example, in some embodiments, the second feed stream has a H₂:CO ratio in the range of 1.4:1 to 3:1, or 1.4:1 to 2:1. The person of ordinary skill in the art will provide a desired ratio of H₂:CO in the second feed stream, based on the disclosure herein that provides a desirable conversion and selectivity in the Fischer-Tropsch process.

As noted above it can be desirable to reduce the amount of water that is conducted to the Fischer-Tropsch process step. Accordingly, in various embodiments as otherwise described herein, the portion of the first product stream that is included in the second feed stream has a water content of no more than 10 mol%, e.g., or no more than 2 mol%, or no more than 0.5 mol%.

And as noted above, it can be desirable to perform the Fischer-Tropsch process with a relatively small amount of water present. Accordingly, in various embodiments, the second feed stream has a water content of no more than 10 mol%, e.g., or no more than 2 mol%, or no more than 0.5 mol%.

The processes as described here include contacting a Fischer-Tropsch catalyst with the second feed stream as described herein. The Fischer-Tropsch catalyst for use in the processes as described herein is not particularly limited and the person of ordinary skill in the art would be able to choose a catalyst as appropriate for their desired Fischer-Tropsch product. In some embodiments, the Fischer-Tropsch catalyst includes cobalt, iron, rhodium, ruthenium, or a combination thereof.

For example, in some embodiments of the present disclosure as described herein, the Fischer-Tropsch catalyst comprises cobalt, e.g., in an amount in the range of 5-25 wt%, calculated as Co(0). "Calculated as Co(0)" and analogous terms mean that the weight of cobalt atoms/ions themselves are used in the calculation, and not the total amount of any compound or polynuclear ion in which those cobalt atoms/ions might be bound. For example, in various embodiments, the Fischer-Tropsch catalyst comprises cobalt in an amount in the range of 7-25 wt%, or 10-25 wt%, or 5-20 wt%, or 7-20 wt%, or 10-20 wt%, calculated as Co(0). As the person of ordinary skill in the art will appreciate, cobalt-based catalysts are often provided to the reaction zone in the form of cobalt oxide on a support; the cobalt can be reductively activated (e.g., with H₂) in situ to provide an active catalyst species with a significant concentration of Co(0).

In some embodiments, the Fischer-Tropsch catalyst comprises iron, e.g., in an amount in the range of 5-95 wt%, calculated as Fe(0). For example, in various embodiments, the Fischer-Tropsch catalyst comprises iron in the range of 10-95 wt%, or 25-95 wt%, or 50-95 wt%, or 5-85 wt%, or 10-85 wt%, or 25-85 wt%, or 50-85 wt%, or 5-75 wt%, or 10-75 wt%, or 25-75 wt%, calculated as Fe(0). As the person of ordinary skill in the art will appreciate, iron-based catalysts are often provided to the reaction zone in the form of metallic iron or iron oxide, optionally on a support; the iron can be activated (e.g., by reaction with H₂ and CO) to provide an active catalyst species with a significant concentration of iron carbide.

In various embodiments of the disclosure as described herein, especially when the catalyst is a cobalt-based catalyst, the Fischer-Tropsch catalyst further includes manganese. For example, in various embodiments, the Fischer-Tropsch catalyst includes manganese in an amount up to 15 wt%, e.g., up to 12 wt%, or up to 10 wt%, or up to 7 wt%, calculated as Mn(0). In certain such embodiments, a catalyst material includes manganese in an amount in the range of 0.1-15 wt%, e.g., 0.1-10 wt%, or 0.1-5 wt%, 0.5-15 wt%, or 0.5-10 wt%, or 0.5-5 wt%, or calculated as Mn(0). Of course, in other embodiments substantially no manganese is present (e.g., less than 0.1 wt% or less than 0.5 wt% manganese is present).

The Fischer-Tropsch catalysts suitable for use in the process as described herein can be a variety of forms and are not particularly limited. For example, the Fischer-Tropsch catalyst may be a supported or unsupported catalyst. While the form of the catalyst is not particularly limited, in various desirable embodiments, the Fischer-Tropsch catalyst is a supported catalyst, wherein the support comprises at least one of titanium oxide, zirconium oxide, cerium oxide, aluminum oxide, silicon oxide and zinc oxide. For example, in various embodiments, the support comprises at least one or titanium oxide, aluminum oxide, and silicon oxide. In some embodiments of the present disclosure as described herein, the support is a titanium dioxide support.

The person of ordinary skill in the art will appreciate that the Fischer-Tropsch catalysts of the disclosure can be provided in many forms, depending especially on the particular form of the reactor system in which they are to be used, e.g., in a fixed bed or as a fluidized bed. The supports of the Fischer-Tropsch catalysts can be provided themselves as discrete bodies of material, e.g., as porous particles, pellets or shaped extrudates, with the metals provided thereon to provide the Fischer-Tropsch catalyst. However, in other embodiments, a Fischer-Tropsch catalyst of the disclosure can itself be formed as a layer on an underlying substrate. The underlying substrate is not particularly limited. It can be formed of, e.g., a metal or metal oxide, and can itself be provided in a number of forms, such as particles, pellets, shaped extrudates, or monoliths. The person of ordinary skill in the art will select an appropriate Fischer-Tropsch catalyst for the particular reactor system.

As with the rWGS catalyst, Fischer-Tropsch catalysts are typically activated before use, e.g., to provide cobalt(0) species on a cobalt-based catalyst, or iron carbide species on an iron-based catalyst. Such activation can be performed prior to contacting the Fischer-Tropsch catalyst with a second feed stream.

For example, in some embodiments, the Fischer-Tropsch catalyst is activated by contact with a reducing gas. For example, hydrogen can be an especially suitable gas for activating Fischer-Tropsch catalyst, e.g., when the activation is a reduction to metal(0) species, e.g., as for many cobalt-based catalysts. In various embodiments of the present disclosure as otherwise described herein, the reducing gas comprises at least a portion of H₂ from the first product stream. For example, in some embodiments, the process further comprises separating at least a portion of H₂ of the first product stream and contacting it with the Fischer-Tropsch catalyst to activate Fischer-Tropsch catalyst. In the process 100 shown schematically in FIG. 2, at least a portion of hydrogen stream 125 is separated from the first product stream 112 and contacted with the Fischer-Tropsch catalyst 123 to activate it. In other embodiments, H₂ present in the second feed stream can be used to activate the catalyst. As would be understood by the person of ordinary skill in the art, activation temperatures can vary depending on the Fischer-Tropsch catalyst used. As such, the person of ordinary skill in the art would be able to select an appropriate temperature for activating the catalyst, e.g., in the range of 200-400 °C.

In various embodiments, the Fischer-Tropsch catalyst is activated by contact with H₂ and CO. This can be especially suitable when the activation provides conversion to carbide, e.g., as for many iron-based catalysts. In various embodiments of the present disclosure as otherwise described herein, the reducing gas comprises at least a portion of H₂ and CO from the first product stream. For example, in some embodiments, the process further comprises separating at least a portion of H₂ and at least a portion of CO of the first product stream and contacting it with the Fischer-Tropsch catalyst to activate Fischer-Tropsch catalyst. In the process 200 shown schematically in FIG. 3, at least a portion of H₂ and CO stream 227 is separated from the first product stream 212 and contacted with the Fischer-Tropsch catalyst 223 to activate it. In other embodiments, H₂ and CO present in the second feed stream can be used to activate the catalyst. Activation temperatures can vary, e.g., in the range of 200-400 °C.

As described above, the process includes contacting at a second temperature and at a second pressure a Fischer-Tropsch catalyst with a second feed stream. The person of ordinary skill in the art will select appropriate reaction conditions in conjunction with the particular feed and catalyst used to provide desired Fischer-Tropsch processes. In some embodiments of the disclosure as described herein, the second temperature is in the range of 150-400 °C. For example, in various embodiments, the second temperature is in the range of 150-350 °C, or 150-300 °C, or 150-250°C, or 150-200°C, or 200-400 °C, or 200-350 °C, or 200-300°C, or 200-250 °C, or 250-400 °C, or 250-350 °C, or 250-300 °C, or 300-400 °C. In some particular embodiments, the second temperature is in the range of 200-350 °C.

Notably, in many embodiments, the first temperature and the second temperature can be relatively close to one another. The present inventors have noted that the reverse water-gas shift catalysts described herein can provide suitable activity and CO selectivity even at relatively low temperatures. Accordingly, the first product stream can be provided with a temperature that is suitable for, or at least close to suitable for, the Fischer-Tropsch reaction step. This can desirably provide for increased process integration. For example, in various embodiments, the first temperature is within 100 °C of the second temperature, e.g., within 50 °C of the second temperature, or within 25 °C of the second temperature.

However, in other embodiments, the first temperature and the second temperature are less close to one another. The present inventors have noted that in many cases a desirable reverse water-gas shift process temperature will be significantly greater than a desirable Fischer-Tropsch process temperature. For example, in various embodiments, the first temperature is at least 100 °C greater than the second temperature, e.g., at least 150 °C greater than the second temperature, or at least 200 °C greater than the second temperature. The excess heat in the first product stream can be used for a number of purposes, for example, to preheat at least part of the first feed stream or to generate steam for use in generating electricity, as described above.

In some embodiments of the disclosure as described herein, the second pressure is in the range of 10-50 barg. For example, in various embodiments, the second pressure is in the range of 20-50 barg, or 25-50 barg, or 10-40 barg, or 20-40 barg, or 25-40 barg or 10-35 barg, or 20-35 barg, or 25-35 barg. In some embodiments, the second pressure is in the range of 20-50 barg.

The Fischer-Tropsch processes described herein can be performed at a variety of GHSV (gas hourly space velocity) values, as would be appreciated by the person of ordinary skill in the art. As such, the GHSV for performing the Fischer-Tropsch reaction is not particularly limited. For example, in some embodiments of the present disclosure, the process for performing the Fischer-Tropsch reaction is conducted at a GHSV in the range of 1,000 to 2,000,000 h⁻¹. In various embodiments, the process for performing the reverse water-gas shift reaction is conducted at a GHSV in the range of 1,000 to 1,200,000 h⁻¹, or 1,000 to 500,000 h⁻¹, or 1,000 to 100,000 h⁻¹, or 5,000 to 1,200,000 h⁻¹, or 5,000 to 500,000 h⁻¹, or 5,000 to 100,000 h⁻¹, or 10,000 to 1,200,000 h⁻¹, or 10,000 to 500,000 h⁻¹, or 10,000 to 100,000 h⁻¹. In various embodiments of the present disclose, the process for performing the Fischer-Tropsch reaction is conducted at a GHSV in the range of 1,000 to 50,000 h⁻¹, or 2,000 to 50,000 h⁻¹, or 5,000 to 50,000 h⁻¹, or 10,000 to 50,000, or 1,000 to 40,000 h⁻¹, or 2,000 to 40,000 h⁻¹, or 5,000 to 40,000 h⁻¹, or 10,000 to 40,000 h⁻¹, or 1,000 to 30,000 h⁻¹, or 2,000 to 30,000 h⁻¹, or 5,000 to 30,000 h⁻¹, or 10,000 to 30,000 h⁻¹.

The Fischer-Tropsch process is typically used to make C₅₊ hydrocarbons, for example, unsubstituted C₅₊ hydrocarbons (e.g., alkanes and alkenes) and oxygenated C₅₊ hydrocarbons (e.g., C₅₊ alcohols, aldehydes, ketones, carboxylic acids). In various embodiments of the disclosure as described herein, contacting the Fischer-Tropsch catalyst with the second feed stream to provide the second product stream is performed with a C₅₊ selectivity (i.e., for all C₅₊ species) of at least 30%, e.g., at least 50%, or at least 70%. For example, in some embodiments, the selectivity for C₅₊ alkanes is at least 30%, e.g., at least 50%, or at least 70%. In some embodiments, the selectivity for C₅₊ alkanes and C₅₊ alcohols is at least 30%, e.g., at least 50%, or at least 70%.

Additional components may be in present in the second product stream. For example, in some embodiments, the second product stream includes water, which is another product of the Fischer-Tropsch reaction. Also present can be one or more light hydrocarbons (i.e., C₁-C₄) as a side product. CO and/or H₂ can be present, e.g., unreacted from the second feed stream. CO₂ or other inerts as described herein can also be present. Such components of the second product stream can be separated and/or recycled in various manners. When the second product steam includes methane, such methane may be substantially from biogas provided to the first feed stream (e.g., at least 50%, at least 75%, or at least 90%).

For example, in various embodiments, the process further comprises separating at least a portion of water from the second product stream. This is shown schematically in FIG. 4. In the embodiment of FIG. 4, the reverse water-gas shift catalyst 313 and the Fischer-Tropsch catalyst 323 are provided in separate beds in the same reactor. Thus, the first reaction zone 310 is a volume of the reactor 305 that includes the bed 314 containing the reverse water-gas shift catalyst 313, and the second reaction zone 320 is a volume of the reactor 305 that includes the bed 324 containing the Fischer-Tropsch catalyst 323. First feed stream 311 is contacted with the reverse water-gas shift catalyst 313 to provide first product stream 312, which is passed directly as the second feed stream 321 to the Fischer-Tropsch catalyst 323 to provide second product stream 322. Here, the process also optionally includes separating at least a portion of water (e.g., at least 50%, at least 75%, or at least 90%) from the second product stream 322 to provide water-containing stream 334.

Light hydrocarbons, while often not a desired portion of a Fischer-Tropsch product to be used as a fuel or a lubricant, can themselves be useful for a number of purposes. Accordingly, in various embodiments, the process further includes separating at least a portion of C₁-C₄ hydrocarbons from the second product stream to provide a light hydrocarbon stream. The light hydrocarbon stream can, for example, be recycled to the first feed stream or the second feed stream. For example, in the process 200 of FIG. 3, light hydrocarbons can be provided as part of the recycle stream 236, which becomes part of the second feed stream 221. In the process 300 of FIG. 4, light hydrocarbons can be provided as part of the recycle stream 336, which becomes part of the first feed stream 311. In the process 400 of FIG. 5, light hydrocarbons are recycled via recycle stream 442 to first feed stream 411.

There are other uses for the light hydrocarbon stream. For example, in some embodiments, the process further comprises oxidizing at least a portion of the light hydrocarbon stream to provide a CO- and/or CO₂-containing partial oxidation (pOX) stream, and including at least a portion of the pOX stream in the first feed stream and/or the second feed stream. In some embodiments as described herein, the light hydrocarbon stream comprises methane from biogas. In some embodiments herein, at least 50% of methane of the light hydrocarbon stream is methane from biogas. An example of such a process is shown schematically in FIG. 5, in which the process 400, the first feed stream 411, the first product stream 412, the reverse water-gas shift catalyst 413, the second feed stream 421, the second product stream 422 and the Fischer-Tropsch catalyst 423 can be as otherwise described herein. Here, the process includes oxidizing at least a portion of the light hydrocarbon stream 450) in a partial oxidation reaction zone 452 to provide a CO- and/or CO₂ containing pOX stream, and including at least a portion of the pOX stream 454 stream in the first feed stream 411 and/or the second feed stream 421.

As described above, at least part of the CO₂ of the first feed stream may be from biogas. In some embodiments as described herein, the process includes providing a biogas comprising CO₂ and methane, and providing at least a portion of the CO₂ to the first feed stream, and at least a portion of the methane to the oxidation of at least a portion of the light hydrocarbon stream as shown in the embodiment of FIG. 6.

Other methods can be used to provide CO and/or CO₂ from the light hydrocarbon stream. For example, reforming techniques such as steam reforming and autothermal reforming can be used to provide CO by reaction of hydrocarbons with water. Accordingly, in various embodiments, the process further comprises reforming (e.g., steam reforming and/or autothermal reforming) at least a portion of the light hydrocarbon stream to provide a CO- and/or CO₂-containing reformed stream, and including at least a portion of the reformed stream in the first feed stream and/or the second feed stream. Water separated from the first and/or second product streams can be provided as part of a feed to the reforming described herein.

Moreover, the light hydrocarbon stream can be burned to provide heat energy, which can be used to heat various process streams, or to generate electricity. Accordingly, in various embodiments, the process includes burning at least a portion of the light hydrocarbon stream to provide energy, e.g., heat energy or electrical energy. For example, in the process 400 of FIG. 5, a portion of light hydrocarbon stream 450 is burned in a power generation zone (here, in an electrical generator 470), to generate electricity stream 472. In various embodiments, the heat energy may be used to provide the needed heat duty for the reverse water-gas shift process. For example, in the process 400 of FIG. 5, a portion of the light hydrocarbon stream 450 is burned in a power generation zone (here, in a heat generator 480), to generate heat stream 482. The heat stream 482 is conducted to a heat exchange zone 490 to heat the first feed stream 411. Heat energy can similarly be provided to the Fischer-Tropsch reaction. And as the person of ordinary skill in the art will appreciate, other treatments of the light hydrocarbon stream (e.g., partial oxidation) can also provide energy, which can be used, e.g., as described herein.

As with the first product stream, heat can be exchanged from the second product stream to provide heat to, for example, a feed stream or a steam generation zone. For example, in various embodiments, the process further comprises exchanging heat between at least a portion of the second product stream and at least a portion of the first feed stream, thereby cooling at least a portion of the second product stream and heating at least a portion of the first feed stream. In process 300 of FIG. 4, heat is exchanged between at least a portion of the second product stream 322 and first feed stream 311 in a second heat exchange zone 330, thereby cooling the second product stream 322 and heating the first feed stream 311. Of course, heat can also be exchanged from the second product stream to the second feed stream. For example, in various embodiments, the process further comprises exchanging heat between at least a portion of the second product stream and at least a portion of the second feed stream, thereby cooling at least a portion of the second product stream and heating at least a portion of the second feed stream. In process 400 of FIG. 5, heat is exchanged between at least a portion of the second product stream 422 and second feed stream 421 in a second heat exchange zone 430, thereby cooling the second product stream 422 and heating the second feed stream 421. The person of ordinary skill in the art will appreciate that a wide variety of heat exchangers can be used for this purpose.

Of course, any excess heat in the second product stream can be additionally or alternatively used for other purposes. For example, in various embodiments the process further comprises exchanging heat between at least a portion of the second product stream and a steam generation zone, thereby cooling at least a portion of the second product stream and providing heat to the steam generation zone. This is shown in FIG. 4. Here, after heat exchange with the first feed stream 311, the second product stream 322 is conducted to steam generation zone 332, to cool the second product stream 322 and provide heat to the steam generation zone 332. Steam can be generated from the heat provided, and electricity can be generated from the steam (not shown here).

It can be desirable to recycle hydrogen from the second product stream, for example, to the first feed stream and/or the second feed stream. For example, in various embodiments, the process includes recycling at least a portion of H₂ of the second product stream to the second feed stream. For example, in the process of FIG. 3, at least a portion of H₂ of the second product stream (e.g., at least 25%, at least 50%, or at least 75%) can be recycled to the second feed stream 221 via recycle stream 236. In various embodiments, the process includes recycling at least a portion of H₂ of the second product stream to the first feed stream. For example, in the process of FIG. 4, at least a portion of H₂ of the second product stream (e.g., at least 25%, at least 50%, or at least 75%) can be recycled to the first feed stream 311 via recycle stream 336. In various embodiments, at least 25%, e.g., at least 50% of H₂ of the second product stream is recycled to the first feed stream or the second feed stream. In various embodiments, at least 75%, e.g., at least 90% of H₂ of the second product stream is recycled to the first feed stream or the second feed stream.

In some cases, e.g., when H₂ is provided to the second feed stream from an H₂ source other than the first product stream, H₂ from the second product stream can make up most of the H₂ of the first feed stream, e.g., at least 90%, at least 95%, or at least 98% of the H₂ of the first feed stream. This is shown, e.g., in FIG. 5. Here, the primary H₂ input to the process is through stream 440, which becomes part of the second feed stream 421. H₂ of the second product stream is included in recycle stream 442, which becomes part of first feed stream 411.

Similarly, it can be desirable to recycle CO of the second product stream, for example, to the first feed stream and/or the second feed stream. For example, in various embodiments, the process includes recycling at least a portion of CO of the second product stream to the second feed stream. For example, in the process of FIG. 3, at least a portion of CO of the second product stream (e.g., at least 25%, at least 50%, or at least 75%) can be recycled to the second feed stream 221 via recycle stream 236. In various embodiments, the process includes recycling at least a portion of CO of the second product stream to the first feed stream. For example, in the process of FIG. 4, at least a portion of CO of the second product stream (e.g., at least 25%, at least 50%, or at least 75%) can be recycled to the first feed stream 311 via recycle stream 336. In various embodiments, at least 25%, e.g., at least 50% of CO of the second product stream is recycled to the first feed stream or the second feed stream. In various embodiments, at least 75%, e.g., at least 90% of CO of the second product stream is recycled to the first feed stream or the second feed stream.

In many cases, both CO and H₂ of the second product stream will be recycled.

Moreover, when one or more inerts are used in the Fischer-Tropsch process step, it can be desirable to recycle these. For example, in various embodiments, the process includes recycling at least a portion of inerts of the second product stream to the second feed stream. For example, in the process of FIG. 3, at least a portion of inerts of the second product stream (e.g., at least 25%, at least 50%, or at least 75%) can be recycled to the second feed stream 221 via recycle stream 236. In various embodiments, the process includes recycling at least a portion of inerts of the second product stream to the first feed stream. For example, in the process of FIG. 4, at least a portion of inerts of the second product stream (e.g., at least 25%, at least 50%, or at least 75%) can be recycled to the first feed stream 311 via recycle stream 336. In various embodiments, at least 25%, e.g., at least 50% of inerts of the second product stream is recycled to the first feed stream or the second feed stream. In various embodiments, at least 75%, e.g., at least 90% of inerts of the second product stream is recycled to the first feed stream or the second feed stream. In various embodiments, a purge stream can be incorporated with the recycle stream to prevent uncontrolled accumulation of inerts in the recycle stream (not shown here).

Specifically, as CO₂ is the carbon source for the reverse water-gas shift process step, it can be especially desirable to recycle CO₂ to the first feed stream. Accordingly, in various embodiments, the process includes recycling at least a portion (e.g., at least 50%, at least 75%, or at least 90%) of CO₂ of the second product stream to the first feed stream. For example, in the process of FIG. 4, at least a portion of CO₂ of the second product stream (e.g., at least 50%, at least 75%, or at least 90%) can be recycled to the first feed stream 311 via recycle stream 336.

In some cases, e.g., when CO₂ is provided to the second feed stream from a CO₂ source other than the first product stream, CO₂ from the second product stream can make up most of the CO₂ of the first feed stream, e.g., at least 90%, at least 95%, or at least 98% of the CO₂ of the first feed stream. This is shown, e.g., in FIG. 5. Here, the primary CO₂ input to the process is through stream 440, which becomes part of the second feed stream 421. CO₂ of the second product stream is included in recycle stream 442, which becomes part of first feed stream 411.

As noted above, the Fischer-Tropsch process step provides a second product stream that includes C₅₊ hydrocarbons (e.g., unsubstituted hydrocarbons like alkanes and alkenes, and/or oxygenated hydrocarbons such as alcohols). Accordingly, in various embodiments, one or more products are provided from at least a portion of C₅₊ hydrocarbons of the second product stream. The C₅₊ hydrocarbons can be used as the basis of a variety of fuels, e.g., gasoline, diesel, aviation fuel. Other products, like waxes and lubricants, can also be made. And alkenes and oxygenates can be used as feedstocks in a variety of other processes.

The person of ordinary skill in the art will use conventional post-processing techniques to convert the C₅₊ hydrocarbon-containing product to desirable products such as desirable fuels. For example, in various embodiments, the process further includes hydroprocessing at least a portion of C₅₊ hydrocarbons of the second product stream. As the person of ordinary skill in the art will appreciate, hydroprocessing is a treatment of the hydrocarbon stream with hydrogen in the presence of a suitable catalyst. A wide variety of hydroprocessing techniques are known, and the person of ordinary skill in the art will apply them here. For example, in the process 300 of FIG. 4, second product stream 322 is hydroprocessed in hydroprocessing reactor 350, to provide a hydroprocessed product stream 352.

As described above, CO₂ and H₂ are substantial inputs to the claimed processes. Advantageously, the present inventors have recognized that each of these can come from renewable or otherwise environmentally responsible sources. As described above, a least a part of the CO₂ of the first feed stream is from biogas, a CO₂ emission source, and/or direct air capture. A part of the CO₂ of the second feed stream may also be from biogas, a CO₂ emission source, and/or direct air capture.

Accordingly, in some embodiments of the disclosure as described herein, at least a part of the CO₂ of the first feed stream and/or the second feed stream is from a renewable source. In some embodiments, at least part (e.g., at least 25%, at least 50%, or at least 75%) of the CO₂ of the first feed stream and/or the second feed stream is from direct air capture. In some embodiments, at least part (e.g., at least 25%, at least 50%, or at least 75%) of the CO₂ of the first feed stream and/or the second feed stream is from a manufacturing plant such as a bioethanol plant (e.g., CO₂ produced fermentation), a steel plant, or a cement plant. Accordingly, the rWGS-Fischer Tropsch integrated processes of the disclosure as described herein can be not only carbon neutral, but in some cases a net consumer of carbon dioxide. These benefits in particular make the integrated processes highly attractive for decarbonizing transportation fuels, for both automotive and aviation sectors, since the carbon monoxide produced in the rWGS reaction can be readily utilized by well-established technologies to synthesize liquid hydrocarbon fuels by Fischer-Tropsch processes.

Similarly, H₂ can be provided from environmentally-responsible sources. In some embodiments, at least a part of the H₂ of the first feed stream and/or the second feed stream is from a renewable source. For example, in various embodiments, at least part (e.g., at least 25%, at least 50%, or at least 75%) of the H₂ of the first feed stream and/or the second feed stream can be so-called "green" hydrogen, e.g., produced from the electrolysis of water operated using renewable electricity (such as wind, solar, or hydro-electric power). In some embodiments, at least part (e.g., at least 25%, at least 50%, or at least 75%) of the H₂ of the first feed stream and/or the second feed stream may be from a so-called "blue" source, e.g., from a natural gas reforming process with carbon capture. Of course, other sources of H₂ can be used in part or in full. For example, in some embodiments, at least part (e.g., at least 25%, at least 50%, or at least 75%) of the H₂ of the first feed stream and/or the second feed stream is grey hydrogen, black hydrogen, brown hydrogen, pink hydrogen, turquoise hydrogen, yellow hydrogen, and/or white hydrogen.

The present inventors have noted that electrolysis of water is a desirable way to provide hydrogen to the claimed processes. Accordingly, in some embodiments, the process includes providing at least a portion of H₂ to the first feed stream and/or the second feed stream by electrolysis of water. In some embodiments, the electrolysis of water is performed using at least partially electricity from a renewable source, e.g., to provide so-called "green hydrogen." However, the present inventors have noted that electricity can be generated as part of the claimed process, e.g., using heat exchange from the first or second product stream, or by burning light hydrocarbons as described above. In some embodiments, the electrolysis of water is performed using at least partially electricity generated according to the processes as described herein. For example, in the process 200 of FIG. 3, water 262 separated from the first product stream is electrolyzed in electrolyzer 260, using electricity 264 generated from steam made in the steam generation zone 232 by heat exchange from the first product stream. H₂ generated in the electrolysis is provided via stream 265 to the first feed stream. In some embodiments, at least a portion of O₂ generated in the electrolysis is provided to a partial oxidation reaction zone as described herein and as shown in the embodiment of FIG. 7. Hydrogen from electrolysis can also burned to provide heat energy, e.g., which can be used to heat the first feed stream.

The processes described herein can be operated in a wide variety of reactor systems. In some embodiments, the first reaction zone (i.e., in which the reverse water-gas shift process step is performed) comprises a first reactor in which a reverse water-gas shift catalyst is disposed, and the second reaction zone (i.e., in which the Fischer-Tropsch process step is performed) comprises a second reactor in which the Fischer-Tropsch catalyst is disposed. Examples of such processes are shown schematically in FIGS. 1, 2, and 4. In these examples, the process (100, 200, 400) is performed in a reactor system that includes a first reactor (110, 210, 410) in which a reverse water-gas shift catalyst (113, 213, 413) is disposed, and a second reactor (120, 220, 420) in which the Fischer-Tropsch catalyst (123, 223, 423) is disposed. The reactors used for the integrated process of the present disclosure as described herein are not particularly limited, and the person of ordinary skill in the art will be able to select an appropriate reactor.

But other embodiments are possible. For example, in some embodiments, the process is performed in a reactor system comprising first catalyst bed in which the reverse water-gas shift catalyst is disposed, and wherein the second reaction zone comprises a second catalyst bed in which the Fischer-Tropsch catalyst is disposed. In some embodiments, the first reactor bed and the second reactor bed are disposed within the same reactor. Such a configuration is shown in FIG. 4, in which the reverse water-gas shift catalyst 313 is disposed in a first catalyst bed 314, and the Fischer-Tropsch catalyst 323 is disposed in a second catalyst bed 324. Here, the catalyst beds 314 and 324 are in the same reactor 305, with process gases flowing between them. Such a configuration can be especially desirable when the first temperature and the second temperature are relatively close to one another.

In various embodiments, the process is performed in a reactor system comprising one or more first catalyst containers in which the reverse water-gas shift catalyst is disposed, and wherein the second reaction zone comprises one or more second catalyst containers in which the Fischer-Tropsch catalyst is disposed. These can be provided in the same reactor, such as described above with respect to catalyst beds.

As noted above, the reverse water-gas shift process step using the palladium and platinum catalysts described herein and the Fischer-Tropsch process step can be performed under similar conditions. Accordingly, in various embodiments, the reverse water-gas shift catalyst and the Fischer-Tropsch catalyst can be provided together in the same catalyst bed, e.g., mixed together. Such an embodiment is shown in FIG. 6. Here, the process 500 is performed in a reactor system that includes a reactor 505 in which the reverse water-gas shift catalyst 513 and the Fischer-Tropsch catalyst 523 are mixed together in a single catalyst bed 524. Here, first feed stream 511 and second product stream 522 can be substantially as described herein. The first product stream and the second feed stream are understood to be the mixture of process gases within the mixed catalysts.

In the embodiments particularly-described above, separate rWGS and Fischer-Tropsch catalysts are used, e.g., in separate reactors, in separate regions of the same reactor, or even comingled in the same region of a reactor.

However, the present inventors also note that there are certain commonalities between the rWGS catalysts described herein and certain Fischer-Tropsch catalysts. For example, as the person of ordinary skill in the art would appreciate, manganese is a common modifier used in Fischer-Tropsch catalysts, especially those based on cobalt. The present inventors also note that similar supports can be used for each.

Accordingly, in addition to the configurations described above, the present inventors contemplate the provision of a single bifunctional catalyst with both reverse water-gas shift activity and Fischer-Tropsch activity. Such a bifunctional catalyst includes both rWGS-active catalyst metal and the Fischer-Tropsch active catalyst metal in the same body. The person or ordinary skill in the art will appreciate that both the rWGS catalysts and the Fischer-Tropsch catalysts are supported catalyst, e.g., metal oxide supported catalyst. As such, in various embodiments of the present disclosure, the rWGS-active catalyst metals and Fischer-Tropsch active catalyst metals can be provided together on the same support to provide a bifunctional catalyst. For example, in some embodiments, the supports of bifunctional catalyst are provided themselves as discrete body of material, e.g., as porous particles, pellets, or shaped extrudates, with the rWGS-active catalyst metals and the FT-active catalyst metals provided thereon to provide a bifunctional catalyst. The rWGS-active catalyst metals and the FT-active catalyst metals may be homogenous distributed throughout the support or may be distributed in discrete areas throughout the support. However, in other embodiments, the bifunctional catalyst of the disclosure can itself be formed as a layer on an underlying substrate. For example, in some embodiments, the bifunctional catalyst is formed from a layer of rWGS-active catalyst metals and a layer of FT-active catalyst metals on an underlying substrate. The rWGS-active catalyst metals and the FT-active catalyst metals may be homogeneously distributed on the underlying substrate. In other embodiments, the rWGS-active catalyst metals and the FT-active catalyst metals may be in discrete areas on the underlying substrate. The underlying substrate is not particularly limited. It can be formed of, e.g., a metal or metal oxide, and can itself be provided in a number of forms, such as particles, pellets, shaped extrudates, or monoliths.

The bifunctional catalyst includes a support material, the rWGS-active catalyst metals as described herein, and the Fischer-Tropsch active catalyst metals as described herein. For example, the bifunctional catalyst includes a support that is a metal oxide support as described herein, at least one of platinum, palladium, gold, and metal as described herein, and at least one of cobalt, iron, rhodium, and ruthenium. In some embodiments of present disclosure, the bifunctional catalyst includes a support that is a metal oxide support as described herein, at least one of platinum, palladium, gold, metal as described herein, and cobalt. In some embodiments of the present disclosure, the bifunctional catalyst includes a support comprising at least one of titanium oxide, zirconium oxide, cerium oxide, or aluminum oxide, at least one of platinum, palladium, gold, and nickel, metals as described herein, and cobalt. In some embodiments, the bifunctional catalyst includes a titanium oxide support, at least one of platinum, palladium, gold, and nickel, metal as described herein, and cobalt. In some embodiments, the bifunctional catalyst includes a titanium oxide support, platinum, metal as described herein, and cobalt. In some embodiments, the bifunctional catalyst includes a titanium oxide support, palladium, metals as described herein, and cobalt. In some embodiments, the bifunctional catalyst includes a titanium oxide support, gold, metals as described herein, and cobalt. For example, in some embodiments, the bifunctional catalyst includes a titanium oxide support, at least one of platinum, palladium, gold, and nickel, present in an amount in the range of 0.05 to 10 wt%, metal as described herein, present in an amount in the range of 0.5 to 20 wt%, and cobalt, present in an amount in the range of 7-25 wt%. In some embodiments, the bifunctional catalyst includes a titanium oxide support, platinum, present in an amount in the range of 0.05 to 10 wt%, metal as described herein, present in an amount in the range of 0.5 to 20 wt%, and cobalt, present in an amount in the range of 7-25 wt%. In some embodiments, the bifunctional catalyst includes a titanium oxide support, palladium, present in an amount in the range of 0.05 to 10 wt%, metal as described herein, present in an amount in the range of 0.5 to 20 wt%, and cobalt, present in an amount in the range of 7-25 wt%. In some embodiments, the bifunctional catalyst includes a titanium oxide support, gold, present in an amount in the range of 0.05 to 10 wt%, metal as described herein, present in an amount in the range of 0.5 to 20 wt%, and cobalt, present in an amount in the range of 7-25 wt%.

The ratio of rWGS-active catalyst metals to FT-active catalyst metals in the bifunctional catalyst is not particularly limited and the person of ordinary skill in the art would be able to select an appropriate ratio. For example, in some embodiments, the ratio of rWGS-active catalyst metals to FT-active catalyst metals in the bifunctional catalyst is at least 0.1:1. In various embodiments, the ratio of rWGS-active catalyst metals to FT-active catalyst metals in the bifunctional catalyst is at least 0.2:1, or 0.5, or 1:1.

Such catalysts can be used in embodiments like those described with respect to FIG. 6. The person of ordinary skill in the art will select reaction conditions that provide the appropriate balance of reverse water-gas shift activity and Fischer-Tropsch activity.

FIG. 7 is a schematic depiction of another integrated process according to the disclosure. Here, the reverse water-gas shift and Fischer-Tropsch process steps are integrated together with partial oxidation of light hydrocarbons to provide CO and H₂ to the Fischer-Tropsch process step; electrolysis to provide H₂ for the reverse water-gas shift process step and O₂ for the partial oxidation; and various recycles and optional feeds, as described throughout the present specification.

Additional aspects of the disclosure are provided by the following enumerated embodiments, which may be combined in any number and in any combination that is not logically or technically inconsistent.
Embodiment 1. A supported reverse water-gas shift catalyst comprising:
   a support that is a cerium oxide support, a titanium oxide support, an aluminum oxide support, zinc oxide support, a zirconium oxide support, or a mixed oxide support comprising a mixture of two or more of cerium oxide, titanium oxide, aluminum oxide, zinc oxide and zirconium oxide;
   a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
   optionally, at least one of platinum, palladium, gold, and nickel, present in an amount in the range of 0.05 to 10 wt% of the catalyst, based on the total weight of the catalyst.
Embodiment 2. The catalyst of embodiment 1, wherein the support makes up at least 70 wt% (e.g., at least 75 wt%, or 80 wt%, or 85 wt%, or 90 wt%) of the catalyst, on an oxide basis.
Embodiment 3. The catalyst of embodiment 1 or embodiment 2, wherein the support is a cerium oxide support.
Embodiment 4. The catalyst of embodiment 3, wherein at least a surface layer of the cerium oxide support comprises at least 60 wt% cerium oxide, e.g., at least 70 wt% cerium oxide or at least 80 wt% cerium oxide, on an oxide basis.
Embodiment 5. The catalyst of embodiment 3, wherein at least a surface layer of the cerium oxide support comprises at least 90 wt% cerium oxide, e.g., at least 95 wt% cerium oxide, or at least 98 wt% cerium oxide, on an oxide basis.
Embodiment 6. The catalyst of any of embodiments 3-5, wherein the cerium oxide support comprises at least 50 wt% cerium oxide, e.g., at least 60 wt% cerium oxide, or at least 70 wt% cerium oxide, or at least 80 wt% cerium oxide, on an oxide basis.
Embodiment 7. The catalyst of any of embodiments 3-5, wherein the cerium oxide support comprises at least 90 wt% cerium oxide, e.g., at least 95 wt% cerium oxide, or at least 98 wt% cerium oxide, on an oxide basis.
Embodiment 8. The catalyst of embodiment 1 or embodiment 2, wherein the support is a titanium oxide support.
Embodiment 9. The catalyst of embodiment 8, wherein at least a surface layer of the titanium oxide support comprises at least 60 wt% titanium oxide, e.g., at least 70 wt% titanium oxide, or at least 80 wt% titanium oxide, on an oxide basis.
Embodiment 10. The catalyst of embodiment 8, wherein at least a surface layer of the titanium oxide support comprises at least 90 wt% titanium oxide, e.g., at least 95 wt% titanium oxide, or at least 98 wt% titanium oxide, on an oxide basis.
Embodiment 11. The catalyst of any of embodiments 8-10, wherein the titanium oxide support comprises at least 50 wt% titanium oxide, e.g., at least 60 wt% titanium oxide, or at least 70 wt% titanium oxide, or at least 80 wt% titanium oxide, on an oxide basis.
Embodiment 12. The catalyst of any of embodiments 8-10, wherein the titanium oxide support comprises at least 90 wt% titanium oxide, e.g., at least 95 wt% titanium oxide, or at least 98 wt% titanium oxide, on an oxide basis.
Embodiment 14. The catalyst of embodiment 1 or embodiment 2, wherein the support is an aluminum oxide support.
Embodiment 15. The catalyst of embodiment 14, wherein at least a surface layer of the aluminum oxide support comprises at least 60 wt% aluminum oxide, e.g., at least 70 wt% aluminum oxide or at least 80 wt% aluminum oxide, on an oxide basis.
Embodiment 16. The catalyst of embodiment 14, wherein at least a surface layer of the aluminum oxide support comprises at least 90 wt% aluminum oxide, e.g., at least 95 wt% aluminum oxide, or at least 98 wt% aluminum oxide, on an oxide basis.
Embodiment 17. The catalyst of any of embodiments 14-16, wherein the aluminum oxide support comprises at least 50 wt% aluminum oxide, e.g., at least 60 wt% aluminum oxide, or at least 70 wt% aluminum oxide, or at least 80 wt% aluminum oxide, on an oxide basis.
Embodiment 18. The catalyst of any of embodiments 14-16, wherein the aluminum oxide support comprises at least 90 wt% aluminum oxide, e.g., at least 95 wt% aluminum oxide, or at least 98 wt% aluminum oxide, on an oxide basis.
Embodiment 19. The catalyst of embodiment 1 or embodiment 2, wherein the support is a zinc oxide support.
Embodiment 20. The catalyst of embodiment 19, wherein at least a surface layer of the zinc oxide support comprises at least 60 wt% zinc oxide, e.g., at least 70 wt% zirconium oxide or at least 80 wt% zinc oxide, on an oxide basis.
Embodiment 21. The catalyst of embodiment 19, wherein at least a surface layer of the zinc oxide support comprises at least 90 wt% zinc oxide, e.g., at least 95 wt% zinc oxide, or at least 98 wt% zinc oxide, on an oxide basis.
Embodiment 22. The catalyst of any of embodiments 19-21, wherein the zinc oxide support comprises at least 50 wt% zinc oxide, e.g., at least 60 wt% zinc oxide, or at least 70 wt% zinc oxide, or at least 80 wt% zinc oxide, on an oxide basis.
Embodiment 23. The catalyst of any of embodiments 19-22, wherein the zinc oxide support comprises at least 90 wt% zinc oxide, e.g., at least 95 wt% zinc oxide, or at least 98 wt% zinc oxide, on an oxide basis.
Embodiment 24. The catalyst of embodiment 1 or embodiment 2, wherein the support is a zirconium oxide support.
Embodiment 25. The catalyst of embodiment 24, wherein at least a surface layer of the zirconium oxide support comprises at least 60 wt% zirconium oxide, e.g., at least 70 wt% zirconium oxide or at least 80 wt% zirconium oxide, on an oxide basis.
Embodiment 26. The catalyst of embodiment 24, wherein at least a surface layer of the zirconium oxide support comprises at least 90 wt% zirconium oxide, e.g., at least 95 wt% zirconium oxide, or at least 98 wt% zirconium oxide, on an oxide basis.
Embodiment 27. The catalyst of any of embodiments 24-26, wherein the zirconium oxide support comprises at least 50 wt% zirconium oxide, e.g., at least 60 wt% zirconium oxide, or at least 70 wt% zirconium oxide, or at least 80 wt% zirconium oxide, on an oxide basis.
Embodiment 28. The catalyst of any of embodiments 24-27, wherein the zirconium oxide support comprises at least 90 wt% zirconium oxide, e.g., at least 95 wt% zirconium oxide, or at least 98 wt% zirconium oxide, on an oxide basis.
Embodiment 29. The catalyst of embodiment 1 or embodiment 2, wherein the support is a mixed oxide support having at least a surface layer comprising at least 50 wt% of two or more of cerium oxide, titanium oxide, aluminum oxide, zinc oxide, and zirconium oxide, on an oxide basis.
Embodiment 30. The catalyst of any of embodiments 1-29, wherein the support does not include additional metals in a total amount of additional metals in excess of 2 wt%, e.g., in excess of 1 wt% or in excess of 0.5 wt%, on an oxide basis.
Embodiment 31. The catalyst of any of embodiments 1-29, wherein the support includes at least one additional metal.
Embodiment 32. The catalyst of embodiment 31, wherein the total amount of the at least one additional metal is in the range of 0.5-20 wt%, e.g., 1-20 wt%, or 2-20 wt%, or 0.5-15 wt%, or 1-15 wt%, or 2-15 wt%, or 0.5-10 wt%, or 1-10 wt%, or 2-10 wt%, or 0.5-5 wt%, or 1-5 wt%, on an oxide basis.
Embodiment 33. The catalyst of any of embodiments 1-32, wherein the support has a pore volume of at least 0.05 mL/g.
Embodiment 34. The catalyst of any of embodiments 1-33, wherein the support has a pore volume of at most 1.5 mL/g.
Embodiment 35. The catalyst of any of embodiments 1-34, wherein the support has a pore volume in the range of 0.05-1.5 mL/g.
Embodiment 36. The catalyst of any of embodiments 1-35, wherein the metal is manganese.
Embodiment 37. The catalyst of embodiment 36, wherein manganese is present in the catalyst in an amount in the range of 0.5 to 15 wt%, e.g., in the range of 0.5 to 12 wt% or 0.5 to 10 wt%, based on the total weight of the catalyst.
Embodiment 38. The catalyst of embodiment 36, wherein manganese is present in the catalyst in an amount in the range of 1 to 20 wt%, e.g., in the range of 1 to15 wt%, or 1 to 12 wt%, or 1 to 10 wt%, based on the total weight of the catalyst.
Embodiment 39. The catalyst of embodiment 36, wherein manganese is present in the catalyst in an amount in the range of 2 to 20 wt%, e.g., in the range of 2 to15 wt%, or 2 to 12 wt%, or 2 to 10 wt%, based on the total weight of the catalyst.
Embodiment 40. The catalyst of embodiment 36, wherein manganese is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 41. The catalyst of any of embodiments 1-35, wherein the metal is copper.
Embodiment 42. The catalyst of embodiment 41, wherein copper is present in the catalyst in an amount in the range of 0.5 to 15 wt%, e.g., in the range of 0.5 to 12 wt% or 0.5 to 10 wt%, based on the total weight of the catalyst.
Embodiment 43. The catalyst of embodiment 41, wherein copper is present in the catalyst in an amount in the range of 1 to 20 wt%, e.g., in the range of 1 to15 wt%, or 1 to 12 wt%, or 1 to 10 wt%, based on the total weight of the catalyst.
Embodiment 44. The catalyst of embodiment 41, wherein copper is present in the catalyst in an amount in the range of 2 to 20 wt%, e.g., in the range of 2 to15 wt%, or 2 to 12 wt%, or 2 to 10 wt%, based on the total weight of the catalyst.
Embodiment 45. The catalyst of embodiment 41, wherein copper is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 46. The catalyst of any of embodiments 1-35, wherein the metal is gallium.
Embodiment 47. The catalyst of embodiment 46, wherein gallium is present in the catalyst in an amount in the range of 0.5 to 15 wt%, e.g., in the range of 0.5 to 12 wt% or 0.5 to 10 wt%, based on the total weight of the catalyst.
Embodiment 48. The catalyst of embodiment 46, wherein gallium is present in the catalyst in an amount in the range of 1 to 20 wt%, e.g., in the range of 1 to15 wt%, or 1 to 12 wt%, or 1 to 10 wt%, based on the total weight of the catalyst.
Embodiment 49. The catalyst of embodiment 46, wherein gallium is present in the catalyst in an amount in the range of 2 to 20 wt%, e.g., in the range of 2 to15 wt%, or 2 to 12 wt%, or 2 to 10 wt%, based on the total weight of the catalyst.
Embodiment 50. The catalyst of embodiment 46, wherein gallium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 51. The catalyst of any of embodiments 1-35, wherein the is indium.
Embodiment 52. The catalyst of embodiment 51, wherein indium is present in the catalyst in an amount in the range of 0.5 to 15 wt%, e.g., in the range of 0.5 to 12 wt% or 0.5 to 10 wt%, based on the total weight of the catalyst.
Embodiment 53. The catalyst of embodiment 51, wherein indium is present in the catalyst in an amount in the range of 1 to 20 wt%, e.g., in the range of 1 to15 wt%, or 1 to 12 wt%, or 1 to 10 wt%, based on the total weight of the catalyst.
Embodiment 54. The catalyst of embodiment 51, wherein indium is present in the catalyst in an amount in the range of 2 to 20 wt%, e.g., in the range of 2 to15 wt%, or 2 to 12 wt%, or 2 to 10 wt%, based on the total weight of the catalyst.
Embodiment 55. The catalyst of embodiment 51, wherein indium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 56. The catalyst of any of embodiments 1-35, wherein the metal is lanthanum.
Embodiment 57. The catalyst of embodiment 56, wherein lanthanum is present in the catalyst in an amount in the range of 0.5 to 15 wt%, e.g., in the range of 0.5 to 12 wt% or 0.5 to 10 wt%, based on the total weight of the catalyst.
Embodiment 58. The catalyst of embodiment 56, wherein lanthanum is present in the catalyst in an amount in the range of 1 to 20 wt%, e.g., in the range of 1 to15 wt%, or 1 to 12 wt%, or 1 to 10 wt%, based on the total weight of the catalyst.
Embodiment 59. The catalyst of embodiment 56, wherein lanthanum is present in the catalyst in an amount in the range of 2 to 20 wt%, e.g., in the range of 2 to15 wt%, or 2 to 12 wt%, or 2 to 10 wt%, based on the total weight of the catalyst.
Embodiment 60. The catalyst of embodiment 56, wherein lanthanum is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 61. The catalyst of any of embodiments 1-35, wherein the metal is titanium.
Embodiment 62. The catalyst of embodiment 61, wherein titanium is present in the catalyst in an amount in the range of 0.5 to 15 wt%, e.g., in the range of 0.5 to 12 wt% or 0.5 to 10 wt%, based on the total weight of the catalyst.
Embodiment 63. The catalyst of embodiment 61, wherein titanium is present in the catalyst in an amount in the range of 1 to 20 wt%, e.g., in the range of 1 to 15 wt%, or 1 to 12 wt%, or 1 to 10 wt%, based on the total weight of the catalyst.
Embodiment 64. The catalyst of embodiment 61, wherein titanium is present in the catalyst in an amount in the range of 2 to 20 wt%, e.g., in the range of 2 to 15 wt%, or 2 to 12 wt%, or 2 to 10 wt%, based on the total weight of the catalyst.
Embodiment 65. The catalyst of embodiment 61, wherein titanium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 66. The catalyst of any of embodiments 1-35, wherein the metal is niobium.
Embodiment 67. The catalyst of embodiment 66, wherein niobium is present in the catalyst in an amount in the range of 0.5 to 15 wt%, e.g., in the range of 0.5 to 12 wt% or 0.5 to 10 wt%, based on the total weight of the catalyst.
Embodiment 68. The catalyst of embodiment 66, wherein niobium is present in the catalyst in an amount in the range of 1 to 20 wt%, e.g., in the range of 1 to15 wt%, or 1 to 12 wt%, or 1 to 10 wt%, based on the total weight of the catalyst.
Embodiment 69. The catalyst of embodiment 66, wherein niobium is present in the catalyst in an amount in the range of 2 to 20 wt%, e.g., in the range of 2 to15 wt%, or 2 to 12 wt%, or 2 to 10 wt%, based on the total weight of the catalyst.
Embodiment 70. The catalyst of embodiment 66, wherein niobium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 71. The catalyst of any of embodiments 1-35, wherein the metal is vanadium.
Embodiment 72. The catalyst of embodiment 71, wherein vanadium is present in the catalyst in an amount in the range of 0.5 to 15 wt%, e.g., in the range of 0.5 to 12 wt% or 0.5 to 10 wt%, based on the total weight of the catalyst.
Embodiment 73. The catalyst of embodiment 71, wherein vanadium is present in the catalyst in an amount in the range of 1 to 20 wt%, e.g., in the range of 1 to15 wt%, or 1 to 12 wt%, or 1 to 10 wt%, based on the total weight of the catalyst.
Embodiment 74. The catalyst of embodiment 71, wherein vanadium is present in the catalyst in an amount in the range of 2 to 20 wt%, e.g., in the range of 2 to15 wt%, or 2 to 12 wt%, or 2 to 10 wt%, based on the total weight of the catalyst.
Embodiment 75. The catalyst of embodiment 71, wherein vanadium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 76. The catalyst of any of embodiments 1-35, wherein the metal is zirconium.
Embodiment 77. The catalyst of embodiment 76, wherein zirconium is present in the catalyst in an amount in the range of 0.5 to 15 wt%, e.g., in the range of 0.5 to 12 wt% or 0.5 to 10 wt%, based on the total weight of the catalyst.
Embodiment 78. The catalyst of embodiment 76, wherein zirconium is present in the catalyst in an amount in the range of 1 to 20 wt%, e.g., in the range of 1 to15 wt%, or 1 to 12 wt%, or 1 to 10 wt%, based on the total weight of the catalyst.
Embodiment 79. The catalyst of embodiment 76, wherein zirconium is present in the catalyst in an amount in the range of 2 to 20 wt%, e.g., in the range of 2 to15 wt%, or 2 to 12 wt%, or 2 to 10 wt%, based on the total weight of the catalyst.
Embodiment 80. The catalyst of embodiment 76, wherein zirconium is present in the catalyst in an amount in the range of 4 to 20 wt%, e.g., in the range of 4 to 15 wt%, or 4 to 12 wt%, or 4 to 10 wt%, based on the total weight of the catalyst.
Embodiment 81. The catalyst of any of embodiments 1-80, wherein the total amount of cerium, titanium, aluminum, zirconium, metal (e.g., manganese, gallium, indium, lanthanum, titanium, niobium, vanadium, and zirconium), in the catalyst is at least 90 wt%, e.g., at least 95 wt% or at least 98 wt% of the catalyst, on a metallic basis.
Embodiment 82. The catalyst of any of embodiments 1-81, wherein platinum, palladium, gold, or nickel is present in the catalyst.
Embodiment 83. A supported reverse water-gas shift catalyst comprising:
   a support that is a cerium oxide support, a titanium oxide support, a zirconium oxide support, or a mixed oxide support comprising a mixture of two or more of cerium oxide, titanium oxide, aluminum oxide, zinc oxide, and zirconium oxide;
   a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
   at least one of platinum, palladium, gold, and nickel present in an amount in the range of 0.05 to 10 wt% of the catalyst, based on the total weight of the catalyst.
Embodiment 84. The catalyst of embodiment 83, wherein the support is as described in any of embodiments 2-35.
Embodiment 85. The catalyst of embodiment 83 or embodiment 84, wherein the metal is manganese and is present in the amounts as described in embodiments 36-40.
Embodiment 86. The catalyst of embodiment 83 or embodiment 84, wherein the metal is copper and is present in the amounts as described in embodiments 41-45.
Embodiment 87. The catalyst of embodiment 83 or embodiment 84, wherein the metal is gallium and is present in the amounts as described in embodiments 46-50.
Embodiment 88. The catalyst of embodiment 83 or embodiment 84, wherein the metal is indium and is present in the amounts as described in embodiments 51-55.
Embodiment 89. The catalyst of embodiment 83 or embodiment 84, wherein the metal is lanthanum and is present in the amounts as described in embodiments 56-60. Embodiment 90. The catalyst of embodiment 83 or embodiment 84, wherein the metal is titanium and is present in the amounts as described in embodiments 61-65.
Embodiment 91. The catalyst of embodiment 83 or embodiment 84, wherein the metal is niobium and is present in the amounts as described in embodiments 66-70.
Embodiment 92. The catalyst of embodiment 83 or embodiment 84, wherein the metal is vanadium and is present in the amounts as described in embodiments 71-75.
Embodiment 93. The catalyst of embodiment 83 or embodiment 84, wherein the metal is zirconium and is present in the amounts as described in embodiments 76-80.
Embodiment 94. The catalyst of any of embodiments 83-93, wherein platinum is present in the catalyst.
Embodiment 95. The catalyst of embodiment 94, wherein platinum is present in the catalyst in an amount in the range of 0.1 to 10 wt%, e.g., in the range of 0.5 to 10 wt%, or 1 to 10 wt%, or 2 to 10 wt%, or 5 to 10 wt%, based on the total weight of the catalyst.
Embodiment 96. The catalyst of embodiment 94, wherein platinum is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst.
Embodiment 97. The catalyst of embodiment 94, wherein platinum is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst.
Embodiment 98. The catalyst of embodiment 94, wherein platinum is present in the catalyst in an amount in a range of 0.05 to 2 wt%, e.g., in the range of 0.1 to 2 wt%, or 0.3 to 2 wt%, or 0.5 to 2 wt%, or 1 to 2 wt%, based on the total weight of the catalyst.
Embodiment 99. The catalyst of embodiment 94, wherein platinum is present in the catalyst in an amount in a range of 0.05 to 1.5 wt%, e.g., in the range of 0.1 to 1.5 wt%, or 0.3 to 1.5 wt%, or 0.5 to 1.5 wt%, based on the total weight of the catalyst.
Embodiment 100. The catalyst of embodiment 94, wherein platinum is present in the catalyst in an amount in the range of 0.05 to 1 wt%, e.g., in the range of 0.1 to 1 wt%, or 0.3 to 1 wt%, or 0.5 to 1 wt%, based on the total weight of the catalyst.
Embodiment 101. The catalyst of embodiment 94, wherein platinum is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.
Embodiment 102. The catalyst of any of embodiments 83-93, wherein palladium is present in the catalyst.
Embodiment 103. The catalyst of embodiment 102, wherein palladium is present in the catalyst in an amount in the range of 0.1 to 10 wt%, e.g., in the range of 0.5 to 10 wt%, or 1 to 10 wt%, or 2 to 10 wt%, or 5 to 10 wt%, based on the total weight of the catalyst.
Embodiment 104. The catalyst of embodiment 102, wherein palladium is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst.
Embodiment 105. The catalyst of embodiment 102, wherein palladium is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst.
Embodiment 106. The catalyst of embodiment 102, wherein palladium is present in the catalyst in an amount in a range of 0.05 to 2 wt%, e.g., in the range of 0.1 to 2 wt%, or 0.3 to 2 wt%, or 0.5 to 2 wt%, based on the total weight of the catalyst.
Embodiment 107. The catalyst of embodiment 102, wherein palladium is present in the catalyst in an amount in a range of 0.05 to 1.5 wt%, e.g., in the range of 0.1 to 1.5 wt%, or 0.3 to 1.5 wt%, or 0.5 to 1.5 wt%, based on the total weight of the catalyst.
Embodiment 108. The catalyst of embodiment 102, wherein palladium is present in the catalyst in an amount in the range of 0.05 to 1 wt%, e.g., in the range of 0.1 to 1 wt%, or 0.3 to 1 wt%, or 0.5 to 1 wt%, based on the total weight of the catalyst.
Embodiment 109. The catalyst of embodiment 102, wherein palladium is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.
Embodiment 110. The catalyst of any of embodiments 82-93, wherein gold is present in the catalyst.
Embodiment 111. The catalyst of embodiment 110, wherein gold is present in the catalyst in an amount in the range of 0.1 to 10 wt%, e.g., in the range of 0.5 to 10 wt%, or 1 to 10 wt%, or 2 to 10 wt%, or 5 to 10 wt%, based on the total weight of the catalyst.
Embodiment 112. The catalyst of embodiment 110, wherein gold is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst.
Embodiment 113. The catalyst of embodiment 110, wherein gold is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst.
Embodiment 114. The catalyst of embodiment 110, wherein gold is present in the catalyst in an amount in a range of 0.05 to 2 wt%, e.g., in the range of 0.1 to 2 wt%, or 0.3 to 2 wt%, or 0.5 to 2 wt%, based on the total weight of the catalyst.
Embodiment 115. The catalyst of embodiment 110, wherein gold is present in the catalyst in an amount in a range of 0.05 to 1.5 wt%, e.g., in the range of 0.1 to 1.5 wt%, or 0.3 to 1.5 wt%, or 0.5 to 1.5 wt%, based on the total weight of the catalyst.
Embodiment 116. The catalyst of embodiment 110, wherein gold is present in the catalyst in an amount in the range of 0.05 to 1 wt%, e.g., in the range of 0.1 to 1 wt%, or 0.3 to 1 wt%, or 0.5 to 1 wt%, based on the total weight of the catalyst.
Embodiment 117. The catalyst of embodiment 110, wherein gold is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.
Embodiment 118. The catalyst of any of embodiments 82-93, wherein nickel is present in the catalyst.
Embodiment 119. The catalyst of embodiment 118, wherein nickel is present in the catalyst in an amount in the range of 0.1 to 10 wt%, e.g., in the range of 0.5 to 10 wt%, or 1 to 10 wt%, or 2 to 10 wt%, or 5 to 10 wt%, based on the total weight of the catalyst.
Embodiment 120. The catalyst of embodiment 118, wherein nickel is present in the catalyst in an amount in the range of 0.05 to 7 wt%, e.g., in the range of 0.1 to 7 wt%, or 0.5 to 7 wt%, or 1 to 7 wt%, or 2 to 7 wt%, based on the total weight of the catalyst.
Embodiment 121. The catalyst of embodiment 118, wherein nickel is present in the catalyst in an amount in the range of 0.05 to 5 wt%, e.g., in the range of 0.1 to 5 wt%, or 0.5 to 5 wt%, or 1 to 5 wt%, or 2 to 5 wt%, based on the total weight of the catalyst.
Embodiment 122. The catalyst of embodiment 118, wherein nickel is present in the catalyst in an amount in a range of 0.05 to 2 wt%, e.g., in the range of 0.1 to 2 wt%, or 0.3 to 2 wt%, or 0.5 to 2 wt%, based on the total weight of the catalyst.
Embodiment 123. The catalyst of embodiment 118, wherein nickel is present in the catalyst in an amount in a range of 0.05 to 1.5 wt%, e.g., in the range of 0.1 to 1.5 wt%, or 0.3 to 1.5 wt%, or 0.5 to 1.5 wt%, based on the total weight of the catalyst.
Embodiment 124. The catalyst of embodiment 118, wherein nickel is present in the catalyst in an amount in the range of 0.05 to 1 wt%, e.g., in the range of 0.1 to 1 wt%, or 0.3 to 1 wt%, or 0.5 to 1 wt%, based on the total weight of the catalyst.
Embodiment 125. The catalyst of embodiment 118, wherein nickel is present in the catalyst in an amount in the range of 0.05 to 0.8 wt%, e.g., in the range of 0.1 to 0.8 wt%, or 0.3 to 0.8 wt%, or 0.5 to 0.8 wt%, based on the total weight of the catalyst.
Embodiment 126. The catalyst of any of embodiments 83-125, wherein a weight ratio of platinum, palladium, gold, and/or nickel to the metal (e.g., manganese, gallium, indium, lanthanum, titanium, niobium, vanadium, and zirconium) is at least 0.05:1, e.g., at least 0.1:1.
Embodiment 127. The catalyst of any of embodiments 83-126, wherein a weight ratio of platinum, palladium, gold, and/or nickel to the metal (e.g., manganese, gallium, indium, lanthanum, titanium, niobium, vanadium, and zirconium) is at most 5:1, e.g., at most 2:1, or 1:1, or 0.5:1.
Embodiment 128. The catalyst of any of embodiments 83-127, wherein a ratio of platinum, palladium, gold, and/or nickel to the metal (e.g., manganese, gallium, indium, lanthanum, titanium, niobium, vanadium, and zirconium) is in the range of 0.05:1 to 1:1 (e.g., in the range of 0.05:1 to 2:1, or 0.05:1 to 1:1, or 0.05:1 to 0.5:1, or 0.05:1 to 0.3:1, or 0.07:1 to 5:1, or 0.07:1 to 2:1, or 0.07:1 to 1:1, or 0.07:1 to 0.5:1, or 0.07:1 to 0.3:1, or 0.1:1 to 5:1, or 0.1:1 to 2:1, or 0.1:1 to 1:1, or 0.1:1 to 0.5:1, or 0.1:1 to 0.3:1).
Embodiment 129. The catalyst of any of embodiments 83-128, wherein the total amount of cerium, titanium, zinc, zirconium, metal (e.g., manganese, copper, gallium, indium, lanthanum, titanium, niobium, vanadium, and zirconium), platinum, palladium, gold, and nickel in the catalyst is at least 90 wt%, e.g., at least 95 wt% or at least 98 wt% of the catalyst, on a metallic basis.
Embodiment 130. A method for making the catalyst of any of embodiments 1-129, the method comprising:
   providing a support that is a cerium oxide support, a titanium oxide support, an aluminum oxides support, a zinc oxide support, a zirconium oxide support, or a mixed oxide support comprising a mixture of two or more of cerium oxide, titanium oxide, aluminum oxide, zinc oxide, and zirconium oxide;
   contacting the support with one or more liquids each comprising one or more metalcontaining compounds dispersed in a solvent(s), wherein the metal is selected from manganese, copper, gallium, indium, lanthanum, titanium, niobium, vanadium, and zirconium, and optionally one or more platinum-, palladium-, gold-, or nickel- containing compounds;
   allowing the solvent(s) to evaporate to provide a catalyst precursor; and calcining the catalyst precursor.
Embodiment 131. The method of embodiment 130, wherein contacting the support with the liquid comprises adding the liquid in an amount equal to the pore volume of the support.
Embodiment 132. The method of embodiment 130, wherein contacting the support with the liquid comprises adding the liquid in an amount greater than the pore volume of the support.
Embodiment 133. The method of any of embodiments 130-132, wherein ratio of the amount liquid to the amount of support on a mass basis is in the range of 1:1 to 5:1 (e.g., in the range of 1:1 to 3:1).
Embodiment 134. The method of any of embodiments 130-133, wherein contacting the support with the liquid provides a slurry.
Embodiment 135. The method of any of embodiments 130-134, wherein allowing the solvent to evaporate is conducted at ambient temperature.
Embodiment 136. The method of embodiments 130-135, wherein allowing the solvent to evaporate is conducted at an elevated temperature (e.g., in the range of 50-150 °C) for a drying time (e.g., 24 hours).
Embodiment 137. The method of embodiments 130-135, wherein allowing the solvent to evaporate is conducted under vacuum and at an elevated temperature (e.g., in the range of 50-150 °C) for a drying time (e.g., 24 hours).
Embodiment 138. The method of any of embodiments 130-135, wherein allowing the solvent to evaporate is conducted in a stirring drybath at an elevated temperature (e.g., in the range of 30-100 °C).
Embodiment 139. The method of any of embodiments 130-138, wherein calcining the catalyst precursor is conducted for a calcining time in the range of 0.5 to 24 hours (e.g., 0.5 to 15 hours, or 0.5 to 10 hours, or 0.5 to 5 hours).
Embodiment 140. The method of any of embodiments 130-139, wherein calcining the catalyst precursor is conducted for a calcining is in the range of 100-600 °C (e.g., in the range of 120-500 °C).
Embodiment 141. The catalyst of any of embodiments 1-129, made by a method according to embodiments 130-140.
Embodiment 142. A method for performing a reverse water-gas shift reaction, the method comprising:
   contacting at a temperature in the range of 100-1100 °C a catalyst according to any of embodiments 1-104 and 116 with a feed stream comprising CO₂ and H₂,wherein at least part of the CO₂ of the first feed stream is from biogas, a CO₂ emission source, and/or direct air capture, to provide a product stream comprising CO and H₂, the product stream having a lower concentration of CO₂ and a higher concentration of CO than the feed stream.
Embodiment 143. The method of embodiment 142, wherein the reverse water-gas shift reaction has a CO selectivity of at least 50%, e.g., of at least 60%.
Embodiment 144. The method of embodiment 142, wherein the reverse water-gas shift reaction has a CO selectivity of at least 70%, e.g., of at least 80%.
Embodiment 145. The method of embodiment 142, wherein the reverse water-gas shift reaction has a CO selectivity of at least 85%, e.g., of at least 95%.
Embodiment 146. The method of embodiment 142, wherein the reverse water-gas shift reaction has a CO selectivity of at least 85%, e.g., of at least 96%.
Embodiment 147. The method of embodiment 142, wherein the reverse water-gas shift reaction has a CO selectivity of 50-99 wt%, e.g., 60-99%, or 70-99%, or 80-99%, or 90-99%, or 95-99%.
Embodiment 148. The method of embodiment 142, wherein the reverse water-gas shift reaction has a CO selectivity of 50-90%, e.g., 60-90%, or 70-90%, or 50-80%, or 60-80%, or 50-70%.
Embodiment 149. The method of any of embodiments 142-148, wherein the reverse water-gas shift reaction has a methane selectivity of no more than 40%, e.g., no more than 35%, or 30%, or 25%, or 20%.
Embodiment 150. The method of any of embodiments 142-148, wherein the reverse water-gas shift reaction has a methane selectivity of no more than 15%, e.g., no more than 12%, or 10%, or 8%.
Embodiment 151. The method of any of embodiments 142-148, wherein the reverse water-gas shift reaction has a methane selectivity of no more than 5%, e.g., no more than 4%.
Embodiment 152. The method of any of embodiments 142-148, wherein the reverse water-gas shift reaction has a methane selectivity of no more than 2%, e.g., no more than 1%.
Embodiment 153. The method of any of embodiments 142-148, wherein the reverse water-gas shift reaction has a methane selectivity of no more than 0.5%, e.g., no more than 0.2%.
Embodiment 154. The method of any of embodiments 142-153, having a CO₂ conversion of at least 5%, e.g., at least 10%, or 20%.
Embodiment 155. The method of any of embodiments 142-153, having a CO₂ conversion of at least 30%, e.g., at least 40%.
Embodiment 156. The method of any of embodiments 142-155, having a CO₂ conversion of no more than 90%, e.g., no more than 80%, or no more than 70%.
Embodiment 157. The method of any of embodiments 142-156, having a CO₂ conversion of no more than 65%, e.g., no more than 60%.
Embodiment 158. The method of any of embodiments 142-157, conducted at a temperature in the range of 250-1050 °C, e.g., in the range of 250-1000 °C, or 250-950 °C.
Embodiment 159. The method of any of embodiments 142-157, conducted at a temperature in the range of 250-900 °C, e.g., in the range of 250-850 °C , or 250-800 °C, or 250-750 °C, or 250-700 °C, or 250-650 °C, or 250-600 °C.
Embodiment 160. The method of any of embodiments 142-157, conducted at a temperature in the range of 300-1100 °C, e.g., in the range of 300-1050 °C, or 300-1000 °C, or 300-950 °C.
Embodiment 161. The method of any of embodiments 142-157, conducted at a temperature in the range of 300-900 °C, e.g., in the range of 300-850 °C, or 300-800 °C, or 300-750 °C, or 300-700 °C, or 300-650 °C, or 300-600 °C.
Embodiment 162. The method of any of embodiments 142-157, conducted at a temperature in the range of 350-1100 °C, e.g., in the range of 350-1050 °C, or 350-1000 °C , or 350-950 °C.
Embodiment 163. The method of any of embodiments 142-157, conducted at a temperature in the range of 350-900 °C, e.g., in the range of 350-850 °C, or 350-800 °C , or 350-750 °C, or 350-700 °C, or 350-650 °C, or 350-600 °C.
Embodiment 164. The method of any of embodiments 142-157, conducted at a temperature in the range of 400-1100 °C, e.g., in the range of 400-1050 °C, or 400-1000 °C , or 400-950 °C.
Embodiment 165. The method of any of embodiments 142-157, conducted at a temperature in the range of 400-900 °C, e.g., in the range of 400-850 °C, or 400-800 °C , or 400-750 °C, or 400-700 °C, or 400-650 °C, or 400-600 °C.
Embodiment 166. The method of any of embodiments 142-157, conducted at a temperature in the range of 450-1100 °C, e.g., in the range of 450-1050 °C, or 450-1000 °C, or 450-950 °C.
Embodiment 167. The method of any of embodiments 142-157, conducted at a temperature in the range of 450-900 °C, e.g., in the range of 450-850 °C, or 450-800 °C, or 450-750 °C, or 450-700 °C, or 450-650 °C, or 450-600 °C.
Embodiment 168. The method of any of embodiments 142-157, conducted at a temperature in the range of 500-1100 °C, e.g., in the range of 500-1050 °C, or 500-1000 °C, or 500-950 °C.
Embodiment 169. The method of any of embodiments 142-157, conducted at a temperature in the range of 500-900 °C, e.g., in the range of 500-850 °C, or 500-800 °C, or 500-750 °C , or 500-700 °C, or 500-650 °C, or 500-600 °C.
Embodiment 170. The method of any of embodiments 142-157, conducted at a temperature in the range of 550-1100 °C, e.g., in the range of 550-1050 °C, or 550-1000 °C, or 550-950°C.
Embodiment 171. The method of any of embodiments 142-157, conducted at a temperature in the range of 550-900 °C, e.g., in the range of 550-850 °C, or 550-800 °C, or 550-750°C, or 550-700 °C, or 550-650 °C, or 550-600 °C.
Embodiment 172. The method of any of embodiments 142-157, conducted at a temperature in the range of 600-1100 °C, e.g., in the range of 600-1050 °C, or 600-1000 °C, or 600-950°C.
Embodiment 173. The method of any of embodiments 142-157, conducted at a temperature in the range of 600-900 °C, e.g., in the range of 600-850 °C, or 600-800 °C, or 600-750°C, or 600-700 °C, or 600-650 °C.
Embodiment 174. The method of any of embodiments 142-157, conducted at a temperature in the range of 650-1100 °C, e.g., in the range of 650-1050 °C, or 650-1000 °C, or 650-950°C.
Embodiment 175. The method of any of embodiments 142-157, conducted at a temperature in the range of 650-900 °C, e.g., in the range of 650-850 °C, or 650-800 °C, or 650-750°C, or 650-700 °C.
Embodiment 176. The method of any of embodiments 142-157, conducted at a temperature in the range of 700-1100 °C, e.g., in the range of 700-1050 °C, or 700-1000 °C, or 700-950°C.
Embodiment 177. The method of any of embodiments 142-157, conducted at a temperature in the range of 700-900 °C, e.g., in the range of 700-850 °C, or 700-800 °C, or 700-750°C.
Embodiment 178. The method of any of embodiments 142-177, wherein at least part of the H₂ of the feed stream is from a renewable source.
Embodiment 179. The method of any of embodiments 142-178, wherein at least part of the H₂ of the feed stream is green hydrogen.
Embodiment 180. The method of any of embodiments 142-179, wherein at least part of the H₂ of the feed stream is blue hydrogen.
Embodiment 181. The method of any of embodiments 142-180, wherein at least a part of the H₂ of the feed stream is grey hydrogen, black hydrogen, brown hydrogen, pink hydrogen, turquoise hydrogen, yellow hydrogen, and/or white hydrogen.
Embodiment 182. The process of embodiment 142-180, wherein the CO₂ of the first feed stream comprises at least 50 vol% (e.g., at least 75 vol%, at least 90 vol%, or at least 95 vol%) CO₂ from biogas, a CO₂ emission source, and/or CO₂ from direct air capture.
Embodiment 183. The process of claim 142-180, wherein at least part of the CO₂ of the first feed stream is from biogas.
Embodiment 184. The process of embodiment 183, wherein the CO₂ of the first feed stream comprises at least 50 vol% (e.g., at least 75 vol%, at least 90 vol%, or at least 95 vol%) CO₂ from biogas.
Embodiment 185. The process of claim 142-180, wherein at least part of the CO₂ of the first feed stream is from direct air capture.
Embodiment 186. The process of embodiment 185, wherein the CO₂ of the first feed stream comprises at least 50 vol% (e.g., at least 75 vol%, at least 90 vol%, or at least 95 vol%) CO₂ from direct air capture.
Embodiment 187. The process of embodiment 142-180, wherein at least part of the CO₂ of the first feed stream is from a CO₂ emission source (e.g., from a manufacturing plant, e.g., a bioethanol plant, a steel plant, or a cement plant).
Embodiment 188. The process of embodiment 187, wherein the CO₂ of the first feed stream comprises at least 50 vol% (e.g., at least 75 vol%, at least 90 vol%, or at least 95 vol%) CO₂ from a CO₂ emission source.
Embodiment 189. The method of any of embodiments 142-188, wherein the molar ratio of H₂ to CO₂ in the feed stream is at least 0.1:1, e.g., at least 0.5:1.
Embodiment 190. The method of any of embodiments 142-189, wherein the molar ratio of H₂ to CO₂ in the feed stream is at least 0.9:1, e.g., at least 1:1 or at least 1.5:1.
Embodiment 191. The method of any of embodiments 142-189, wherein the molar ratio of H₂ to CO₂ in the feed stream is at least 2:1, e.g., at least 2.5:1.
Embodiment 192. The method of any of embodiments 142-191, wherein the molar ratio of H₂ to CO₂ in the feed stream is no more than 100:1, e.g., no more than 75:1, or 50:1.
Embodiment 193. The method of any of embodiments 142-191, wherein the molar ratio of H₂ to CO₂ in the feed stream is no more than 20:1, e.g., no more than 15:1, or 10:1.
Embodiment 194. The method of any of embodiments 142-191, wherein the molar ratio of H₂ to CO₂ in the feed stream is in the range of 0.5:1 to 10:1.
Embodiment 195. The method of any of embodiments 142-194, conducted at a pressure in the range of 1 to 100 barg (e.g., in the range of 1 to 70 barg, or 1 to 50 barg, or 1 to 40 barg, or 1 to 35 barg, or 5 to 80 barg, or 5 to 50 barg, or 5 to 40 barg, or 5 to 35 barg, or 10 to 70 barg, 10 to 50 barg, or 10 to 40 barg, or 10 to 35 barg, or 20 to 70 barg, 20 to 50 barg, or 20 to 40 barg, or 20 to 35 barg, or 25 to 70 barg, 25 to 50 barg, or 25 to 40 barg, or 25 to 35 barg).
Embodiment 196. The method of any of embodiments 142-195, conducted at a GHSV in the range of 1,000 to 2,000,000 h⁻¹ (e.g., in the range of 1,000 to 1,200,000 h⁻¹, or 1,000 to 500,000 h⁻¹, or 1,000 to 100,000 h⁻¹, or 5,000 to 1,200,000 h⁻¹, or 5,000 to 500,000 h⁻¹, or 5,000 to 100,000 h⁻¹, or 10,000 to 1,200,000 h⁻¹, or 10,000 to 500,000 h⁻¹, or 10,000 to 100,000 h⁻¹).
Embodiment 197. The method of any of embodiments 142-196, wherein the product stream comprises no more than 95 mol% CO₂ (e.g., no more than 90 mol% CO₂).
Embodiment 198. The method of any of embodiments 142-196, wherein the product stream comprises no more than 85 mol% CO₂ (e.g., no more than 80 mol% CO₂).
Embodiment 199. The method of any of embodiments 142-196, wherein the product stream comprises no more than 75 mol% CO₂ (e.g., no more than 70 mol% CO₂).
Embodiment 200. The method of any of embodiments 142-199, wherein the product stream further comprises CO₂, and wherein the method further comprises recycling at least a portion of the CO₂ of the product stream to the feed stream.
Embodiment 201. The method of any of embodiments 142-200, wherein the product stream further comprises hydrogen and wherein the method further comprises recycling at least a portion of the hydrogen of the product stream to the feed stream.
Embodiment 202. The method of any of embodiments 142-201, wherein a ratio of H₂:CO in the product stream is in the range of 0.1:1 to 100:1. (e.g., in the range of 0.1:1 to 50:1, or 0.1:1 to 25:1, or 0.1:1 to 10:1, or 0.1:1 to 5:1, or 1:1 to 100:1, or 1:1 to 50:1, or 1:1 to 25:1, or 1:1 to 10:1, or 1:1 to 5:1).
Embodiment 203. The method of any of embodiments 142-202, wherein the product stream comprises no more than 20 mol% methane, e.g., no more than 15 mol% methane.
Embodiment 204. The method of any of embodiments 142-202, wherein the product stream comprises no more than 10 mol% methane, e.g., no more than 5 mol%, or 1 mol%, or 0.5 mol%, or 0.1 mol% methane.
Embodiment 205. The method of any of embodiments 142-204, wherein the method comprises activating the catalyst prior to contacting the catalyst with the feed stream.
Embodiment 206. The method of embodiment 205, wherein activating the catalyst comprises contacting the catalyst with a reducing stream comprising a reductive gas (e.g., hydrogen).
Embodiment 207. The method of embodiment 205 or embodiment 206, wherein the reducing stream comprises hydrogen in an amount of at least 25 mol% (e.g., at least 50 mol%, or 75 mol%, or 90 mol%).
Embodiment 208. The method of any of embodiments 205-207, wherein activating the catalyst is conducted at a temperature in the range of 200 to 1000 °C. (e.g., in the range of 250 °C to 1000 °C, or 300 °C to 1000 °C, 200 °C to 900 °C, 250 °C to 900 °C, or 300 °C to 900 °C, 200 °C to 800 °C, or 250 °C to 800 °C, or 300 °C to 800 °C, or 200 °C to 700 °C, or 250 °C to 800 °C, or 300 °C to 700 °C).
Embodiment 209. The method of any of embodiments 207-208, wherein activating the catalyst provides a catalyst that is at least 10% reduced (e.g., at least 25%, or 50%).
Embodiment 210. A process for performing an integrated Fischer-Tropsch process, the process comprising:
   providing a first feed stream comprising H₂ and CO₂, wherein at least part of the CO₂ of the first feed stream is from biogas, a CO₂ emission source, and/or direct air capture;
   contacting at a first temperature in the range of 200-1100 °C and at a first pressure a reverse water-gas shift catalyst with the first feed stream to perform a reverse water-gas shift reaction to provide a first product stream comprising CO and H₂, the first product stream having a lower concentration of CO₂ and a higher concentration of CO than the first feed stream;
   contacting at a second temperature and at a second pressure a Fischer-Tropsch catalyst with a second feed stream comprising H₂ and at least a portion of CO of the first product stream to provide a second product stream comprising C₅₊ hydrocarbons,
   wherein the reverse water-gas shift catalyst is a supported reverse water-gas shift catalyst comprising:
      a support that is a cerium oxide support, a titanium oxide support, an aluminum oxide support, a zinc oxide support, a zirconium oxide support, or a mixed oxide support comprising a mixture of two or more of cerium oxide, titanium oxide, aluminum oxide, zinc oxide, and zirconium oxide;
      a metal selected from at least one of manganese, copper, gallium, indium, lanthanum, titanium, niobium, vanadium, and zirconium, present in an amount in the range of 0.5 to 20 wt% of the catalyst, based on the total weight of the catalyst; and
      optionally, at least one of platinum, palladium, gold, and nickel present in an amount in the range of 0.05 to 10 wt% of the catalyst, based on the total weight of the catalyst.
Embodiment 211. The process of embodiment 210, wherein the reverse water-gas shift catalyst is as described in any embodiments 1 to 129.
Embodiment 212. The process of any embodiment 210, wherein the reverse water-gas shift catalyst is made by the method of any of embodiments 130 to 141.
Embodiment 213. The process of any of embodiments 210-212, wherein the CO₂ of the first feed stream comprises at least 50 vol% (e.g., at least 75 vol%, at least 90 vol%, or at least 95 vol%) CO₂ from biogas, a CO₂ emission source, and/or CO₂ from direct air capture.
Embodiment 214. The process of any of embodiments 210-212, wherein at least part of the CO₂ of the first feed stream is from biogas.
Embodiment 215. The process of embodiment 214, wherein the CO₂ of the first feed stream comprises at least 50 vol% (e.g., at least 75 vol%, at least 90 vol%, or at least 95 vol%) CO₂ from biogas.
Embodiment 216. The process of any of embodiments 210-212, wherein at least part of the CO₂ of the first feed stream is from direct air capture.
Embodiment 217. The process of embodiment 216, wherein the CO₂ of the first feed stream comprises at least 50 vol% (e.g., at least 75 vol%, at least 90 vol%, or at least 95 vol%) CO₂ from direct air capture.
Embodiment 218. The process of any of embodiments 210-212, wherein at least part of the CO₂ of the first feed stream is from a CO₂ emission source (e.g., from a manufacturing plant, e.g., a bioethanol plant, a steel plant, or a cement plant).
Embodiment 219. The process of embodiment 218, wherein the CO₂ of the first feed stream comprises at least 50 vol% (e.g., at least 75 vol%, at least 90 vol%, or at least 95 vol%) CO₂ from a CO₂ emission source.
Embodiment 220. The process of any of embodiments 210-219, wherein the molar ratio of H₂ to CO₂ in the first feed stream is at least 0.1:1, e.g., at least 0.5:1.
Embodiment 221. The process of any of embodiments 210-219, wherein the molar ratio of H₂ to CO₂ in the first feed stream is at least 0.9:1, e.g., at least 1:1 or at least 1.5:1.
Embodiment 222. The process of any of embodiments 210-219, wherein the molar ratio of H₂ to CO₂ in the first feed stream is at least 2:1, e.g., at least 2.5:1.
Embodiment 223. The process of any of embodiments 210-222, wherein the molar ratio of H₂ to CO₂ in the first feed stream is no more than 100:1, e.g., no more than 75:1, or 50:1.
Embodiment 224. The process of any of embodiments 210-222, wherein the molar ratio of H₂ to CO₂ in the first feed stream is no more than 20:1, e.g., no more than 15:1, or 10:1.
Embodiment 225. The process of any of embodiments 210-224, wherein the molar ratio of H₂ to CO₂ in the first feed stream is in the range of 0.5:1 to 10:1.
Embodiment 226. The process according to any of embodiments 210-225, wherein the first feed stream further comprises CO.
Embodiment 227. The process according to any of embodiments 210-226, wherein the first feed stream comprises no more than 20 mol% (e.g., no more than 10 mol%, or no more than 5 mol%, or no more than 3 mol%, or no more than 1 mol%) of CO.
Embodiment 228. The process according to any of embodiments 210-227,wherein the first feed stream further comprises one or more inert gases (e.g., nitrogen and/or methane).
Embodiment 229. The process according to embodiment 228, wherein the first feed stream comprise no more than 50 mol% (e.g., no more than 30 mol%, no more than 20 vml%, or no more than 10 mol%) of methane.
Embodiment 230. The process according to embodiment 228 or embodiment 229, wherein the first feed stream comprises no more than 10 mol% (e.g., no more than 6 mol%, or no more than 2 mol%) of nitrogen.
Embodiment 231. The method of any of embodiments 210-230, wherein the reverse water-gas shift reaction has a CO selectivity of at least 50%, e.g., of at least 60%.
Embodiment 232. The method of any of embodiments 210-231, wherein the reverse water-gas shift reaction has a CO selectivity of at least 70%, e.g., of at least 80%.
Embodiment 233. The method of any of embodiments210-231, wherein the reverse water-gas shift reaction has a CO selectivity of at least 85%, e.g., of at least 95%.
Embodiment 234. The method of any of embodiments 210-231, wherein the reverse water-gas shift reaction has a CO selectivity of at least 85%, e.g., of at least 96%.
Embodiment 235. The method of any of embodiments 210-231, wherein the reverse water-gas shift reaction has a CO selectivity of 50-99 wt%, e.g., 60-99%, or 70-99%, or 80-99%, or 90-99%, or 95-99%.
Embodiment 236. The method of any of embodiments 210-231, wherein the reverse water-gas shift reaction has a CO selectivity of 50-90%, e.g., 60-90%, or 70-90%, or 50-80%, or 60-80%, or 50-70%.
Embodiment 237. The method of any of embodiments 210-236, wherein the reverse water-gas shift reaction has a methane selectivity of no more than 40%, e.g., no more than 35%, or 30%, or 25%, or 20%.
Embodiment 238. The method of any of embodiments 210-236, wherein the reverse water-gas shift reaction has a methane selectivity of no more than 15%, e.g., no more than 12%, or 10%, or 8%.
Embodiment 239. The process of any of embodiments 210-236, wherein the reverse water-gas shift reaction has a methane selectivity of no more than 5%, e.g., no more than 4%.
Embodiment 240. The process of any of embodiments 210-236, wherein the reverse water-gas shift reaction has a methane selectivity of no more than 2%, e.g., no more than 1%.
Embodiment 241. The process of any of embodiments 210-236, wherein the reverse water-gas shift reaction has a methane selectivity of no more than 0.5%, e.g., no more than 0.2%.
Embodiment 242. The process of any of embodiments 210-241, wherein the reverse water-gas shift reaction has a CO₂ conversion of at least 5%, e.g., at least 10%, or 20%.
Embodiment 243. The process of any of embodiments 210-241, wherein the reverse water-gas shift reaction has a CO₂ conversion of at least 30%, e.g., at least 40%.
Embodiment 244. The process of any of embodiments 210-243, wherein the reverse water-gas shift reaction has a CO₂ conversion of no more than 90%, e.g., no more than 80%, or no more than 70%.
Embodiment 245. The process of any of embodiments 210-243, wherein the reverse water-gas shift reaction has a CO₂ conversion of no more than 65%, e.g., no more than 60%.
Embodiment 246. The process of any of embodiments 210-245, wherein the reverse water-gas shift reaction is conducted at a temperature in the range of 250-1050 °C, e.g., in the range of 250-1000 °C, or 250-950 °C.
Embodiment 247. The process of any of embodiments 210-245, wherein the reverse water-gas shift reaction is conducted at a temperature in the range of 250-900 °C, e.g., in the range of 250-850 °C , or 250-800 °C, or 250-750 °C, or 250-700 °C, or 250-650 °C, or 250-600 °C.
Embodiment 248. The process of any of embodiments 210-245, wherein the reverse water-gas shift reaction is conducted at a temperature in the range of 300-1100 °C, e.g., in the range of 300-1050 °C, or 300-1000 °C, or 300-950 °C.
Embodiment 249. The process of any of embodiments 210-245, wherein the reverse water-gas shift reaction is conducted at a temperature in the range of 300-900 °C, e.g., in the range of 300-850 °C, or 300-800 °C, or 300-750 °C, or 300-700 °C, or 300-650 °C, or 300-600 °C.
Embodiment 250. The process of any of embodiments 210-245, wherein the reverse water-gas shift reaction is conducted at a temperature in the range of 350-1100 °C, e.g., in the range of 350-1050 °C, or 350-1000 °C , or 350-950 °C.
Embodiment 251. The process of any of embodiments 210-245, wherein the reverse water-gas shift reaction is conducted at a temperature in the range of 350-900 °C, e.g., in the range of 350-850 °C, or 350-800 °C , or 350-750 °C, or 350-700 °C, or 350-650 °C, or 350-600 °C.
Embodiment 252. The process of any of embodiments 210-245, wherein the reverse water-gas shift reaction is conducted at a temperature in the range of 400-1100 °C, e.g., in the range of 400-1050 °C, or 400-1000 °C , or 400-950 °C.
Embodiment 253. The process of any of embodiments 210-245, wherein the reverse water-gas shift reaction is conducted at a temperature in the range of 400-900 °C, e.g., in the range of 400-850 °C, or 400-800 °C , or 400-750 °C, or 400-700 °C, or 400-650 °C, or 400-600 °C.
Embodiment 254. The process of any of embodiments 210-245, wherein the reverse water-gas shift reaction is conducted at a temperature in the range of 450-1100 °C, e.g., in the range of 450-1050 °C, or 450-1000 °C, or 450-950 °C.
Embodiment 255. The process of any of embodiments 210-245, wherein the reverse water-gas shift reaction is conducted at a temperature in the range of 450-900 °C, e.g., in the range of 450-850 °C, or 450-800 °C, or 450-750 °C, or 450-700 °C, or 450-650 °C, or 450-600 °C.
Embodiment 256. The process of any of embodiments 210-245, wherein the reverse water-gas shift reaction is conducted at a temperature in the range of 500-1100 °C, e.g., in the range of 500-1050 °C, or 500-1000 °C, or 500-950 °C.
Embodiment 257. The process of any of embodiments 210-245, wherein the reverse water-gas shift reaction is conducted at a temperature in the range of 500-900 °C, e.g., in the range of 500-850 °C, or 500-800 °C, or 500-750 °C , or 500-700 °C, or 500-650 °C, or 500-600 °C.
Embodiment 258. The process of any of embodiments 210-245, wherein the reverse water-gas shift reaction is conducted at a temperature in the range of 550-1100 °C, e.g., in the range of 550-1050 °C, or 550-1000 °C, or 550-950°C.
Embodiment 259. The process of any of embodiments 210-245, wherein the reverse water-gas shift reaction is conducted at a temperature in the range of 550-900 °C, e.g., in the range of 550-850 °C, or 550-800 °C, or 550-750°C, or 550-700 °C, or 550-650 °C, or 550-600 °C.
Embodiment 260. The process of any of embodiments 210-245, wherein the reverse water-gas shift reaction is conducted at a temperature in the range of 600-1100 °C, e.g., in the range of 600-1050 °C, or 600-1000 °C, or 600-950°C.
Embodiment 261. The process of any of embodiments 210-245, wherein the reverse water-gas shift reaction is conducted at a temperature in the range of 600-900 °C, e.g., in the range of 600-850 °C, or 600-800 °C, or 600-750°C, or 600-700 °C, or 600-650 °C.
Embodiment 262. The process of any of embodiments 210-245, wherein the reverse water-gas shift reaction is conducted at a temperature in the range of 650-1100 °C, e.g., in the range of 650-1050 °C, or 650-1000 °C, or 650-950°C.
Embodiment 263. The process of any of embodiments 210-245, wherein the reverse water-gas shift reaction is conducted at a temperature in the range of 650-900 °C, e.g., in the range of 650-850 °C, or 650-800 °C, or 650-750°C, or 650-700 °C.
Embodiment 264. The process of any of embodiments 210-245, wherein the reverse water-gas shift reaction is conducted at a temperature in the range of 700-1100 °C, e.g., in the range of 700-1050 °C, or 700-1000 °C, or 700-950°C.
Embodiment 265. The process of any of embodiments 210-245, wherein the reverse water-gas shift reaction is conducted at a temperature in the range of 700-900 °C, e.g., in the range of 700-850 °C, or 700-800 °C, or 700-750°C.
Embodiment 266. The process of any of embodiments 210-245, wherein the reverse water-gas shift reaction is conducted at a temperature in the range of 200-500 °C, e.g., 200-450 °C, or 200-400 °C, or 200-350 °C, or 250-500 °C, e.g., 250-450 °C, or 250-400 °C, or 250-350 °C.
Embodiment 267. The process of any of embodiments 210-266, wherein the reverse water-gas shift reaction is conducted at a pressure in the range of 1 to 100 barg (e.g., in the range of 1 to 70 barg, or 1 to 50 barg, or 1 to 40 barg, or 1 to 35 barg, or 5 to 80 barg, or 5 to 50 barg, or 5 to 40 barg, or 5 to 35 barg, or 10 to 70 barg, 10 to 50 barg, or 10 to 40 barg, or 10 to 35 barg, or 20 to 70 barg, 20 to 50 barg, or 20 to 40 barg, or 20 to 35 barg, or 25 to 70 barg, 25 to 50 barg, or 25 to 40 barg, or 25 to 35 barg).
Embodiment 268. The process of any of embodiments 210-267, wherein the reverse water-gas shift reaction is conducted at a GHSV in the range of 1,000 to 2,000,000 h⁻¹ (e.g., in the range of 1,000 to 1,200,000 h⁻¹, or 1,000 to 500,000 h⁻¹, or 1,000 to 100,000 h⁻¹, or 5,000 to 1,200,000 h⁻¹, or 5,000 to 500,000 h⁻¹, or 5,000 to 100,000 h⁻¹, or 10,000 to 1,200,000 h⁻¹, or 10,000 to 500,000 h⁻¹, or 10,000 to 100,000 h⁻¹).
Embodiment 269. The process of any of embodiments 210-268, wherein the process comprises activating the reverse water-gas shift catalyst, e.g., prior to contacting the reverse water-gas shift catalyst with the first feed stream.
Embodiment 270. The process of embodiment 269, wherein activating the rWGS catalyst comprises contacting the rWGS catalyst with a reducing stream comprising a reductive gas (e.g., hydrogen).
Embodiment 271. The process of embodiment 269 or embodiment 270, wherein the reducing stream comprises hydrogen in an amount of at least 25 mol% (e.g., at least 50 mol%, or 75 mol%, or 90 mol%).
Embodiment 272. The process of any of embodiments 269-271, wherein activating the rWGS catalyst is conducted at a temperature in the range of 200 °C to 1000 °C. (e.g., in the range of 250 °C to 1000 °C, or 300 °C to 1000 °C, 200 °C to 900 °C, 250 °C to 900 °C, or 300 °C to 900 °C, 200 °C to 800 °C, or 250 °C to 800 °C, or 300 °C to 800 °C, or 200 °C to 700 °C, or 250 °C to 700 °C, or 300 °C to 700 °C).
Embodiment 273. The process of any of embodiments 269-272, wherein activating the rWGS catalyst provides a catalyst that is at least 10% reduced (e.g., at least 25%, or 50%).
Embodiment 274. The process of any of embodiments 210-273, wherein the first product stream comprises no more than 95 mol% CO₂ (e.g., no more than 90 mol% CO₂).
Embodiment 275. The process of any of embodiments 210-273, wherein the first product stream comprises no more than 85 mol% CO₂ (e.g., no more than 80 mol% CO₂).
Embodiment 276. The process of any of embodiments 210-273, wherein the first product stream comprises no more than 75 mol% CO₂ (e.g., no more than 70 mol% CO₂).
Embodiment 277. The process of any of embodiments 210-276, wherein the first product stream comprises in the range of 5-95 mol% CO₂, e.g., 5-90 mol%, or 5-85 mol%, or 5-80 mol%, or 5-75 mol%, or 5-70 mol%, or 10-95 mol%, or 10-90 mol%, or 10-85 mol%, or 10-80 mol%, or 10-75 mol%, or 10-70 mol%, or 20-95 mol%, or 20-90 mol%, or 20-85 mol%, or 20-80 mol%, or 20-75 mol%, or 20-70 mol%, or 30-95 mol%, or 30-90 mol%, or 30-85 mol%, or 30-80 mol%, or 30-75 mol%, or 30-70 mol% CO₂.
Embodiment 278. The process of any of embodiments 210-277, wherein the first product stream comprises methane in an amount in the range of 10-70 mol% (e.g., in the range of 10-50 mol%, or 20-70 mol%, or 20-50 mol%, or 30-70 mol%, or 30-50 mol%).
Embodiment 279. The process of any of embodiments 210-277, wherein the first product stream comprises no more than 20 mol% methane, e.g., no more than 15 mol% methane.
Embodiment 280. The process of any of embodiments 210-277, wherein the first product stream comprises no more than 10 mol% methane, e.g., no more than 5 mol% or 1 mol%, or 0.5 mol%, or 0.1 mol% methane.
Embodiment 281. The process of any of embodiments 210-280, wherein a ratio of H₂:CO in the first product stream is up to 100:1, e.g., up to 50:1, or up to 25:1, or up to 10:1.
Embodiment 282. The process of any of embodiments 210-280, wherein a ratio of H₂:CO in the first product stream is in the range of 0.1:1 to 100:1 (e.g., in the range of 0.1:1 to 50:1, or 0.1:1 to 25:1, or 0.1:1 to 10:1, or 0.1:1 to 5:1, or 1:1 to 100:1, or 1:1 to 50:1, or 1:1 to 25:1, or 1:1 to 10:1, or 1:1 to 5:1).
Embodiment 283. The process of any of embodiments 210-282, wherein the process further comprises separating the first product stream to recycle at least a portion of one or more components of the first product stream to the first feed stream.
Embodiment 284. The process of any of embodiments 210-283, wherein the process further comprises separating the first product stream to recycle at least a portion (e.g., at least 5 mol%, at least 10 mol%, at least 25 mol%, at least 50 mol%, at least 75 mol%, or at least 90 mol%) of CO₂ of the first product stream to the first feed stream.
Embodiment 285. The process of any of embodiments 210-284, wherein the process further comprises separating the first product stream to recycle at least a portion of H₂ (e.g., at least 5 mol%, at leat10 mol%, at least 25 mol%, at least 50 mol%, at least 75 mol%, or at least 90 mol%) to the first feed stream.
Embodiment 286. The process of any of embodiments 210-285, wherein the process further comprises separating at least a portion of H₂ and/or CO from the first product stream and contacting it with the Fischer-Tropsch catalyst to activate the Fischer-Tropsch catalyst.
Embodiment 287. The process of any of embodiments 210-286, wherein the process further comprises removing at least a portion (e.g., at least 25%, at least 50%, or at least 75%) of water from the first product stream.
Embodiment 288. The process according to any of embodiments 210-287, wherein the first product stream further comprises one or more light hydrocarbons (e.g., methane, ethane, propane).
Embodiment 289. The process according to embodiment 288, further comprising separating at least a portion of the one or more light hydrocarbons from the first product stream to provide a light hydrocarbon stream.
Embodiment 290. The process according to embodiment 288 or 289, wherein the light hydrocarbon stream comprises methane from biogas.
Embodiment 291. The process according to embodiment 290, further comprising burning at least a portion of the light hydrocarbon stream to provide energy, e.g., heat energy or electrical energy.
Embodiment 292. The process according to embodiment 291, wherein the heat energy is used to heat the first feed stream.
Embodiment 293. The process of any of embodiments 210-292, wherein the process further comprises exchanging heat between at least a portion of the first product stream and at least a portion of the first feed stream, thereby cooling at least a portion of the first product stream and heating at least a portion of the first feed stream.
Embodiment 294. The process of any of embodiments 210-293, wherein the process further comprises exchanging heat between at least a portion of the first product stream and a steam generation zone, thereby cooling at least a portion of the first product stream and providing heat to the steam generation zone.
Embodiment 295. The process of embodiment 294, further comprising generating steam from the heat provided to the steam generation zone, and generating electricity from the steam.
Embodiment 296. The process of embodiment 294 or 295, wherein steam is used to heat the first feed stream and/or the second feed stream.
Embodiment 297. The process of any of embodiments 210-296, wherein at least 25% of the CO of the first product stream, e.g., at least 50% of the CO, at least 75% of the CO, or at least 90% of the CO of the first product stream is included in the second feed stream.
Embodiment 298. The process of any of embodiments 210-297, wherein CO is provided to the second feed stream from a CO source other than the first product stream.
Embodiment 299. The process of any of embodiments 210-298, wherein the first product stream includes H₂, and wherein the second feed stream includes at least a portion of the H₂ of the first product stream.
Embodiment 300. The process of any of embodiments 210-299, wherein at least 25% of the H₂ of the first product stream, e.g., at least 50% of the H₂, at least 75% of the H₂, or at least 90% of the H₂ of the first product stream is included in the second feed stream.
Embodiment 301. The process of any of embodiments 210-300, wherein H₂ is provided to the second feed stream from a hydrogen source other than the first product stream.
Embodiment 302. The process of any of embodiments 210-301, wherein the second feed stream includes at least a portion of CO₂ of the first product stream.
Embodiment 303. The process of any of embodiments 210-302, wherein at least 10% of the CO₂ of the first product stream, e.g., at least 25% of the CO₂, at least 50% of the CO₂, at least 75% of the CO₂, or at least 90% of the CO₂ of the first product stream is included in the second feed stream.
Embodiment 304. The process of any of embodiments 210-302, wherein the second feed stream does not include a substantial amount of CO₂ of the first product stream.
Embodiment 305. The process of any of embodiments 210-304, wherein the portion of the first product stream that is included in the second feed stream has a H₂:CO ratio in the range of 0.5:1 to 10:1, e.g., in the range of 1:1 to 3:1.
Embodiment 306. The process of any of embodiments 210-305, wherein the portion of the first product stream that is included in the second feed stream has a water content of no more than 10 mol%, e.g., or no more than 2 mol%, or no more than 0.5 mol%.
Embodiment 307. The process of any of embodiments 210-306, wherein the portion of the first product stream that is included in the second feed stream has a CO₂ content in the range of 10-95 mol% CO₂, e.g., 10-90 mol%, or 10-85 mol%, or 10-80 mol%, or 10-75 mol%, or 10-70 mol%, or 20-95 mol%, or 20-90 mol%, or 20-85 mol%, or 20-80 mol%, or 20-75 mol%, or 20-70 mol%, or 30-95 mol%, or 30-90 mol%, or 30-85 mol%, or 30-80 mol%, or 30-75 mol%, or 30-70 mol% CO₂.
Embodiment 308. The process of any of embodiments 210-307, wherein the second feed stream has a H₂:CO ratio in the range of 0.5:1 to 6:1.
Embodiment 309. The process of any of embodiments 210-307, wherein the second feed stream has a H₂:CO ratio in the range of 1:1 to 3:1, e.g., 1:1 to 2.5:1.
Embodiment 310. The process of any of embodiments 210-307, wherein the second feed stream has a H₂:CO ratio of at least 1.4:1, e.g., in the range of 1.4:1 to 3:1, or 1.4:1 to 2.5:1.
Embodiment 311. The process of any of embodiments 210-310, wherein the second feed stream includes up to 80% of one or more inerts, e.g., up to 70 mol%, up to 60 mol%, or up to 50 mol%, or 15-70 mol%, or 30-70 mol%, or 15-60 mol%, or 30-60 mol%, or 15-50 mol%, or 30-50 mol%.
Embodiment 312. The process of any of embodiments 210-310, wherein the second feed stream includes up to 80% of one or more inerts selected from CO₂, methane and nitrogen, e.g., up to 70 mol%, up to 60 mol%, or up to 50 mol%, or 15-70 mol%, or 30-70 mol%, or 15-60 mol%, or 30-60 mol%, or 15-50 mol%, or 30-50 mol%.
Embodiment 313. The process of any of embodiments 210-312, wherein the second feed stream includes up to 80% of CO₂, e.g., up to 70 mol%, up to 60 mol%, or up to 50 mol%, or 15-70 mol%, or 30-70 mol%, or 15-60 mol%, or 30-60 mol%, or 15-50 mol%, or 30-50 mol%.
Embodiment 314. The process of any of embodiments 210-313, wherein the second feed stream has a water content of no more than 10 mol%, e.g., or no more than 2 mol%, or no more than 0.5 mol%.
Embodiment 315. The process of any of embodiments 210-314, wherein the Fischer-Tropsch catalyst comprises cobalt, iron, rhodium, ruthenium, or a combination thereof.
Embodiment 316. The process of any of embodiments 210-314, wherein the Fischer-Tropsch catalyst comprises cobalt, for example, in an amount in the range of 5-25 wt%, e.g., 7-25 wt%, or 10-25 wt%, or 5-20 wt%, or 7-20 wt%, or 10-20 wt%, calculated as Co(0).
Embodiment 317. The process of any of embodiments 210-314, wherein the Fischer-Tropsch catalyst comprises iron, for example, in an amount in the range of 5-95 wt%, e.g., 10-95 wt%, or 25-95 wt%, or 50-95 wt%, or 5-85 wt%, or 10-85 wt%, or 25-85 wt%, or 50-85 wt%, or 5-75 wt%, or 10-75 wt%, or 25-75 wt%, calculated as Fe(0).
Embodiment 318. The process of any of embodiments 313-317, wherein the Fischer-Tropsch catalyst further comprises manganese.
Embodiment 319. The process of embodiment 318, wherein the manganese is present in an amount up to 15 wt%, e.g., up to 12 wt%, or up to 10 wt%, or up to 7 wt%, or in the range of 0.1-15 wt%, e.g., 0.1-10 wt%, or 0.1-5 wt%, 0.5-15 wt%, or 0.5-10 wt%, or 0.5-5 wt%, calculated as Mn(0).
Embodiment 320. The process of any of embodiments 210-319, wherein the Fischer-Tropsch catalyst is a supported catalyst, wherein the support comprises at least one of titanium oxide, zirconium oxide, cerium oxide, aluminum oxide, silicon oxide and zinc oxide.
Embodiment 321. The process of any of embodiments 210-319, wherein the Fischer-Tropsch catalyst is a supported catalyst, wherein the support comprises at least one of titanium oxide, aluminum oxide, and silicon oxide.
Embodiment 322. The process of any of embodiments 210-319, wherein the Fischer-Tropsch catalyst is a supported catalyst, wherein the support is a titanium dioxide support.
Embodiment 323. The process of any of embodiments 185210-322, wherein the Fischer-Tropsch catalyst is activated by contact with a reducing gas, e.g., hydrogen.
Embodiment 324. The process of embodiment 323, wherein the reducing gas comprises at least a portion of hydrogen from the first product stream.
Embodiment 325. The process of any of embodiments 210-324, wherein the Fischer-Tropsch catalyst is activated by contact with H₂ and CO.
Embodiment 326. The process of embodiment 325, wherein the reducing gas comprises at least a portion of H₂ and CO from the first product stream.
Embodiment 327. The process of any of embodiments 210-326, wherein the activation is performed at a temperature in the range of 200-400 °C
Embodiment 328. The process of any of embodiments 210-327, wherein the second temperature is in the range of 150-400 °C (e.g., in the range of 150-350 °C, or 150-300 °C, or 150-250°C, or 150-200°C, or 200-400 °C, or 200-350 °C, or 200-300°C, or 200-250 °C, or 250-400 °C, or 250-350 °C, or 250-300 °C, or 300-400 °C).
Embodiment 329. The process of any of embodiments 210-328, wherein the second temperature is in the range of 200-350 °C.
Embodiment 330. The process of any of embodiments 210-329, wherein the first temperature is within 100 °C of the second temperature, e.g., within 50 °C of the second temperature, or within 25 °C of the second temperature.
Embodiment 331. The process of any of embodiments 210-330, wherein the first temperature is at least 100 °C greater than the second temperature, e.g., at least 150 °C greater than the second temperature, or at least 200 °C greater than the second temperature.
Embodiment 332. The process of any of embodiments 210-331, wherein the second pressure is in the range of 10-50 barg (e.g., 20-50 barg, or 25-50 barg, or 10-40 barg, or 20-40 barg, or 25-40 barg or 10-35 barg, or 20-35 barg, or 25-35 barg).
Embodiment 333. The process of any of embodiments 210-332, wherein the second pressure is in the range of 20-50 barg.
Embodiment 334. The process of any of embodiments 210-333, wherein the Fischer-Tropsch reaction is conducted at a GHSV in the range of 1,000 to 2,000,000 h⁻¹ (e.g., in the range of 1,000 to 1,200,000 h⁻¹, or 1,000 to 500,000 h⁻¹, or 1,000 to 100,000 h⁻¹, or 5,000 to 1,200,000 h⁻¹, or 5,000 to 500,000 h⁻¹, or 5,000 to 100,000 h⁻¹, or 10,000 to 1,200,000 h⁻¹, or 10,000 to 500,000 h⁻¹, or 10,000 to 100,000 h⁻¹).
Embodiment 335. The process of any of embodiments 210-334, wherein the contacting of the Fischer-Tropsch catalyst with the second feed stream to provide the second product stream is performed with a C₅₊ selectivity of at least 30%, e.g., at least 50%, or at least 70%.
Embodiment 336. The process of any of embodiments 210-335, wherein the contacting of the Fischer-Tropsch catalyst with the second feed stream to provide the second product stream is performed with a selectivity for C₅₊ alkanes of at least 30%, e.g., at least 50%, or at least 70%.
Embodiment 337. The process of any of embodiments 210-336, wherein the contacting of the Fischer-Tropsch catalyst with the second feed stream to provide the second product stream is performed with a selectivity for C₅₊ alkanes and C₅₊ alcohols of at least 30%, e.g., at least 50%, or at least 70%.
Embodiment 338. The process of any of embodiments 210-337, further comprising separating at least a portion of water from the second product stream.
Embodiment 339. The process of any of embodiments 210-338, further comprising separating at least a portion of C₁-C₄ hydrocarbons from the second product stream to provide a light hydrocarbon stream.
Embodiment 340. The process of embodiment 339, further comprising including at least a portion of the light hydrocarbon stream in the first feed stream and/or the second feed stream.
Embodiment 341. The process of embodiment 339 or embodiment 340, further comprising oxidizing at least a portion of the light hydrocarbon stream to provide a CO- and/or CO₂-containing pOX stream, and including at least a portion of the pOX stream in the first feed stream and/or the second stream.
Embodiment 342. The process of any of embodiments 339-341, wherein the light hydrocarbon stream comprises methane from biogas.
Embodiment 343. The process of embodiment 342, comprising providing a biogas comprising CO₂ and methane, and providing at least a portion of the CO₂ to the first feed stream, and at least a portion of the methane to the oxidation of at least a portion of the light hydrocarbon stream.
Embodiment 344. The process of any of embodiments 339-343, further comprising reforming (e.g., steam reforming and/or autothermal reforming) at least a portion of the light hydrocarbon stream to provide a CO- and/or CO₂-containing reformed stream, and including at least a portion of the reformed stream in the first feed stream and/or the second feed stream.
Embodiment 345. The process of any of embodiments 341-344, wherein the oxidation or the reforming provides energy, heat energy or electrical energy.
Embodiment 346. The process of any of embodiments 339-345, further comprising burning at least a portion of the light hydrocarbon stream to provide energy, e.g., heat energy or electrical energy.
Embodiment 347. The process of embodiment 346, wherein heat energy is provided, and the heat energy is used to heat the first feed stream.
Embodiment 348. The process of any of embodiments 210-347, wherein the process further comprises exchanging heat between at least a portion of the second product stream and a steam generation zone, thereby cooling at least a portion of the first feed stream and providing heat to the steam generation zone.
Embodiment 349. The process of embodiment 348, further comprising generating steam from the heat provided to the steam generation zone, and generating electricity from the steam.
Embodiment 350. The process of embodiment 348 or 349, wherein steam is used to heat the first feed stream and/or the second feed stream.
Embodiment 351. The process of any of embodiments 210-350, wherein the process further comprises exchanging heat between at least a portion of the second product stream and at least a portion of the second feed stream, thereby cooling at least a portion of the second product stream and heating at least a portion of the second feed stream.
Embodiment 352. The process of any of embodiments 210-351, further comprising recycling at least a portion of H₂ of the second product stream to the second feed stream.
Embodiment 353. The process of any of embodiments 210-352, further comprising recycling at least a portion of H₂ of the second product stream to the first feed stream.
Embodiment 354. The process of embodiment 353, further comprising providing H₂ to the second feed stream from a H₂ source other than the first product stream.
Embodiment 355. The process of embodiment 354, when H₂ from the second product stream makes up most of the H₂ of the first feed stream, e.g., at least 90%, at least 95%, or at least 98% of the H₂ of the first feed stream.
Embodiment 356. The process of any of embodiments 210-355, further comprising recycling at least a portion of CO of the second product stream to the second feed stream.
Embodiment 357. The process of any of embodiments 210-356, further comprising recycling at least a portion of CO of the second product stream to the first feed stream.
Embodiment 358. The process of any of embodiments 210-357, further comprising recycling at least a portion of inerts of the second product stream to the second feed stream.
Embodiment 359. The process of any of embodiments 210-358, further comprising recycling at least a portion of inerts of the second product stream to the first feed stream.
Embodiment 360. The process of any of embodiments 210-359, further comprising recycling at least a portion of CO₂ of the second product stream to the first feed stream.
Embodiment 361. The process of embodiment 360, further comprising providing CO₂ to the second feed stream from a CO₂ source other than the first product stream.
Embodiment 362. The process of embodiment 361, when CO₂ from the second product stream makes up most of the CO₂ of the first feed stream, e.g., at least 90%, at least 95%, or at least 98% of the CO₂ of the first product stream.
Embodiment 363. The process of any of embodiments 210-362, wherein one or more products are provided from at least a portion of C5+ hydrocarbons of the second product stream.
Embodiment 364. The process of embodiment 363, wherein the one or more products include fuels (e.g., gasoline, diesel fuel, aviation fuel), lubricants and waxes.
Embodiment 365. The process of any of embodiments 210-364, further comprising hydroprocessing at least a portion of C5+ hydrocarbons of the second product stream. Embodiment 366. The process of any of embodiments 210-365, wherein at least part of the CO₂ of the second feed stream is from a renewable source.
Embodiment 367. The process of any of embodiments 210-365, wherein at least part of the CO₂ of the second feed stream is from biogas.
Embodiment 368. The process of any of embodiments 210-365, wherein at least part of the CO₂ of the second feed stream is from direct air capture.
Embodiment 369. The process of any of embodiments 210-365, wherein at least part of the CO₂ of the second feed stream is from a CO₂ emission source (e.g., from a manufacturing plant, e.g., a bioethanol plant, a steel plant, or a cement plant).
Embodiment 370. The process of any of embodiments 210-369, wherein at least part of the H₂ of the first feed stream or the second feed stream is from a renewable source.
Embodiment 371. The process of any of embodiment 210-370, wherein at least a portion of the hydrogen of the first feed stream or the second feed stream is green hydrogen.
Embodiment 372. The process of any of embodiment 210-371, wherein at least a portion of the hydrogen of the first feed stream or the second feed stream is blue hydrogen.
Embodiment 373. The process of any of embodiment 210-372, wherein at least a portion of the hydrogen of the first feed stream or the second feed stream is grey hydrogen, black hydrogen, brown hydrogen, pink hydrogen, turquoise hydrogen, yellow hydrogen, and/or white hydrogen.
Embodiment 374. The process of any of embodiments 210-373, further comprising providing at least a portion of H₂ to the first feed stream and/or the second feed stream by electrolysis of water.
Embodiment 375. The process of embodiment 374, wherein the electrolysis of water is performed using at least partially electricity from a renewable source.
Embodiment 376. The process of embodiment 374 or embodiment 375, wherein the electrolysis of water is performed using at least partially electricity generated from steam made by heat exchange from the first product stream and/or the second product stream, or by burning a light hydrocarbon stream.
Embodiment 377. The process of any of embodiments 372-376, further comprising providing at least a portion of O₂ generated in the electrolysis to a partial oxidation.
Embodiment 378. The process of any of embodiments 210-377, wherein the process is performed in a reactor system comprising a first reactor in which the reverse water-gas shift catalyst is disposed, and a second reactor in which the Fischer-Tropsch catalyst is disposed.
Embodiment 379. The process of any of embodiments 210-377, wherein the process is performed in a reactor system comprising a first catalyst bed in which the reverse water-gas shift catalyst is disposed and a second catalyst bed in which the Fischer-Tropsch catalyst is disposed.
Embodiment 380. The process of embodiment 379, wherein the first reactor bed and the second reactor bed are disposed within the same reactor.
Embodiment 381. The process of any of embodiments 210-380, wherein the process is performed in a reactor system comprising one or more first catalyst containers in which the reverse water-gas shift catalyst is disposed, and wherein the second reaction zone comprises one or more second catalyst containers in which the Fischer-Tropsch catalyst is disposed.
Embodiment 382. The process of embodiment 381, wherein the one or more first catalyst containers and the one or more second catalyst containers are disposed within the same reactor.
Embodiment 383. The process of any of embodiments 210-382, wherein the process is performed in a reactor system comprising a reactor in which the reverse water-gas shift catalyst and the Fischer-Tropsch catalyst are disposed, e.g., in admixture.

The particulars shown herein are by way of example and for purposes of illustrative discussion of the preferred embodiments of the present invention only and are presented in the cause of providing what is believed to be the most useful and readily understood description of the principles and conceptual aspects of various embodiments of the invention. In this regard, no attempt is made to show structural details of the invention in more detail than is necessary for the fundamental understanding of the invention, the description taken with the drawings and/or examples making apparent to those skilled in the art how the several forms of the invention may be embodied in practice. Thus, before the disclosed processes and devices are described, it is to be understood that the aspects described herein are not limited to specific embodiments, apparatuses, or configurations, and as such can, of course, vary. It is also to be understood that the terminology used herein is for the purpose of describing particular aspects only and, unless specifically defined herein, is not intended to be limiting.

The terms "a," "an," "the" and similar referents used in the context of describing the invention (especially in the context of the following claims) are to be construed to cover both the singular and the plural, unless otherwise indicated herein or clearly contradicted by context. Recitation of ranges of values herein is merely intended to serve as a shorthand process of referring individually to each separate value falling within the range. Unless otherwise indicated herein, each individual value is incorporated into the specification as if it were individually recited herein. It will be further understood that the endpoints of each of the ranges are significant both in relation to the other endpoint, and independently of the other endpoint.

All processes described herein can be performed in any suitable order of steps unless otherwise indicated herein or otherwise clearly contradicted by context. The use of any and all examples, or exemplary language (e.g., "such as") provided herein is intended merely to better illuminate the invention and does not pose a limitation on the scope of the invention otherwise claimed. No language in the specification should be construed as indicating any non-claimed element essential to the practice of the invention.

Unless the context clearly requires otherwise, throughout the description and the claims, the words 'comprise', 'comprising', and the like are to be construed in an inclusive sense as opposed to an exclusive or exhaustive sense; that is to say, in the sense of "including, but not limited to". Words using the singular or plural number also include the plural and singular number, respectively. Additionally, the words "herein," "above," and "below" and words of similar import, when used in this application, shall refer to this application as a whole and not to any particular portions of the application.

As will be understood by one of ordinary skill in the art, each embodiment disclosed herein can comprise, consist essentially of or consist of its particular stated element, step, ingredient or component. As used herein, the transition term "comprise" or "comprises" means includes, but is not limited to, and allows for the inclusion of unspecified elements, steps, ingredients, or components, even in major amounts. The transitional phrase "consisting of" excludes any element, step, ingredient or component not specified. The transition phrase "consisting essentially of" limits the scope of the embodiment to the specified elements, steps, ingredients or components and to those that do not materially affect the embodiment.

Unless indicated to the contrary, the numerical parameters set forth in the specification and attached claims are approximations that may vary depending upon the desired properties sought to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contains certain errors necessarily resulting from the standard deviation found in their respective testing measurements.

Groupings of alternative elements or embodiments of the invention disclosed herein are not to be construed as limitations. Each group member may be referred to and claimed individually or in any combination with other members of the group or other elements found herein. It is anticipated that one or more members of a group may be included in, or deleted from, a group for reasons of convenience and/or patentability. When any such inclusion or deletion occurs, the specification is deemed to contain the group as modified thus fulfilling the written description of all Markush groups used in the appended claims.

Some embodiments of this invention are described herein, including the best mode known to the inventors for carrying out the invention. Of course, variations on these described embodiments will become apparent to those of ordinary skill in the art upon reading the foregoing description. The inventor expects skilled artisans to employ such variations as appropriate, and the inventors intend for the invention to be practiced otherwise than specifically described herein. Accordingly, this invention includes all modifications and equivalents of the subject matter recited in the claims appended hereto as permitted by applicable law. Moreover, any combination of the above-described elements in all possible variations thereof is encompassed by the invention unless otherwise indicated herein or otherwise clearly contradicted by context.

Furthermore, it is to be understood that the embodiments of the invention disclosed herein are illustrative of the principles of the present invention. Other modifications that may be employed are within the scope of the invention. Thus, by way of example, but not of limitation, alternative configurations of the present invention may be utilized in accordance with the teachings herein. Accordingly, the present invention is not limited to that precisely as shown and described.

## Claims

1. A process for performing an integrated Fischer-Tropsch process, the process comprising:
providing a first feed stream comprising H₂ and CO₂, wherein at least part of the CO₂ of the first feed stream is from biogas, a CO₂ emission source, and/or air capture;
contacting at a first temperature in the range of 200-1100 °C and at a first pressure a reverse water-gas shift catalyst with the first feed stream to perform a reverse water-gas shift reaction to provide a first product stream comprising CO and H₂, the first product stream having a lower concentration of CO₂ and a higher concentration of CO than the first feed stream;
contacting at a second temperature and at a second pressure a Fischer-Tropsch catalyst with a second feed stream comprising H₂ and at least a portion of CO of the first product stream to provide a second product stream comprising C₅₊ hydrocarbons,
wherein the reverse water-gas shift catalyst is a supported reverse water-gas shift catalyst comprising:
a support that is a cerium oxide support, a titanium oxide support, an aluminum oxide support, a zinc oxide support, a zirconium oxide support, or a mixed oxide support comprising a mixture of two or more of cerium oxide, titanium oxide, aluminum oxide, zinc oxide, and zirconium oxide;
a metal selected from at least one of manganese, gallium, indium, lanthanum, titanium, niobium, vanadium, copper and zirconium, present in an amount in the range of 0.5 to 20 wt% of the catalyst, based on the total weight of the catalyst; and
optionally, at least one of platinum, palladium, gold, and nickel present in an amount in the range of 0.05 to 10 wt% of the catalyst, based on the total weight of the catalyst

2. The process of claim 1, wherein the CO₂ of the first feed stream comprises at least 50 vol% (e.g., at least 75 vol%, at least 90 vol%, or at least 95 vol%) CO₂ from biogas.

3. The process of claim 1, wherein the CO₂ of the first feed stream comprises at least 50 vol% (e.g., at least 75 vol%, at least 90 vol%, or at least 95 vol%) CO₂ from direct air capture.

4. The process of claim 1, wherein the CO₂ of the first feed stream comprises at least 50 vol% (e.g., at least 75 vol%, at least 90 vol%, or at least 95 vol%) CO₂ from a CO₂ emission source.

5. The process of any of claims 1-4, wherein the reverse water-gas shift reaction has a CO selectivity of at least 95%, a methane selectivity of no more than 2%, and/oror a CO₂ conversion of at least 30%.

6. The process of any of claims 1-5, wherein the reverse water-gas shift reaction is conducted at a temperature in the range of 400-1100 °C, preferably between 500 °C and 1000 °C, most preferably between 500 °C and 900 °C.

7. The process of any of claims 1-6, wherein the process further comprises separating the first product stream to recycle at least a portion of CO₂ of H₂ of the first product stream to the first feed stream.

8. The process of any of claims 1-7, wherein at least 25% of the CO of the first product stream is included in the second feed stream, wherein the first product stream includes H₂, and wherein at least 25% of the H₂ of the first product stream is included in the second feed stream.

9. The process of any of claims 1-8, wherein the second temperature is in the range of 200-350 °C, and wherein the first temperature is at least 100 °C greater than the second temperature.

10. The process of any of claims 1-9, wherein the contacting of the Fischer-Tropsch catalyst with the second feed stream to provide the second product stream is performed with a selectivity for C₅₊ alkanes of at least 30%.

11. The process of any of claims 1-10, further comprising recycling at least a portion of H₂ and/or at least a portion of CO of the second product stream to the second feed stream or to the first feed stream.

12. The process of any of claims 1-11, further comprising recycling at least a portion of CO₂ of the second product stream to the first feed stream.

13. The process of any of claims 1-12, wherein the process is performed in a reactor system comprising a first reactor in which the reverse water-gas shift catalyst is disposed, and a second reactor in which the Fischer-Tropsch catalyst is disposed.

14. The process of any of claims 1-13, wherein the process is performed in a reactor system comprising first catalyst bed in which the reverse water-gas shift catalyst is disposed, and a second catalyst bed in which the Fischer-Tropsch catalyst is dispose, wherein the first reactor bed and the second reactor bed are disposed within the same reactor.

15. The process of any of claims 1-13, wherein the process is performed in a reactor system comprising a reactor in which the reverse water-gas shift catalyst and the Fischer-Tropsch catalyst are disposed in admixture or wherein the process is performed in a reactor system comprising a reactor in which a bifunctional catalyst with both reverse water-gas shift activity and Fischer-Tropsch activity is disposed.
